



US007455960B2

(12) **United States Patent**  
**Funakubo**

(10) **Patent No.:** **US 7,455,960 B2**  
(45) **Date of Patent:** **Nov. 25, 2008**

(54) **PHOTOTHERMOGRAPHIC MATERIAL**

(75) Inventor: **Takeshi Funakubo**, Kanagawa (JP)

(73) Assignee: **FUJIFILM Corporation**, Tokyo (JP)

(\*) Notice: Subject to any disclaimer, the term of this patent is extended or adjusted under 35 U.S.C. 154(b) by 79 days.

(21) Appl. No.: **11/543,023**

(22) Filed: **Oct. 5, 2006**

(65) **Prior Publication Data**

US 2007/0026349 A1 Feb. 1, 2007

**Related U.S. Application Data**

(62) Division of application No. 11/150,429, filed on Jun. 13, 2005, now Pat. No. 7,144,692.

(30) **Foreign Application Priority Data**

Jun. 14, 2004 (JP) 2004-175502

(51) **Int. Cl.**

**G03C 1/00** (2006.01)

(52) **U.S. Cl.** 430/617; 430/618; 430/619;  
430/620

(58) **Field of Classification Search** ..... 430/617-620  
See application file for complete search history.

(56) **References Cited**

**U.S. PATENT DOCUMENTS**

2005/0260529 A1 11/2005 Oyamada et al.  
2005/0277072 A1 12/2005 Ohzeki  
2007/0020566 A1\* 1/2007 Ohzeki ..... 430/619

\* cited by examiner

*Primary Examiner*—Geraldina Visconti

(74) *Attorney, Agent, or Firm*—Margaret A. Burke; Sheldon J. Moss

(57) **ABSTRACT**

The invention provides a photothermographic material having, on both sides of a support, an image forming layer including at least a photosensitive silver halide, a non-photosensitive organic silver salt, a reducing agent, and a binder, which is to be exposed with X-rays using a fluorescent intensifying screen, wherein (1) a coating amount of the photosensitive silver halide per one side is from 0.01 g/m<sup>2</sup> to 0.45 g/m<sup>2</sup> in terms of silver amount; and (2) a crossover (%) is 30% or more, or when parallel light having the same wavelength as a main emission peak wavelength of the fluorescent intensifying screen is incident perpendicular to the surface of the photothermographic material, the parallel light component of transmitted light comprises 5% or more of the incident light. A photothermographic material for medical use having high sensitivity and high image quality is provided.

**8 Claims, 6 Drawing Sheets**

FIG. 1



FIG. 2



FIG. 3



FIG. 4



FIG. 5



FIG. 6



FIG. 7



FIG. 8



FIG. 9



## PHOTOTHERMOGRAPHIC MATERIAL

CROSS-REFERENCE TO RELATED  
APPLICATION

This is a divisional application of, and claims priority to, Application Ser. No. 11/150,429, filed on Jun. 13, 2005 now U.S. Pat. No. 7,144,692. This application claims priority under 35 USC 119 from Japanese Patent Application No. 2004-175502, the disclosure of which is incorporated by reference herein.

## BACKGROUND OF THE INVENTION

## 1. Field of the Invention

The present invention relates to a photothermographic material. More particularly, the invention relates to a photothermographic material for medical use having high sensitivity and high image quality.

## 2. Description of the Related Art

In recent years, in the medical field and the graphic arts field, there has been a strong desire for providing a dry photographic process from the viewpoints of protecting the environment and economy of space. Further, the development of digitization in these fields has resulted in the rapid development of systems in which image information is captured and stored in a computer, and then when necessary processed and output by transmitting it to a desired location. Here the image information is output onto a photosensitive material using a laser image setter or a laser imager, and developed to form an image at the location. It is necessary for the photosensitive material to be able to record an image with high-intensity laser exposure and that a clear black-tone image with a high resolution and sharpness can be formed. While various kinds of hard copy systems using pigments or dyes, such as ink-jet printers or electrophotographic systems, have been distributed as general image forming systems using such digital imaging recording materials, images on the digital imaging recording materials obtained by such general image forming systems are insufficient in terms of the image quality (sharpness, granularity, gradation, and tone) needed for medical images used in making diagnoses, and high recording speeds (sensitivity). These kinds of digital imaging recording materials have not reached a level at which they can replace medical silver halide film processed with conventional wet development.

Photothermographic materials utilizing organic silver salts are already known. Photothermographic materials have an image forming layer in which a reducible silver salt (for example, an organic silver salt), a photosensitive silver halide, and if necessary, a toner for controlling the color tone of developed silver images are dispersed in a binder.

Photothermographic materials form a black silver image by being heated to a high temperature (for example, 80° C. or higher) after imagewise exposure to cause an oxidation-reduction reaction between a silver halide or a reducible silver salt (functioning as an oxidizing agent) and a reducing agent. The oxidation-reduction reaction is accelerated by the catalytic action of a latent image on the silver halide generated by exposure. As a result, a black silver image is formed on the exposed region. Photothermographic materials are described in "Thermally Processed Silver Systems", appearing in "Imaging Processes and Materials", Neblette, 8th edition, edited by Sturge, V. Warlsworth, and A. Shepp, chapter 8, pages 279 to 291, 1989, and the Fuji Medical Dry Imager FM-DPL is an example of a medical image forming system that has been made commercially available.

Since this kind of image forming system utilizing an organic silver salt has no fixing step, undeveloped silver halide remains inside the film after thermal development. Thus, there have intrinsically been two serious problems in the system.

One of them involves image instability after a thermal developing process, particularly fogging due to print-out when the material is exposed to light. As a means to improve print-out, a method of using silver iodide is known. Silver iodide has the characteristic of causing less print-out than silver bromide or silver iodobromide having an iodide content of 5 mol % or less, and has a potential for fundamentally solving the problem. However, the sensitivity of silver iodide grains known until now is extremely low, and the silver iodide grains do not achieve a level of sensitivity that is applicable for an actual system. When means of preventing recombination between photoelectrons and holes is performed to improve the sensitivity, it is an inherent problem that the characteristic of being excellent in the print-out property will be lost.

As means of increasing the sensitivity of a silver iodide photographic emulsion, the literature discloses addition of a halogen acceptor such as sodium nitrite, pyrogallol, hydroquinone or the like, immersion in an aqueous silver nitrate solution, sulfur sensitization at a pAg of 7.5, and the like. However, the sensitization effect of these halogen acceptors is very small and extremely insufficient for use in photothermographic materials.

Another problem is that light scattering due to the remaining silver halide grains may cause cloudiness whereby the film turns translucent or opaque and image quality is degraded. To solve this problem, means in which the grain size of photosensitive silver halide grains is made fine (to within a range of practical use of from 0.08 μm to 0.15 μm) and the addition amount is reduced as much as possible to suppress the cloudiness caused by the silver halide have been practically employed. However, the compromise results in decreasing the sensitivity further, the problem of cloudiness is not completely solved, and a dark milky color continues to remain and generate haze in the film.

In the case of a conventional wet developing process, the remaining silver halide is removed by processing with a fixing solution containing a silver halide solvent after the developing process. For the silver halide solvent, many kinds of inorganic and organic compounds are known which can form complexes with silver ions.

Even in the case of a dry thermal developing process, many attempts to introduce similar fixing measures in the material have been made. For example, a method has been proposed where a compound capable of forming complexes with silver ions is incorporated in the film and the silver halide is solubilized (usually referred to as fixing) through thermal development. However, this proposal only applies to silver bromide and silver chlorobromide, and the process also requires an additional heat treatment step for fixing, and the heating conditions require a high temperature within a range of from 155° C. to 160° C. Thus, the system is one in which fixing is difficult to achieve. In another proposal, a separate sheet (referred to as a fixing sheet) that includes a compound able to form complexes with silver ions is prepared, and after thermally developing the photothermographic material to form an image, the fixing sheet is overlaid on the developed photothermographic material, heating is carried out, and the remaining silver halide is dissolved and removed. However, since this proposal requires two sheets, from a practical viewpoint the obstacles are that the processing step is complicated and the operational stability of the process is hard to maintain,

and that there is a necessity to discard the fixing sheets after processing, resulting in generation of waste.

As another fixing method usable in thermal development, a method is proposed where a fixing agent for the silver halide is encapsulated in microcapsules, and thermal development releases the fixing agent and causes it to act. However, it is difficult to achieve a design that effectively releases the fixing agent. A method for fixing using a fixing solution after thermal development is also proposed, but it requires a wet process and therefore is not adequate for a completely dry process.

As described above, known methods for improving the turbidity of film have negative effects, and there have been substantial difficulties in their practical application.

On the other hand, attempts have also been made at applying the above-mentioned photothermographic material as photosensitive material for X-ray photographing. Conventionally, direct or indirect radiography films, mammography films and the like are generally known in the field of wet developing photosensitive materials for medical use. A featured aspect of X-ray image recording is to device some means to enhance the utilization efficiency of X-ray radiation in order to reduce the patient's X-ray exposure dose. One example is the use of the radiation that has passed through a support and reached a backside of the support, in addition to the use of the X-ray radiation on an incident side, by means of placing a photosensitive material, in which silver halide grains are coated on both sides of the support, between a pair of fluorescent intensifying screens, and performing exposure by X-ray radiation. However, the double-sided type photosensitive material suffers from a serious technical problem. The problem is that the backside photosensitive layer is exposed by the light that has been emitted to the front surface, passed through the support, and reached the backside photosensitive layer. The light, referred to as crossover, is diffused during passage through the support because of light scattering by silver halide grains in the front side, and produces a blurred image. Therefore crossover is not preferred because the crossover brings about a lowering of the image quality. In the case of conventional wet developing photosensitive materials, various attempts for reducing the crossover have been proposed, such as a crossover cutting layer disposed on both sides of the support between the silver halide emulsion layer and the support. The crossover cutting layer absorbs the transmitted light therein to prevent the light from reaching the backside of the support.

However, in the case of a photothermographic material, disposition of a crossover cutting layer on both sides of the support may result in disadvantages such as increasing residual colors in the obtained image to give unfavorable image tone for image observation and increasing haze or the like to unfavorably influence image quality.

An X-ray photothermographic material coated on both sides and using a blue fluorescent intensifying screen is described in Japanese Patent Application Laid-Open (JP-A) No. 59-142539, and a photosensitive material for medical use in which tabular grains that have a high content of silver chloride and have (100) major faces are coated on both sides of a support is described in JP-A No. 10-282606. However, these disclosed examples show a lack of recognition of the above-mentioned problems and give no description of means for solving these problems.

#### SUMMARY OF THE INVENTION

A first aspect of the invention is to provide a photothermographic material comprising, on both sides of a support, an

image forming layer comprising at least a photosensitive silver halide, a non-photosensitive organic silver salt, a reducing agent, and a binder, which is to be exposed with X-rays using a fluorescent intensifying screen, wherein

5 (1) a coating amount of the photosensitive silver halide per one side is from 0.01 g/m<sup>2</sup> to 0.45 g/m<sup>2</sup> in terms of silver amount, and

(2) a crossover (%) is 30% or more.

A second aspect of the invention is to provide a photothermographic material comprising, on both sides of a support, an image forming layer comprising at least a photosensitive silver halide, a non-photosensitive organic silver salt, a reducing agent, and a binder, which is to be exposed with X-rays using a fluorescent intensifying screen, wherein

10 (1) a coating amount of the photosensitive silver halide per one side is from 0.01 g/m<sup>2</sup> to 0.45 g/m<sup>2</sup> in terms of silver amount, and

15 (2) when parallel light having the same wavelength as a main emission peak wavelength of the fluorescent intensifying screen is incident perpendicular to the surface of the photothermographic material, the parallel light component of transmitted light comprises 5% or more of the incident light.

#### BRIEF DESCRIPTION OF THE DRAWINGS

25 FIG. 1 is a structural diagram illustrating a first embodiment of a thermal developing apparatus according to the present invention.

30 FIG. 2 is a sectional view showing a photothermographic material.

35 FIG. 3 is an explanatory diagram indicating a correlation between temperatures of the front and back surfaces of a photothermographic material respectively heated by first and second heating means and time.

40 FIG. 4 is a block diagram showing a control means.

45 FIG. 5 is a structural view showing an essential part of a thermal developing apparatus having a drum and pressing rollers.

50 FIG. 6 is a structural view showing an essential part of a thermal developing apparatus having a carrier, an endless belt, and pressing rollers.

55 FIG. 7 is a structural view showing an essential part of a thermal developing apparatus having plural pairs of first and second heating means.

45 FIG. 8 shows an emission spectrum of a fluorescent intensifying screen A.

50 FIG. 9 is a conceptual view of a heating means which comprises 6 sets of plate heaters.

#### DETAILED DESCRIPTION OF THE INVENTION

The present invention provides a high image quality photothermographic material which has high sensitivity and favorable gradation.

55 The present invention will be described in detail below.

##### 1. Photothermographic Material

The photothermographic material of the present invention is a double-sided type photothermographic material which has an image forming layer on both sides of a support, and is subjected to X-ray exposure using a fluorescent intensifying screen.

In the present invention, photographic properties are expressed by a photographic characteristic curve. A photographic characteristic curve is a D-log E curve representing a relationship between the common logarithm (log E) of a light exposure value, i.e., the exposure energy, and the optical

## 5

density (D), i.e., a scattered light photographic density, by plotting the former on the abscissa axis and the latter on the ordinate axis. From this characteristic curve, photographic properties such as sensitivity, fog, and gradation can be determined.

The photographic characteristic curve according to the invention is a characteristic curve which is obtained by exposing the photothermographic material with monochromatic light having the same wavelength as the main emission peak wavelength of the fluorescent intensifying screen and having a half width of  $15 \text{ nm} \pm 5 \text{ nm}$ .

In the present invention, sensitivity is expressed as an exposure value necessary for obtaining an image density of fog+0.5 after thermal development. The image whose sensitivity is to be measured is an image formed on an exposed side of the support. In the case of a double-sided type photothermographic material according to the invention, measurement is performed after removing the image forming layer that is disposed on the opposite side from an exposure face.

Sensitivity of the photothermographic material according to the invention is preferably from  $1 \times 10^{-6} \text{ watt} \cdot \text{sec} \cdot \text{m}^{-2}$  to  $1 \times 10^{-3} \text{ watt} \cdot \text{sec} \cdot \text{m}^{-2}$ , more preferably from  $2 \times 10^{-6} \text{ watt} \cdot \text{sec} \cdot \text{m}^{-2}$  to  $1 \times 10^{-3} \text{ watt} \cdot \text{sec} \cdot \text{m}^{-2}$ , and even more preferably from  $5 \times 10^{-6} \text{ watt} \cdot \text{sec} \cdot \text{m}^{-2}$  to  $1 \times 10^{-4} \text{ watt} \cdot \text{sec} \cdot \text{m}^{-2}$ .

Gradation in the present invention is expressed as a gradient of a line joining the points at fog+(optical density of 0.50) and fog+(optical density of 1.5) on a photographic characteristic curve (i.e., the value equals tan when the angle between the line and the abscissa axis is). In the present invention, an average gradient is preferably from 1.8 to 5.0, and more preferably from 2.0 to 4.3.

In the photothermographic material of the present invention, it is preferable that haze after thermal development is decreased to less than 80% of that before thermal development. More preferably, haze after thermal development is decreased to less than 75% of that before thermal development, and even more preferably, to less than 73%.

The photothermographic material of the present invention has an image forming layer, on both sides of a support, comprising at least a photosensitive silver halide, a non-photosensitive organic silver salt, a reducing agent, and a binder. The photothermographic material of the present invention may contain a nucleator.

It is a feature of the photothermographic material of the present invention that a crossover (%) is 30% or more, more preferably 35% or more, and even more preferably 40% or more. Crossover is an inherent property in a double-sided type photosensitive material, and means a proportion of light used to imagewise expose a photosensitive layer on one surface that passes through the support, and imagewise exposes a photosensitive layer on the other surface.

The crossover is determined in present invention as a value measured by the following processes.

A sample is inserted between a black paper and a fluorescent intensifying screen, and subjected to X-ray exposure from the black paper side. The sample is subjected to X-ray exposure while changing the X-ray radiation value by a distance method.

After the exposure, the sample is subjected to thermal development. Thereafter, the developed sample is divided into two parts, and then each image forming layer is peeled off. The optical density of the image forming layer of the side which is contacted with the fluorescent intensifying screen and that of the opposite side are measured separately to obtain the photographic characteristic curves of each image forming layer. An average sensitivity difference ( $\Delta \log E$ ) of these images is determined at the straight portion of the curve (from

## 6

a density of 0.5 to a density of 1.0). Crossover is calculated from the average value according to the following formula.

$$\text{Crossover (\%)} = 100 / (\text{Antilog}(\Delta \log E) + 1)$$

It is another feature of the photothermographic material of the present invention that a coating amount of photosensitive silver halide grains per one side is in a range of from  $0.01 \text{ g/m}^2$  to  $0.45 \text{ g/m}^2$  in terms of silver amount, and when parallel light, which has the same wavelength as the main emission peak wavelength of the fluorescent intensifying screen mentioned above, is incident perpendicular to the surface of the photothermographic material, the parallel light component of transmitted light comprises 5% or more of the incident light.

For the measurement of the parallel light component in a double-sided type photothermographic material, the image forming layer on the opposite side of the support from the incident side is removed with the aid of solvent for dissolving the layer, and then measurement is carried out by an optical measuring device (for example, a commercially available photospectrometer). When parallel light perpendicular to the surface of the photothermographic material is incident to the image forming layer surface, one part of the light is reflected totally from the surface of the material and the interface on the support, and another part is absorbed by the silver halide grains and the other layer constituents. The resulting parallel light component and the component scattered by silver halide grains may transmit through the support and reach to the back surface of the support. A small scattered light component is preferred because the light component scattered by silver halide grains may give a blurred image, and therefore a large perpendicular light component is preferred. In the present invention, the transmitted perpendicular light component is preferably 5% or more with respect to the incident light, more preferably 6.5% or more, and even more preferably 8% or more. The scattered light component is preferably less than 5%, more preferably 1% or less, and even more preferably 0.2% or less. Herein, the term "scattered light component" means light scattered at an angle of  $\pm 20^\circ$  or more when an incident angle of the parallel light is  $0^\circ$ .

In the case of a conventional wet developing silver halide photosensitive material well known in the art, the parallel light component comprises 5% or less of the transmitted light, and most of the transmitted light is the scattered light component. Accordingly, reducing the transmitted light is required to attain high image quality. However, in the present invention, there is no need for reducing the transmitted light because the parallel light component can be made the main component, and moreover, enhancing sensitivity becomes possible by increasing the transmitted light. Until now, it was impossible to attain high image quality with high sensitivity by positively utilizing the transmitted light. Hereinafter, the constitutions and components of the layers which make it possible to realize the above improvement are described in detail.

#### (Photosensitive Silver Halide)

Grains in the photosensitive silver halide of the present invention are tabular grains having a mean aspect ratio of from 2 to 100 and a mean equivalent spherical diameter of from  $0.3 \mu\text{m}$  to  $10 \mu\text{m}$ .

The photosensitive silver halide preferably has an average silver iodide content of 40 mol % or higher, more preferably 80 mol % or higher, and even more preferably 90 mol % or higher.

#### 1) Halogen Composition

For the photosensitive silver halide used in the invention, there is no particular restriction on the halogen composition and silver chloride, silver chlorobromide, silver bromide,

silver iodobromide, silver iodochlorobromide, and silver iodide can be used. Among these, silver iodobromide and silver iodide are preferable.

The photosensitive silver halide of the invention preferably has an average silver iodide content of 40 mol % or higher, more preferably 80 mol % or higher, and most preferably 90 mol % or higher.

Other components are not particularly limited and can be selected from silver halides such as silver chloride, silver bromide, or the like and organic silver salts such as silver thiocyanate, silver phosphate, or the like.

The distribution of the halogen composition in a grain may be uniform or the halogen composition may be changed step-wise, or it may be changed continuously. Further, a silver halide grain having a core/shell structure can be preferably used. Preferred structure is a twofold to fivefold structure and, more preferably, core/shell grain having a twofold to fourfold structure can be used. A core-high-silver iodide-structure which has a high content of silver iodide in the core part, and a shell-high-silver iodide-structure which has a high content of silver iodide in the shell part can also be preferably used. Further, a technique of localizing silver bromide or silver iodide on the surface of a grain as form epitaxial parts can also be preferably used.

The silver halide having high silver iodide content of the invention can assume any content of  $\beta$  phase or  $\gamma$  phase. The term " $\beta$  phase" described above means a high silver iodide structure having a wurtzite structure of a hexagonal system and the term " $\gamma$  phase" means a high silver iodide structure having a zinc blende structure of a cubic crystal system. A content of  $\gamma$  phase in the present invention is determined by a method presented by C. R. Berry. In the method, a content of  $\gamma$  phase is calculated from the peak ratio of the intensity owing to  $\gamma$  phase (111) to that owing to  $\beta$  phases (100), (101), and (002) in powder X ray diffraction method. Detail description, for example, is described in Physical Review, volume 161, No. 3, p. 848 to 851 (1967).

### 2) Grain Size

Concerning the photosensitive silver halide grains used in the present invention, any grain size enough to reach the required high sensitivity can be selected. In the present invention, a mean equivalent spherical diameter of the tabular silver halide is from 0.2  $\mu\text{m}$  to 10.0  $\mu\text{m}$ , preferably from 0.25  $\mu\text{m}$  to 6.0  $\mu\text{m}$ , and more preferably from 0.30  $\mu\text{m}$  to 5.0  $\mu\text{m}$ . The term "equivalent spherical diameter" used here means a diameter of a sphere having the same volume as the volume of one silver halide grain. As for measuring method, the volume of a grain is calculated from projected area and thickness of individual grains by observation through electron microscope, and thereafter the equivalent spherical diameter is determined by converting the volume to a sphere having the volume equivalent to the obtained volume.

### 3) Coating Amount

In the present invention, a coating amount of silver halide is preferably in a range of from 0.01 g/ $\text{m}^2$  to 0.45 g/ $\text{m}^2$  per one side, more preferably from 0.02 g/ $\text{m}^2$  to 0.4 g/ $\text{m}^2$  per one side, and even more preferably from 0.05 g/ $\text{m}^2$  to 0.25 g/ $\text{m}^2$  per one side.

With respect to 1 mol of silver contained in the non-photosensitive organic silver salt described below, the coating amount of silver halide is preferably from 1.5 mol % to 70 mol %, more preferably from 3 mol % to 65 mol %, and even more preferably from 7 mol % to 40 mol %.

### 4) Method of Grain Formation

The method of forming photosensitive silver halide is well-known in the relevant art and, for example, methods described in Research Disclosure No. 17029, June 1978 and U.S. Pat.

No. 3,700,458 can be used. Specifically, a method of preparing a photosensitive silver halide by adding a silver-supplying compound and a halogen-supplying compound in a gelatin or other polymer solution and then mixing them with an organic silver salt is used.

Further, a method described in JP-A No. 11-119374 (paragraph Nos. 0217 to 0224) and methods described in JP-A Nos. 11-352627 and 2000-347335 are also preferred.

Concerning the method of forming tabular silver iodide grains, preferably used are those described in JP-A Nos. 59-119350 and 59-119344.

### 5) Grain Form

The form of tabular silver halide grains according to the present invention can be expressed by an aspect ratio which is well known in the art. A mean aspect ratio of the tabular silver halide grains according to the invention is from 2 to 100, more preferably from 3 to 80, and even more preferably from 5 to 50.

A mean thickness of the tabular silver halide grains according to the invention is preferably 0.3  $\mu\text{m}$  or less, more preferably 0.2  $\mu\text{m}$  or less, and even more preferably 0.15  $\mu\text{m}$  or less.

The silver halide having high silver iodide content of the invention can take a complicated form, and as the preferable form, there are listed, for example, connecting grains as shown in R. L. JENKINS et al., J. of Phot. Sci., vol. 28 (1980), p164, FIG. 1. Silver halide grains which are rounded at corners can also be used preferably. The surface indices (Miller indices) of the outer surface of a photosensitive silver halide grain is not particularly restricted, and it is preferable that the ratio occupied by the [100] face is large, because of showing high spectral sensitization efficiency when a spectral sensitizing dye is adsorbed. The ratio is preferably 50% or more, more preferably 65% or more and, further preferably 80% or more. The ratio of the [100] face, Miller index, can be determined by a method described in T. Tani; J. Imaging Sci., vol. 29, page 165, (1985) utilizing adsorption dependency of the [111] face and [100] face in adsorption of a sensitizing dye.

### 6) Heavy Metal

The photosensitive silver halide grain of the invention can contain metals or complexes of metals belonging to groups 3 to 14 of the periodic table (showing groups 1 to 18). Preferably, the photosensitive silver halide grain can contain metals or complexes of metals belonging to groups 6 to 10 of the periodic table. The metal or the center metal of the metal complex from groups 6 to 10 of the periodic table is preferably ferrum, rhodium, ruthenium, or iridium. The metal complex may be used alone, or two or more kinds of complexes comprising identical or different species of metals may be used together. The content is preferably in a range of from  $1 \times 10^{-9}$  mol to  $1 \times 10^{-3}$  mol per 1 mol of silver. The heavy metals, metal complexes and the addition method thereof are described in JP-A No. 7-225449, in paragraph Nos. 0018 to 0024 of JP-A No. 11-65021, and in paragraph Nos. 0227 to 0240 of JP-A No. 11-119374.

In the present invention, a silver halide grain having a hexacyano metal complex present on the outermost surface of the grain is preferred. The hexacyano metal complex includes, for example,  $[\text{Fe}(\text{CN})_6]^{4-}$ ,  $[\text{Fe}(\text{CN})_6]^{3-}$ ,  $[\text{Ru}(\text{CN})_6]^{4-}$ ,  $[\text{Os}(\text{CN})_6]^{4-}$ ,  $[\text{Co}(\text{CN})_6]^{3-}$ ,  $[\text{Rh}(\text{CN})_6]^{3-}$ ,  $[\text{Ir}(\text{CN})_6]^{3-}$ ,  $[\text{Cr}(\text{CN})_6]^{3-}$ , and  $[\text{Re}(\text{CN})_6]^{3-}$ . In the invention, hexacyano Fe complex is preferred.

Since the hexacyano complex exists in ionic form in an aqueous solution, paired cation is not important and alkali metal ion such as sodium ion, potassium ion, rubidium ion, cesium ion, and lithium ion, ammonium ion, and alkyl ammonium ion (for example, tetramethyl ammonium ion, tetraethyl

ammonium ion, tetrapropyl ammonium ion, and tetra(n-butyl) ammonium ion), which are easily miscible with water and suitable to precipitation operation of a silver halide emulsion are preferably used.

The hexacyano metal complex can be added while being mixed with water, as well as a mixed solvent of water and an appropriate organic solvent miscible with water (for example, alcohols, ethers, glycols, ketones, esters, amides, or the like) or gelatin.

The addition amount of the hexacyano metal complex is preferably from  $1 \times 10^{-5}$  mol to  $1 \times 10^{-2}$  mol and, more preferably, from  $1 \times 10^{-4}$  mol to  $1 \times 10^{-3}$ , per 1 mol of silver in each case.

In order to allow the hexacyano metal complex to be present on the outermost surface of a silver halide grain, the hexacyano metal complex is directly added in any stage of: after completion of addition of an aqueous solution of silver nitrate used for grain formation, before completion of an emulsion formation step prior to a chemical sensitization step, of conducting chalcogen sensitization such as sulfur sensitization, selenium sensitization, and tellurium sensitization or noble metal sensitization such as gold sensitization, during a washing step, during a dispersion step and before a chemical sensitization step. In order not to grow fine silver halide grains, the hexacyano metal complex is rapidly added preferably after the grain is formed, and it is preferably added before completion of an emulsion formation step.

Addition of the hexacyano complex may be started after addition of 96% by weight of an entire amount of silver nitrate to be added for grain formation, more preferably started after addition of 98% by weight and, particularly preferably, started after addition of 99% by weight.

When any of the hexacyano metal complexes is added after addition of an aqueous silver nitrate just before completion of grain formation, it can be adsorbed to the outermost surface of the silver halide grain and most of them form an insoluble salt with silver ions on the surface of the grain. Since silver salt of hexacyano iron (II) is a less soluble salt than AgI, re-dissolution with fine grains can be prevented and fine silver halide grains with smaller grain size can be prepared.

Metal atoms that can be contained in the silver halide grain used in the invention (for example,  $[\text{Fe}(\text{CN})_6]^{4-}$ ), desalting method of a silver halide emulsion and chemical sensitizing method are described in paragraph Nos. 0046 to 0050 of JP-A No. 11-84574, in paragraph Nos. 0025 to 0031 of JP-A No. 11-65021, and paragraph Nos. 0242 to 0250 of JP-A No. 11-119374.

### 7) Gelatin

As the gelatin contained the photosensitive silver halide emulsion used in the invention, various kinds of gelatins can be used. It is necessary to maintain an excellent dispersion state of a photosensitive silver halide emulsion in an organic silver salt containing coating solution, and low molecular weight gelatin having a molecular weight of from 500 to 60,000 is preferably used. These low molecular weight gelatins may be used at grain formation or at the time of dispersion after desalting treatment and it is preferably used at the time of dispersion after desalting treatment.

### 8) Chemical Sensitization

The photosensitive silver halide in the present invention can be used without chemical sensitization, but is preferably chemically sensitized by at least one of a chalcogen sensitizing method, gold sensitizing method, and reduction sensitizing method. The chalcogen sensitizing method includes sulfur sensitizing method, selenium sensitizing method and tellurium sensitizing method.

In sulfur sensitization, unstable sulfur compounds can be used. Such unstable sulfur compounds are described in Chimie et Pysique Photographique, written by P. Grafkides, (Paul Momtel, 5th ed., 1987) and Research Disclosure (vol.

307, Item 307105), and the like. As typical examples of sulfur sensitizers, known sulfur compounds such as thiosulfates (e.g., hypo), thioureas (e.g., diphenylthiourea, triethylthiourea, N-ethyl-N'-(4-methyl-2-thiazolyl)thiourea, or carboxymethyltrimeethylthiourea), thioamides (e.g., thioacetamide), rhodanines (e.g., diethylrhodanine or 5-benzylidene-N-ethylrhodanine), phosphinesulfides (e.g., trimethylphosphinesulfide), thiohydantoins, 4-oxo-oxazolidin-2-thiones, disulfides or polysulfides (e.g., dimorphorinedisulfide, cystine, or lenthionine (1,2,3,5,6-pentathiepane)), polythionates, and sulfur element, and active gelatin can be used. Specifically, thiosulfates, thioureas, and rhodanines are preferred.

In selenium sensitization, unstable selenium compounds can be used. These unstable selenium compounds are described in Japanese Patent Application Publication (JP-B) 15 Nos. 43-13489 and 44-15748, JP-A Nos. 4-25832, 4-109340, 4-271341, 5-40324, 5-11385, 6-51415, 6-175258, 6-180478, 6-208186, 6-208184, 6-317867, 7-92599, 7-98483, and 7-140579, and the like.

As typical examples of selenium sensitizers, colloidal metal selenide, selenoureas (e.g., N,N-dimethylselenourea, trifluoromethylcarbonyl-trimethylselenourea, or acetyltrimethylselenourea), selenoamides (e.g., selenoamide or N,N-dimethylphenylselenoamide), phosphineselenides (e.g., triphenylphosphineselenide or pentafluorophenyl-triphenylphosphineselenide), selenophosphates (e.g., tri-p-tolylselenophosphate or tri-n-butylselenophosphate), selenoketones (e.g., selenobenzophenone), isoselenocyanates, selenocarbonic acids, selenoesters, diacylselenides, or the like can be used. Furthermore, non-unstable selenium compounds such as selenius acid, salts of selenocyanic acid, selenazoles, and selenides described in JP-B Nos. 46-4553 and 52-34492, and the like can also be used. Specifically, phosphineselenides, selenoureas, and salts of selenocyanic acids are preferred.

In tellurium sensitization, unstable tellurium compounds are used. Unstable tellurium compounds described in JP-A Nos. 4-224595, 4-271341, 4-333043, 5-303157, 6-27573, 6-175258, 6-180478, 6-208186, 6-208184, 6-317867, 7-140579, 7-301879, 7-301880 and the like, can be used as a tellurium sensitizers.

As typical examples of a tellurium sensitizers, phosphine-tellurides (e.g., butyl-diisopropylphosphinetelluride, tributylphosphinetelluride, tributoxyphosphinetelluride, or ethoxy-diphenylphosphinetelluride), diacyl(di)tellurides (e.g., bis(diphenylcarbamoyl)ditelluride, bis(N-phenyl-N-methylcarbamoyl)ditelluride, bis(N-phenyl-N-methylcarbamoyl)ditelluride, bis(N-phenyl-N-benzylcarbamoyl)telluride, or bis(ethoxy carbonyl)telluride), telluroureas (e.g., N,N'-dimethylthiethylenetellurourea or N,N'-diphenylthiethylenetellurourea), telluramides, or telluroesters may be used. Specifically, diacyl(di)tellurides and phosphinetellurides are preferred. Especially, the compounds described in paragraph No. 0030 of JP-A No. 11-65021 and compounds represented by formulae (II), (III), or (IV) in JP-A No. 5-313284 are preferred.

Specifically, as for the chalcogen sensitization of the invention, selenium sensitization and tellurium sensitization are preferred, and tellurium sensitization is particularly preferred.

In gold sensitization, gold sensitizers described in Chimie et Pysique Photographique, written by P. Grafkides, (Paul Momtel, 5th ed., 1987) and Research Disclosure (vol. 307, Item 307105) can be used. More specifically, chloroauric acid, potassium chloroaurate, potassium aurithiocyanate, gold sulfide, gold selenide, or the like can be used. In addition to these, the gold compounds described in U.S. Pat. Nos. 2,642,361, 5,049,484, 5,049,485, 5,169,751, and 5,252,455, Belg. Patent No. 691857, and the like can also be used. Noble metal salts other than gold such as platinum, palladium, iridium and the like, which are described in Chimie et Pysique

## 11

Photographique, written by P. Grafkides, (Paul Momtel, 5th ed., 1987) and Research Disclosure (vol. 307, Item 307105), can also be used.

The gold sensitization can be used independently, but it is preferably used in combination with the above chalcogen sensitization. Specifically, these sensitizations are gold-sulfur sensitization (gold-plus-sulfur sensitization), gold-selenium sensitization, gold-tellurium sensitization, gold-sulfur-selenium sensitization, gold-sulfur-tellurium sensitization, gold-selenium-tellurium sensitization and gold-sulfur-selenium-tellurium sensitization.

In the invention, chemical sensitization can be applied at any time so long as it is after grain formation and before coating and it can be applied, after desalting, (1) before spectral sensitization, (2) simultaneously with spectral sensitization, (3) after spectral sensitization, (4) just before coating, or the like.

The addition amount of chalcogen sensitizer used in the invention may vary depending on the silver halide grain used, the chemical ripening condition, and the like, and it is about from  $10^{-8}$  mol to  $10^{-1}$  mol, and preferably, about from  $10^{-7}$  mol to  $10^{-2}$  mol, per 1 mol of silver halide.

Similarly, the addition amount of the gold sensitizer used in the invention may vary depending on various conditions and it is generally from  $10^{-7}$  mol to  $10^{-2}$  mol and, more preferably, from  $10^{-6}$  mol to  $5 \times 10^{-3}$  mol, per 1 mol of silver halide. There is no particular restriction on the condition for the chemical sensitization and, appropriately, the pAg is 8 or lower, preferably, 7.0 or lower, more preferably, 6.5 or lower and, particularly preferably, 6.0 or lower, and the pAg is 1.5 or higher, preferably, 2.0 or higher and, particularly preferably, 2.5 or higher; the pH is from 3 to 10, preferably, from 4 to 9; and the temperature is at from 20° C. to 95° C., preferably, from 25° C. to 80° C.

In the invention, reduction sensitization can also be used in combination with the chalcogen sensitization or the gold sensitization. It is specifically preferred to use in combination with the chalcogen sensitization.

As the specific compound for the reduction sensitization, ascorbic acid, thiourea dioxide, or dimethylamine borane is preferred, as well as use of stannous chloride, aminoimino methane sulfonic acid, hydrazine derivatives, borane compounds, silane compounds, polyamine compounds, and the like are preferred. The reduction sensitizer may be added at any stage in the photosensitive emulsion production process from crystal growth to the preparation step just before coating. Further, it is preferred to apply reduction sensitization by ripening while keeping the pH to 8 or higher and the pAg to 4 or lower for the emulsion, and it is also preferred to apply reduction sensitization by introducing a single addition portion of silver ions during grain formation.

The addition amount of the reduction sensitizer may also vary depending on various conditions and it is generally about  $10^{-7}$  mol to  $10^{-1}$  mol and, more preferably,  $10^{-6}$  mol to  $5 \times 10^{-3}$  mol per 1 mol of silver halide.

In the silver halide emulsion used in the invention, a thiosulfonate compound may be added by the method shown in EP-A No. 293917.

The photosensitive silver halide grain in the invention is preferably chemically sensitized by at least one method of gold sensitizing method and chalcogen sensitizing method for the purpose of designing a high-sensitivity photothermographic material.

9) Compound that can be one-electron-oxidized to provide a one-electron oxidation product which releases one or more electrons

The photothermographic material of the invention preferably contains a compound that can be one-electron-oxidized to provide a one-electron oxidation product which releases one or more electrons. The said compound can be used alone

## 12

or in combination with various chemical sensitizers described above to increase the sensitivity of silver halide.

As the compound that can be one-electron-oxidized to provide a one-electron oxidation product which releases one or more electrons is preferably a compound selected from the following Groups 1 or 2.

(Group 1) a compound that can be one-electron-oxidized to provide a one-electron oxidation product which further releases one or more electrons, due to being subjected to a subsequent bond cleavage reaction;

(Group 2) a compound that can be one-electron-oxidized to provide a one-electron oxidation product, which further releases one or more electrons after being subjected to a subsequent bond formation reaction.

The compound of Group 1 will be explained below.

In the compound of Group 1, as for a compound that can be one-electron-oxidized to provide a one-electron oxidation product which further releases one electron, due to being subjected to a subsequent bond cleavage reaction, specific examples include examples of compound referred to as "one photon two electrons sensitizer" or "deprotonating electron-donating sensitizer" described in JP-A No. 9-211769 (Compound PMT-1 to S-37 in Tables E and F, pages 28 to 32); JP-A No. 9-211774; JP-A No. 11-95355 (Compound INV 1 to 36); JP-W No. 2001-500996 (Compound 1 to 74, 80 to 87, and 92 to 122); U.S. Pat. Nos. 5,747,235 and 5,747,236; EP No. 786692A1 (Compound INV 1 to 35); EP No. 893732A1; U.S. Pat. Nos. 6,054,260 and 5,994,051; etc. Preferred ranges of these compounds are the same as the preferred ranges described in the quoted specifications.

In the compound of Group 1, as for a compound that can be one-electron-oxidized to provide a one-electron oxidation product which further releases one or more electrons, due to being subjected to a subsequent bond cleavage reaction, specific examples include the compounds represented by formula (1) (same as formula (1) described in JP-A No. 2003-114487), formula (2) (same as formula (2) described in JP-A No. 2003-114487), formula (3) (same as formula (1) described in JP-A No. 2003-114488), formula (4) (same as formula (2) described in JP-A No. 2003-114488), formula (5) (same as formula (3) described in JP-A No. 2003-114488), formula (6) (same as formula (1) described in JP-A No. 2003-75950), formula (7) (same as formula (2) described in JP-A No. 2003-75950), and formula (8), and the compound represented by formula (9) among the compounds which can undergo the chemical reaction represented by reaction formula (1). And the preferable range of these compounds is the same as the preferable range described in the quoted specification.

Formula (1)



Formula (2)



In formulae (1) and (2),  $RED_1$  and  $RED_2$  each independently represent a reducing group.  $R_1$  represents a nonmetallic atomic group forming a cyclic structure equivalent to a tetrahydro derivative or an octahydro derivative of a 5 or 6-membered aromatic ring (including a hetero aromatic ring) with a carbon atom (C) and  $RED_1$ .  $R_2$ ,  $R_3$ , and  $R_4$  each independently represent a hydrogen atom or a substituent.

$Lv_1$  and  $Lv_2$  each independently represent a leaving group.  
ED represents an electron-donating group.



In formulae (3), (4), and (5),  $Z_1$  represents an atomic group capable to form a 6-membered ring with a nitrogen atom and two carbon atoms of a benzene ring.  $R_5$ ,  $R_6$ ,  $R_7$ ,  $R_9$ ,  $R_{10}$ ,  $R_{11}$ ,  $R_{13}$ ,  $R_{14}$ ,  $R_{15}$ ,  $R_{16}$ ,  $R_{17}$ ,  $R_{18}$ , and  $R_{19}$  each independently represent a hydrogen atom or a substituent.  $R_{20}$  represents a hydrogen atom or a substituent, however, in the case where  $R_{20}$  represents a group other than an aryl group,  $R_{16}$  and  $R_{17}$  bind each other to form an aromatic ring or a hetero aromatic ring.  $R_8$  and  $R_{12}$  represent a substituent capable of substituting for a hydrogen atom on a benzene ring.  $m_1$  represents an integer of 0 to 3, and  $m_2$  represents an integer of 0 to 4.  $Lv_3$ ,  $Lv_4$ , and  $Lv_5$  each independently represent a leaving group.

Formula (3) 5



Formula (8)

In formula (8),  $RED_5$  is a reducing group and represents an arylamino group or a heterocyclic amino group.  $R_{31}$ , represents a hydrogen atom or a substituent.  $X$  represents one selected from an alkoxy group, an aryloxy group, a heterocyclic oxy group, an alkylthio group, an arylthio group, a heterocyclic thio group, an alkylamino group, an arylamino group, or a heterocyclic amino group.  $Lv_6$  is a leaving group and represents a carboxyl group or a salt thereof, or a hydrogen atom.

Formula (4)

15

20

Formula (5)

25

30

35

40

45

50

55

60

65

Reaction formula (1)



Formula (9)



The compound represented by formula (9) is a compound that undergoes a bonding reaction represented by reaction formula (1) after undergoing two-electrons-oxidation accompanied by decarbonization and further oxidized. In reaction formula (1),  $R_{32}$  and  $R_{33}$  represent a hydrogen atom or a substituent.  $Z_3$  represents a group to form a 5 or 6-membered heterocycle with  $C=C$ .  $Z_4$  represents a group to form a 5 or 6-membered aryl group or heterocyclic group with  $C=C$ .  $M$  represents one selected from a radical, a radical cation, and a cation. In formula (9),  $R_{32}$ ,  $R_{33}$ , and  $Z_3$  are the same as those in reaction formula (1).  $Z_5$  represents a group to form a 5 or 6-membered cyclic aliphatic hydrocarbon group or heterocyclic group with  $C=C$ .

Next, the compound of Group 2 is explained.

In the compound of Group 2, as for a compound that can be one-electron-oxidized to provide a one-electron oxidation product which further releases one or more electrons, after being subjected to a subsequent bond cleavage reaction, specific examples can include the compound represented by formula (10) (same as formula (1) described in JP-A No. 2003-140287), and the compound represented by formula (11) which can undergo the chemical reaction represented by



In formulae (6) and (7),  $RED_3$  and  $RED_4$  each independently represent a reducing group.  $R_{21}$  to  $R_{30}$  each independently represent a hydrogen atom or a substituent.  $Z_2$  represents one selected from  $-CR_{111}R_{112}-$ ,  $-NR_{113}-$ , or  $-O-$ .  $R_{111}$  and  $R_{112}$  each independently represent a hydrogen atom or a substituent.  $R_{113}$  represents one selected from a hydrogen atom, an alkyl group, an aryl group, or a heterocyclic group.

Formula (6)

45

Formula (7)

50

55

60

65

65

## 15

reaction formula (1). The preferable range of these compounds is the same as the preferable range described in the quoted specification.

RED<sub>6</sub>Q-Y

Formula (10)

In formula (10), RED<sub>6</sub> represents a reducing group which can be one-electron-oxidized. Y represents a reactive group containing a carbon-carbon double bond part, a carbon-carbon triple bond part, an aromatic group part, or benzo-condensed nonaromatic heterocyclic part which can react with one-electron-oxidized product formed by one-electron-oxidation of RED<sub>6</sub> to form a new bond. Q represents a linking group to link RED<sub>6</sub> and Y.



The compound represented by formula (11) is a compound that undergoes a bonding reaction represented by reaction formula (1) by being oxidized. In reaction formula (1), R<sub>32</sub> and R<sub>33</sub> each independently represent a hydrogen atom or a substituent. Z<sub>3</sub> represents a group to form a 5 or 6-membered heterocycle with C=C. Z<sub>4</sub> represents a group to form a 5 or 6-membered aryl group or heterocyclic group with C=C. Z<sub>5</sub> represents a group to form a 5 or 6-membered cyclic aliphatic hydrocarbon group or heterocyclic group with C=C. M represents one selected from a radical, a radical cation, and a cation. In formula (11), R<sub>32</sub>, R<sub>33</sub>, Z<sub>3</sub>, and Z<sub>4</sub> are the same as those in reaction formula (1).

The compounds of Groups 1 or 2 preferably are “the compound having an adsorptive group to silver halide in a molecule” or “the compound having a partial structure of a spectral sensitizing dye in a molecule”.

The representative adsorptive group to silver halide is the group described in JP-A No. 2003-156823, page 16 right, line 1 to page 17 right, line 12. A partial structure of a spectral sensitizing dye is the structure described in JP-A No. 2003-156823, page 17 right, line 34 to page 18 right, line 6.

As the compound of Groups 1 or 2, “the compound having at least one adsorptive group to silver halide in a molecule” is more preferred.

And, “the compound having two or more adsorptive groups to silver halide in a molecule” is further preferred. In the case

## 16

where two or more adsorptive groups exist in a single molecule, those adsorptive groups may be identical or different with each other.

As preferable adsorptive group, a mercapto-substituted nitrogen-containing heterocyclic group (e.g., a 2-mercaptopthiazole group, a 3-mercaptop-1,2,4-triazole group, a 5-mercaptopetetrazole group, a 2-mercaptop-1,3,4-oxadiazole group, a 2-mercaptopbenzoxazole group, a 2-mercaptopbenzothiazole group, a 1,5-dimethyl-1,2,4-triazolium-3-thiolate group, or the like) or a nitrogen-containing heterocyclic group having —NH— group as a partial structure of heterocycle capable to form a silver imidate (>NAg) (e.g., a benzotriazole group, a benzimidazole group, an indazole group, or the like) are described. A 5-mercaptopetetrazole group, a 3-mercaptop-1,2,4-triazole group and a benzotriazole group are particularly preferable and a 3-mercaptop-1,2,4-triazole group and a 5-mercaptopetetrazole group are most preferable.

As an adsorptive group, the group which has two or more mercapto groups as a partial structure in a molecule is also particularly preferable. Herein, a mercapto group (—SH) may become a thione group in the case where it can tautomerize. Preferred examples of an adsorptive group having two or more mercapto groups as a partial structure (dimercapto-substituted nitrogen-containing heterocyclic group and the like) are a 2,4-dimercaptopyrimidine group, a 2,4-dimercaptotriazine group and a 3,5-dimercapo-1,2,4-triazole group.

Further, a quaternary salt structure of nitrogen or phosphorus is also preferably used as an adsorptive group. As typical quaternary salt structure of nitrogen, an ammonio group (a trialkylammonio group, a dialkylarylammonio group, a dialkylheteroarylammonio group, an alkyldiheteroarylammonio group, or the like) and a nitrogen-containing heterocyclic group containing quaternary nitrogen atom can be used. As a quaternary salt structure of phosphorus, a phosphonio group (a trialkylphosphonio group, a dialkylarylphosphonio group, a dialkylheteroarylphosphonio group, an alkyldiheteroarylphosphonio group, a triarylphosphonio group, a triheteroarylphosphonio group, or the like) is described.

A quaternary salt structure of nitrogen is more preferably used and a 5 or 6-membered aromatic heterocyclic group containing a quaternary nitrogen atom is further preferably used. Particularly preferably, a pyridinio group, a quinolinio group and an isoquinolinio group are used. These nitrogen-containing heterocyclic groups containing a quaternary nitrogen atom may have any substituent.

Examples of counter anions of quaternary salt are a halogen ion, carboxylate ion, sulfonate ion, sulfate ion, perchlorate ion, carbonate ion, nitrate ion, BF<sub>4</sub><sup>-</sup>, PF<sub>6</sub><sup>-</sup>, Ph<sub>4</sub>B<sup>-</sup>, and the like. In the case where the group having negative charge at carboxylate group and the like exists in a molecule, an inner salt may be formed with it. As a counter ion outside of a molecule, chloro ion, bromo ion and methanesulfonate ion are particularly preferable.

The preferred structure of the compound represented by Groups 1 or 2 having a quaternary salt of nitrogen or phosphorus as an adsorptive group is represented by formula (X).

(P-Q<sub>1</sub>-)<sub>r</sub>R-(Q<sub>2</sub>-S)<sub>s</sub>

Formula (X)

In formula (X), P and R each independently represent a quaternary salt structure of nitrogen or phosphorus, which is not a partial structure of a spectral sensitizing dye. Q<sub>1</sub> and Q<sub>2</sub> each independently represent a linking group and typically represent a single bond, an alkylenic group, an arylene group, a heterocyclic group, —O—, —S—, —NR<sub>N</sub>, —C(=O)—, —SO<sub>2</sub>—, —SO—, —P(=O)— or combinations of these

17

groups. Herein,  $R_N$  represents one selected from a hydrogen atom, an alkyl group, an aryl group, or a heterocyclic group. S represents a residue which is obtained by removing one atom from the compound represented by Group 1 or 2. i and j are an integer of one or more and are selected in a range of  $i+j=2$  to 6.

The case where i is 1 to 3 and j is 1 to 2 is preferable, the case where i is 1 or 2 and j is 1 is more preferable, and the case

18

where i is 1 and j is 1 is particularly preferable. The compound represented by formula (X) preferably has 10 to 100 carbon atoms in total, more preferably 10 to 70 carbon atoms, further preferably 11 to 60 carbon atoms, and particularly preferably 12 to 50 carbon atoms in total.

Specific examples of the compounds of Groups 1 or 2 according to the invention are shown below without intention of restricting the scope of the invention.



19

20

-continued



-continued

17



18



19

20



21

22



23

24

-continued

23

24



25

26



27

28



29

30



25

26

-continued



31



32



33



34



37



36



-continued



-continued

45



46



47



30

The compounds of Groups 1 or 2 may be used at any time during preparation of the photosensitive silver halide emulsion and production of the photothermographic material. For example, the compound may be used in a photosensitive silver halide grain formation step, in a desalting step, in a chemical sensitization step, before coating, or the like. The compound may be added in several times during these steps. The compound is preferably added after the photosensitive silver halide grain formation step and before the desalting step; at the chemical sensitization step (just before the chemical sensitization to immediately after the chemical sensitization); or before coating. The compound is more preferably added at the chemical sensitization step or before coating.

It is preferred that the compound of Groups 1 or 2 according to the invention is dissolved in water, a water-soluble solvent such as methanol and ethanol, or a mixed solvent thereof. In the case where the compound is dissolved in water and solubility of the compound is increased by increasing or decreasing a pH value of the solvent, the pH value may be increased or decreased to dissolve and add the compound.

The compound of Groups 1 or 2 according to the invention is preferably used in the image forming layer. The compound may be added to a surface protective layer, or an intermediate layer, as well as the image forming layer, to be diffused to the image forming layer in the coating step. The compound may be added before or after addition of a sensitizing dye. Each compound is contained in the image forming layer preferably in an amount of from  $1 \times 10^{-9}$  mol to  $5 \times 10^{-2}$  mol, more preferably from  $1 \times 10^{-8}$  mol to  $2 \times 10^{-3}$  mol, per 1 mol of silver halide.

#### 10) Compound Having Adsorptive Group and Reducing Group

The photothermographic material of the present invention preferably comprises a compound having an adsorptive group

to silver halide and a reducing group in a molecule. It is preferred that the compound is represented by the following formula (I).

A-(W)n-B

Formula (I)

In formula (I), A represents a group capable of adsorption to a silver halide (hereafter, it is called an adsorptive group), W represents a divalent linking group, n represents 0 or 1, and B represents a reducing group.

In formula (I), the adsorptive group represented by A is a group to adsorb directly to a silver halide or a group to promote adsorption to a silver halide. As typical examples, a mercapto group (or a salt thereof), a thione group ( $-\text{C}(=\text{S})-$ ), a nitrogen atom, a heterocyclic group containing at

least one atom selected from a nitrogen atom, a sulfur atom, a selenium atom, or a tellurium atom, a sulfide group, a disulfide group, a cationic group, an ethynyl group, and the like are described.

The mercapto group as an adsorptive group means a mercapto group (and a salt thereof) itself and simultaneously more preferably represents a heterocyclic group or an aryl group or an alkyl group substituted by at least one mercapto group (or a salt thereof). Herein, as the heterocyclic group, a monocyclic or a condensed aromatic or nonaromatic heterocyclic group having at least a 5 to 7-membered ring, for example, an imidazole ring group, a thiazole ring group, an oxazole ring group, a benzimidazole ring group, a benzothiazole ring group, a benzoxazole ring group, a triazole ring group, a thiadiazole ring group, an oxadiazole ring group, a tetrazole ring group, a purine ring group, a pyridine ring group, a quinoline ring group; an isoquinoline ring group, a pyrimidine ring group, a triazine ring group, and the like are described. A heterocyclic group having a quaternary nitrogen atom may also be adopted, wherein a mercapto group as a substituent may dissociate to form a mesoion. When the mercapto group forms a salt, a counter ion of the salt may be a cation of an alkaline metal, an alkaline earth metal, a heavy

31

metal, or the like, such as  $\text{Li}^+$ ,  $\text{Na}^+$ ,  $\text{K}^+$ ,  $\text{Mg}^{2+}$ ,  $\text{Ag}^+$  and  $\text{Zn}^{2+}$ ; an ammonium ion; a heterocyclic group containing a quaternary nitrogen atom; a phosphonium ion; or the like.

Further, the mercapto group as an adsorptive group may become a thione group by a tautomerization.

The thione group used as the adsorptive group also include a linear or cyclic thioamide group, thioureide group, thio-urethane group, and dithiocarbamate ester group.

The heterocyclic group, as an adsorptive group, which contains at least one atom selected from a nitrogen atom, a sulfur atom, a selenium atom, or a tellurium atom, represents a nitrogen-containing heterocyclic group having  $-\text{NH}-$  group, as a partial structure of a heterocycle, capable to form a silver iminate ( $>\text{N}=\text{Ag}$ ) or a heterocyclic group, having an  $-\text{S}-$  group, a  $-\text{Se}-$  group, a  $-\text{Te}-$  group or a  $-\text{N}-$  group as a partial structure of a heterocycle, and capable to coordinate to a silver ion by a chelate bonding. As the former examples, a benzotriazole group, a triazole group, an indazole group, a pyrazole group, a tetrazole group, a benzimidazole group, an imidazole group, a purine group, and the like are described. As the latter examples, a thiophene group, a thiazole group, an oxazole group, a benzophthiophene group, a benzothiazole group, a benzoazazole group, a thiadiazole group, an oxadiazole group, a triazine group, a selenoazole group, a benzoselenazole group, a tellurazole group, a benzotellurazole group, and the like are described.

The sulfide group or disulfide group as an adsorptive group contains all groups having  $-\text{S}-$  or  $-\text{S}-\text{S}-$  as a partial structure.

The cationic group as an adsorptive group means the group containing a quaternary nitrogen atom, such as an ammonium group or a nitrogen-containing heterocyclic group including a quaternary nitrogen atom. As examples of the heterocyclic group containing a quaternary nitrogen atom, a pyridinio group, a quinolinio group, an isoquinolinio group, an imidazolio group, and the like are described.

The ethynyl group as an adsorptive group means  $-\text{C}\equiv\text{CH}$  group and the said hydrogen atom may be substituted.

The adsorptive group described above may have any substituent. Further, as typical examples of an adsorptive group, the compounds described in pages 4 to 7 in the specification of JP-A No. 11-95355 are described. As an adsorptive group represented by A in formula (I), a heterocyclic group substituted by a mercapto group (e.g., a 2-mercaptopthiadiazole group, a 2-mercaptop-5-aminothiadiazole group, a 3-mercaptop-1,2,4-triazole group, a 5-mercaptopetetrazole group, a 2-mercaptop-1,3,4-oxadiazole group, a 2-mercaptopbenzimidazole group, a 1,5-dimethyl-1,2,4-triazorium-3-thiolate group, a 2,4-dimercaptopyrimidine group, a 2,4-dimercaptotriazine group, a 3,5-dimercapto-1,2,4-triazole group, a 2,5-dimercapto-1,3-thiazole group, or the like) and a nitrogen atom containing heterocyclic group having an  $-\text{NH}-$  group capable to form an imino-silver ( $>\text{N}=\text{Ag}$ ) as a partial structure of heterocycle (e.g., a benzotriazole group, a benzimidazole group, an indazole group, or the like) are preferable, and more preferable as an adsorptive group are a 2-mercaptopbenzimidazole group and a 3,5-dimercapto-1,2,4-triazole group.

In formula (I), W represents a divalent linking group. The said linking group may be any divalent linking group, as far as it does not give a bad effect toward photographic properties. For example, a divalent linking group which includes a carbon atom, a hydrogen atom, an oxygen atom, a nitrogen atom, or a sulfur atom, can be used. As typical examples, an alkylene group having 1 to 20 carbon atoms (e.g., a methylene group, an ethylene group, a trimethylene group, a tetramethylene group, a hexamethylene group, or the like), an alkynylene group having 2 to 20 carbon atoms, an alkynynylene

32

group having 2 to 20 carbon atoms, an arylene group having 6 to 20 carbon atoms (e.g., a phenylene group, a naphthylene group, or the like),  $-\text{CO}-$ ,  $-\text{SO}_2-$ ,  $-\text{O}-$ ,  $-\text{S}-$ ,  $-\text{NR}_1-$ , and the combinations of these linking groups are described. Herein,  $\text{R}_1$  represents a hydrogen atom, an alkyl group, a heterocyclic group, or an aryl group.

The linking group represented by W may have any substituent.

In formula (I), a reducing group represented by B represents the group capable to reduce a silver ion. As the examples, a formyl group, an amino group, a triple bond group such as an acetylene group, a propargyl group and the like, a mercapto group, and residues which are obtained by removing one hydrogen atom from hydroxylamines, hydroxamic acids, hydroxyureas, hydroxyurethanes, hydroxysemicarbazides, reductones (reductone derivatives are contained), anilines, phenols (chroman-6-ols, 2,3-dihydrobenzofuran-5-ols, aminophenols, sulfonamidophenols, and polyphenols such as hydroquinones, catechols, resorcinols, benzenetriols, bisphenols are included), acylhydrazines, carbamoylhydrazines, 3-pyrazolidones, and the like can be described. They may have any substituent.

The oxidation potential of a reducing group represented by B in formula (I), can be measured by using the measuring method described in Akira Fujishima, "DENKIKAGAKU SOKUTEIHO", pages 150 to 208, GIHODO SHUPPAN and The Chemical Society of Japan, "ZIKKEN-KAGAKUKOZA", 4th ed., vol. 9, pages 282 to 344, MARUZEN. For example, the method of rotating disc voltammetry can be used; namely the sample is dissolved in the solution (methanol:pH 6.5 Britton-Robinson buffer=10%: 90% (% by volume)) and after bubbling with nitrogen gas during 10 minutes the voltamograph can be measured under the conditions of 1000 rotations/minute, the sweep rate 20 mV/second, at 25° C. by using a rotating disc electrode (RDE) made by glassy carbon as a working electrode, a platinum electrode as a counter electrode and a saturated calomel electrode as a reference electrode. The half wave potential ( $E^{1/2}$ ) can be calculated by that obtained voltamograph. When a reducing group represented by B in the present invention is measured by the method described above, an oxidation potential is preferably in a range of from about -0.3 V to about 1.0 V, more preferably from about -0.1 V to about 0.8 V, and particularly preferably about from 0 to about 0.7 V.

In formula (I), a reducing group represented by B is preferably a residue which is obtained by removing one hydrogen atom from hydroxylamines, hydroxamic acids, hydroxyureas, hydroxysemicarbazides, reductones, phenols, acylhydrazines, carbamoylhydrazines, or 3-pyrazolidones.

The compound of formula (I) according to the present invention may have the ballasted group or polymer chain in it generally used in the non-moving photographic additives as a coupler. And as a polymer, for example, the polymer described in JP-A No. 1-100530 can be selected.

The compound of formula (I) according to the present invention may be bis or tris type of compound. The molecular weight of the compound represented by formula (I) according to the present invention is preferably from 100 to 10000, more preferably from 120 to 1000, and particularly preferably from 150 to 500.

The examples of the compound represented by formula (I) according to the present invention are shown below, but the present invention is not limited in these.

33



34

-continued

(7)



-continued



The preferred addition amount is largely dependent on the adding method described above or the kind of the compound, but generally from  $1 \times 10^{-6}$  mol to 1 mol, preferably from  $1 \times 10^{-5}$  mol to  $5 \times 10^{-1}$  mol, and more preferably from  $1 \times 10^{-4}$  mol to  $1 \times 10^{-1}$  mol, per 1 mol of photosensitive silver halide in each case.

The compound represented by formula (I) according to the present invention can be added by dissolving in water or water-soluble solvent such as methanol, ethanol and the like or a mixed solution thereof. At this time, the pH may be arranged suitably by an acid or an alkaline and a surfactant can coexist. Further, these compounds can be added as an emulsified dispersion by dissolving them in an organic solvent having a high boiling point and also can be added as a solid dispersion.

**(Compound which Substantially Reduces Haze by Photosensitive Silver Halide after Thermal Development)**

In the present invention, it is preferred that the photothermographic material contains a compound which substantially reduces haze by photosensitive silver halide after thermal development versus before thermal development.

In the present invention, it is particularly preferred that a silver iodide complex-forming agent is used as the compound which substantially reduces haze by photosensitive silver halide after thermal development.

**<Silver Iodide Complex-Forming Agent>**

Concerning the silver iodide complex-forming agent according to the present invention, at least one of a nitrogen atom or a sulfur atom in the compound can contribute to a Lewis acid-base reaction which gives an electron to a silver ion, as a ligand atom (electron donor: Lewis base). The stability of the complex is defined by successive stability constant or total stability constant, but it depends on the combination of silver ion, iodo ion and the silver complex forming agent. As a general guide, it is possible to obtain a large stability constant by a chelate effect from intramolecular chelate ring formation, by means of increasing the acid-base dissociation constant, or the like.

The haze of the photosensitive silver halide can be measured by a commercially available turbidimeter or a haze measuring apparatus. When the absorption derived from other compounds added to the photothermographic material overlaps with the absorption of photosensitive silver halide, the haze of photosensitive silver halide can be observed by using,

independently or in combination, the means of difference spectrum or removal of other compounds by solvent, or the like.

As a silver iodide complex-forming agent according to the present invention, a 5 to 7-membered heterocyclic compound containing at least one nitrogen atom is preferable. In the case where the compound does not have a mercapto group, a sulfide group, or a thione group as a substituent, the said nitrogen containing 5 to 7-membered heterocycle may be 10 saturated or unsaturated, and may have another substituent. The substituent on a heterocycle may bind to each other to form a ring.

As preferable examples of 5 to 7-membered heterocyclic compounds, pyrrole, pyridine, oxazole, isoxazole, thiazole, isothiazole, imidazole, pyrazole, pyrazine, pyrimidine, pyridazine, indole, isoindole, indolizine, quinoline, isoquinoline, benzimidazole, 1H-imidazole, quinoxaline, quinazoline, cinnoline, phthalazine, naphthylizine, purine, pterazine, carbazole, acridine, phenanthroline, phenanthroline, phenazine, phenoxazine, phenothiazine, benzothiazole, benzoxazole, 1,2,4-triazine, 1,3,5-triazine, pyrrolidine, imidazoline, pyrazolidine, piperidine, piperazine, morpholine, indoline, isoindoline, and the like can be described. More preferably, pyridine, imidazole, pyrazole, pyrazine, pyrimidine, pyridazine, indole, isoindole, indolizine, quinoline, isoquinoline, benzimidazole, 1H-imidazole, quinoxaline, quinazoline, cinnoline, phthalazine, 1,8-naphthylizine, 1,10-phenanthroline, benzotriazole, 1,2,4-triazine, 1,3,5-triazine, and the like can be described. Particularly preferably, pyridine, imidazole, pyrazine, pyrimidine, pyridazine, phthazine, triazine, 1,8-naphthylizine, 1,10-phenanthroline, and the like can be described.

These rings may have a substituent and any substituent can be used as far as it does not negatively impact the photographic property.

As preferable examples, a halogen atom (fluorine atom, chlorine atom, bromine atom, or iodine atom), an alkyl group (a straight, a branched, a cyclic alkyl group containing a bicycloalkyl group and an active methine group), an alkenyl group, an alkynyl group, an aryl group, a heterocyclic group (substituted position is not asked), an acyl group, an alkoxy-carbonyl group, an aryloxycarbonyl group, a heterocyclic oxycarbonyl group, a carbamoyl group, an N-acylcarbamoyl group, an N-sulfonylcarbamoyl group, an N-carbamoylcarbamoyl group, an N-sulfamoylcarbamoyl group, a carbazoyl group, a carboxyl group and a salt thereof, an oxazyl group, an oxamoyl group, a cyano group, a carbonimidoyl group, a formyl group, a hydroxy group, an alkoxy group (including the group in which ethylene oxy group units or propylene oxy group units are repeated), an aryloxy group, a heterocyclic oxy group, an acyloxy group, an alkoxy carbonyloxy group, an aryloxycarbonyloxy group, a carbamoyloxy group, a sulfonyloxy group, an amino group, an alkylamino group, an arylamino group, a heterocyclic amino group, an acylamino group, a sulfonamide group, a ureido group, a thioureido group, an imide group, an alkoxy carbonyl amino group, an aryloxycarbonyl amino group, a sulfamoyl amino group, a semicarbazide group, an ammonio group, an oxamoyl amino group, an N-alkylsulfonylureido group, an N-arylsulfonylureido group, an N-acylureido group, an N-acylsulfamoyl amino group, a nitro group, a heterocyclic group containing a quaternary nitrogen atom (e.g., a pyridinio group, an imidazolio group, a quinolinio group, or an isoquinolinio group), an isocyanogroup, an imino group, an alkylsulfonyl group, an arylsulfonyl group, an alkylsulfinyl group, an arylsulfinyl group, a sulfo group and a salt thereof, a sulfamoyl group, an N-acylsulfamoyl group, an N-sulfonylsulfamoyl group and a

salt thereof, a phosphino group, a phosphinyl group, a phosphinyloxy group, a phosphinylamino group, a silyl group, and the like are described. Here, an active methine group means a methine group substituted by two electron-attracting groups, wherein the electron-attracting group means an acyl group, an alkoxy carbonyl group, an aryloxycarbonyl group, a carbamoyl group, an alkylsulfonyl group, an arylsulfonyl group, a sulfamoyl group, a trifluoromethyl group, a cyano group, a nitro group, a carbonimidoyl group. Herein, two electron-attracting groups may bind each other to form a cyclic structure. And, the salt means a salt formed with positive ion such as an alkaline metal, an alkaline earth metal, a heavy metal, or the like, or organic positive ion such as an ammonium ion, a phosphonium ion, or the like. These substituents may be further substituted by these substituents.

These heterocycles may be further condensed by another ring. In the case where the substituent is an anion group (e.g.,  $-\text{CO}_2^-$ ,  $-\text{SO}_3^-$ ,  $-\text{S}^-$ , or the like), the heterocycle containing nitrogen atom of the invention may become a positive ion (e.g., pyridinium, 1,2,4-triazolium, or the like) and may form an intramolecular salt.

In the case where a heterocyclic compound is pyridine, pyrazine, pyrimidine, pyridazine, phthalazine, triazine, naphthalazine, or phenanthroline derivative, the acid dissociation constant ( $\text{pKa}$ ) of a conjugated acid of nitrogen containing heterocyclic part in acid dissociation equilibrium of the said compound preferably is from 3 to 8 in the mixture solution of tetrahydrofuran/water (3/2) at 25°C., and more preferably, the  $\text{pKa}$  is from 4 to 7.

As the heterocyclic compound, pyridine, pyridazine, and phthalazine derivative are preferable, and particularly preferable are pyridine and phthalazine derivative.

In the case where these heterocyclic compounds have a mercapto group, a sulfide group or a thione group as the substituent, pyridine, thiazole, isothiazole, oxazole, isoxazole, imidazole, pyrazole, pyrazine, pyrimidine, pyridazine, triazine, triazole, thiadiazole, and oxadiazole derivatives are preferable, and thiazole, imidazole, pyrazole, pyrazine, pyrimidine, pyridazine, triazine, and triazole derivatives are particularly preferable.

For example, as the said silver iodide complex-forming agent, the compound represented by the following formulae (1) or (2) can be used.



In formula (1),  $\text{R}^{11}$  and  $\text{R}^{12}$  each independently represent a hydrogen atom or a substituent. In formula (2),  $\text{R}^{21}$  and  $\text{R}^{22}$  each independently represent a hydrogen atom or a substituent. However, both of  $\text{R}^{11}$  and  $\text{R}^{12}$  are not hydrogen atoms together and both of  $\text{R}^{21}$  and  $\text{R}^{22}$  are not hydrogen atoms together. As the substituent herein, the substituent explained as the substituent of a 5 to 7-membered nitrogen containing heterocyclic type silver iodide complex-forming agent mentioned above can be described.

Further, the compound represented by formula (3) described below can also be used preferably.



Formula (3)

10

In formula (3),  $\text{R}^{31}$  to  $\text{R}^{35}$  each independently represent a hydrogen atom or a substituent. As the substituent represented by  $\text{R}^{31}$  to  $\text{R}^{35}$ , the substituent of a 5 to 7-membered nitrogen containing heterocyclic type silver iodide complex-forming agent mentioned above can be used. In the case where the compound represented by formula (3) has a substituent, preferred substituting position is  $\text{R}^{32}$  to  $\text{R}^{34}$ .  $\text{R}^{31}$  to  $\text{R}^{35}$  may bind each other to form a saturated or an unsaturated ring. A preferred substituent is a halogen atom, an alkyl group, an aryl group, a carbamoyl group, a hydroxy group, an alkoxy group, an aryloxy group, a carbamoyloxy group, an amino group, an acylamino group, a ureido group, an alkoxy-carbonylamino group, an aryloxycarbonylamino group, or the like.

In the compound represented by formula (3), the acid dissociation constant ( $\text{pKa}$ ) of conjugated acid of pyridine ring part is preferably from 3 to 8 in the mixed solution of tetrahydrofuran/water (3/2) at 25°C., and particularly preferably from 4 to 7.

Furthermore, the compound represented by formula (4) is also preferable.



Formula (4)

35

In formula (4),  $\text{R}^{41}$  to  $\text{R}^{44}$  each independently represent a hydrogen atom or a substituent.  $\text{R}^{41}$  to  $\text{R}^{44}$  may bind each other to form a saturated or an unsaturated ring. As the substituent represented by  $\text{R}^{41}$  to  $\text{R}^{44}$ , the substituent of a 5 to 7-membered nitrogen containing heterocyclic type silver iodide complex-forming agent mentioned above can be described. As preferred group, an alkyl group, an alkenyl group, an alkynyl group, an aryl group, a hydroxy group, an alkoxy group, an aryloxy group a heterocyclic oxy group, and a group which forms a phthalazine ring by benzo-condensation are described. In the case where a hydroxy group exists at the carbon atom adjacent to nitrogen atom of the compound represented by formula (4), there exists equilibrium between pyridazinone.

The compound represented by formula (4) more preferably forms a phthalazine ring represented by the following formula (5), and furthermore, this phthalazine ring particularly preferably has at least one substituent. As examples of  $\text{R}^{51}$  to  $\text{R}^{56}$  in formula (5), the substituent of a 5 to 7-membered nitrogen containing heterocyclic type silver iodide complex-forming agent mentioned above can be described. And as more preferable examples of the substituent, an alkyl group, an alkenyl group, an alkynyl group, an aryl group, a hydroxy group, an alkoxy group, an aryloxy group, and the like are

39

described. An alkyl group, an alkenyl group, an aryl group, an alkoxy group, and an aryloxy group are preferable and an alkyl group, an alkoxy group, and an aryloxy group are more preferable.



Formula (5)

40

group, an aryloxycarbonyl group, an alkoxy carbonyl group, a carbamoyl group, an imide group, and the like are described as examples.

Among the silver iodide complex-forming agents described above, the compounds represented by formulae (3), (4), (5), (6), or (7) are more preferable and, the compounds represented by formulae (3) or (5) are particularly preferable.

Preferable examples of silver iodide complex-forming agent are described below, however the present invention is not limited in these.

Further, the compound represented by formula (6) described below is also a preferable embodiment.



Formula (6)

In formula (6), R<sup>61</sup> to R<sup>63</sup> each independently represent a hydrogen atom or a substituent. As examples of the substituent represented by R<sup>62</sup>, the substituent of a 5 to 7-membered nitrogen containing heterocyclic type silver iodide complex-forming agent mentioned above can be described.

As the compound preferably used, the compound represented by the following formula (7) is described.



Formula (7)

In formula (7), R<sup>71</sup> and R<sup>72</sup> each independently represent a hydrogen atom or a substituent. L represents a divalent linking group. n represents 0 or 1. As the substituent represented by R<sup>71</sup> and R<sup>72</sup>, an alkyl group (containing a cycloalkyl group), an alkenyl group (containing a cycloalkenyl group), an alkynyl group, an aryl group, a heterocyclic group, an acyl group, an aryloxycarbonyl group, an alkoxy carbonyl group, a carbamoyl group, an imide group, and a complex substituent containing these groups are described as examples. A divalent linking group represented by L preferably has the length of 1 to 6 atoms and more preferably has the length of 1 to 3 atoms, and furthermore, may have a substituent.

One more of the compounds preferably used is a compound represented by formula (8).



Formula (8)

In formula (8), R<sup>81</sup> to R<sup>84</sup> each independently represent a hydrogen atom or a substituent. As the substituent represented by R<sup>81</sup> to R<sup>84</sup>, an alkyl group (including a cycloalkyl group), an alkenyl group (including a cycloalkenyl group), an alkynyl group, an aryl group, a heterocyclic group, an acyl



(1)



(2)



(3)



(4)

C<sub>5</sub>H<sub>11</sub>SC<sub>5</sub>H<sub>11</sub>

(5)

C<sub>4</sub>H<sub>9</sub>SCH<sub>2</sub>CH<sub>2</sub>SC<sub>4</sub>H<sub>9</sub>

(6)



(7)



(8)



(9)



(10)

**41**

-continued

**42**

-continued

(11)



5

(12)



15

(13)



20

(14)



30

(15)



35

(16)



40

(17)



45

(18)



55

(19)



60

(20)



(21)

(22)

(23)

(24)

(25)

(26)

(27)

(28)

(29)

(30)

(31)

-continued



The silver iodide complex-forming agent according to the present invention can also be a compound common to a toner,

in the case where the agent achieves the function of conventionally known toner. The silver iodide complex-forming agent according to the present invention can be used in combination with a toner. And, two or more kinds of the silver iodide complex-forming agents may be used in combination.

The silver iodide complex-forming agent according to the present invention preferably exists in a film under the state separated from a photosensitive silver halide, such as a solid state or the like. It is also preferably added to the layer adjacent to the image forming layer. Concerning the silver iodide complex-forming agent according to the present invention, a melting point of the compound is preferably adjusted to a suitable range so that it can be dissolved when heated at thermal developing temperature.

15 The silver iodide complex-forming agent according to the invention may be incorporated into a photothermographic material by being added into the coating solution, such as in the form of a solution, an emulsion dispersion, a solid fine particle dispersion, or the like.

20 Well known emulsion dispersing methods include a method comprising dissolving the silver iodide complex-forming agent in an oil such as dibutylphthalate, tricresylphosphate, glyceryl triacetate, diethylphthalate, or the like, using an auxiliary solvent such as ethyl acetate, cyclohexanone, or the like, followed by mechanically forming an emulsified dispersion.

25 Solid fine particle dispersing methods include a method comprising dispersing the powder of the silver iodide complex-forming agent according to the invention in a proper solvent such as water or the like, by means of ball mill, colloid mill, vibrating ball mill, sand mill, jet mill, roller mill, or ultrasonics, thereby obtaining a solid dispersion.

30 In this case, there can also be used a protective colloid (such as poly(vinyl alcohol)), or a surfactant (for instance, an anionic surfactant such as sodium triisopropylnaphthalene-sulfonate (a mixture of compounds having the three isopropyl groups in different substitution sites)). In the mills enumerated above, generally used as the dispersion media are beads made of zirconia and the like, and Zr and the like eluting from 35 the beads may be incorporated in the dispersion. Depending on the dispersing conditions, the amount of Zr and the like generally incorporated in the dispersion is in a range of from 1 ppm to 1000 ppm. It is practically acceptable so long as Zr is incorporated in the photothermographic material in an 40 amount of 0.5 mg or less per 1 g of silver.

45 Preferably, an antiseptic (for instance, benzisothiazolinone sodium salt) is added in the water dispersion.

The silver iodide complex-forming agent according to the invention is preferably used in the form of a solid dispersion.

50 The silver iodide complex-forming agent according to the invention is preferably used in a range of from 1 mol % to 5000 mol %, more preferably, from 10 mol % to 1000 mol % and, even more preferably, from 50 mol % to 300 mol %, with respect to the photosensitive silver halide in each case.

(41) 55 (Organic Silver Salt)

The organic silver salt used in the invention is relatively stable to light but serves as to supply silver ions and forms silver images when heated to 80° C. or higher under the presence of an exposed photosensitive silver halide and a reducing agent. The organic silver salt may be any organic material containing a source capable of reducing silver ions. Such a non-photosensitive organic silver salt is disclosed, for example, in JP-A No. 10-62899 (paragraph Nos. 0048 to 0049), EP No. 0803764A1 (page 18, line 24 to page 19, line 37), EP No. 0962812A1, JP-A Nos. 11-349591, 2000-7683, and 2000-72711, and the like. A silver salt of an organic acid, particularly, a silver salt of long chained fatty acid carboxylic

45

acid (having 10 to 30 carbon atoms, preferably, having 15 to 28 carbon atoms) is preferable. Preferred examples of the organic silver salt can include, for example, silver behenate, silver arachidinate, silver stearate, silver oleate, silver laurate, silver capronate, silver myristate, silver palmitate and mixtures thereof. In the present invention, among the organic silver salts, it is preferred to use an organic silver salt with a silver behenate content of 50 mol % or higher, and particularly preferably, from 75 mol % or higher.

There is no particular restriction on the shape of the organic silver salt usable in the invention and it may be needle-like, bar-like, tabular, or flake shaped.

In the invention, a flake shaped organic silver salt is preferred. In the present specification, the flake-shaped organic silver salt is defined as described below. When an organic acid silver salt is observed under an electron microscope, calculation is made while approximating the shape of an organic acid silver salt particle to a rectangular body and assuming each side of the rectangular body as a, b, c from the shorter side (c may be identical with b) and determining x based on numerical values a, b for the shorter side as below.

$$x = b/a$$

As described above, x is determined for the particles by the number of about 200 and those capable of satisfying the relation:  $x(\text{average}) \geq 1.5$  as an average value x is defined as a flake shape. The relation is preferably:  $30 \geq x(\text{average}) \geq 1.5$  and, more preferably,  $15 \geq x(\text{average}) \geq 1.5$ . By the way, needle-like is expressed as  $1 \leq x(\text{average}) < 1.5$ .

In the flake shaped particle, a can be regarded as a thickness of a tabular particle having a main plate with b and c being as the sides. a in average is preferably from 0.01  $\mu\text{m}$  to 0.3  $\mu\text{m}$  and, more preferably, from 0.1  $\mu\text{m}$  to 0.23  $\mu\text{m}$ . c/b in average is preferably from 1 to 6, more preferably from 1 to 4, further preferably from 1 to 3 and, particularly preferably from 1 to 2.

Concerning the particle size distribution of the organic silver salt, monodispersion is preferred. In the monodispersion, the percentage for the value obtained by dividing the standard deviation for the length of minor axis and major axis by the minor axis and the major axis respectively is, preferably, 100% or less, more preferably, 80% or less and, further preferably, 50% or less. The shape of the organic silver salt can be measured by analyzing a dispersion of an organic silver salt using transmission type electron microscopic images. Another method of measuring the monodispersion is a method of determining of the standard deviation of the volume weighted mean diameter of the organic silver salt in which the percentage for the value defined by the volume weight mean diameter (variation coefficient), is preferably, 100% or less, more preferably, 80% or less and, further preferably, 50% or less. The monodispersion can be determined from particle size (volume weighted mean diameter) obtained, for example, by a measuring method of irradiating a laser beam to an organic silver salt dispersed in a liquid, and determining a self correlation function of the fluctuation of scattered light to the change of time.

Methods known in the art may be applied to the method for producing the organic silver salt used in the invention and to the dispersing method thereof. For example, reference can be made to JP-A No. 1062899, EP Nos. 0803763A1 and 0962812A1, JP-A Nos. 11-349591, 2000-7683, 2000-72711, 2001-163827, 2001-163889, 2001-163890, 11-203413, 2001-188313, 2001-83652, 2002-6442, 2002-31870, 2000-214155, 2002-6442, and the like.

In the invention, the photothermographic material can be prepared by mixing an aqueous dispersion of an organic silver salt and an aqueous dispersion of a photosensitive silver salt.

46

A method of mixing two or more kinds of aqueous dispersions of organic silver salts and two or more kinds of aqueous dispersions of photosensitive silver salts upon mixing are used preferably for controlling the photographic properties.

While an organic silver salt in the invention can be used in a desired amount, an amount of an organic silver salt is preferably in a range of from 0.1 g/m<sup>2</sup> to 5 g/m<sup>2</sup>, more preferably from 1 g/m<sup>2</sup> to 3 g/m<sup>2</sup>, and particularly preferably from 1.2 g/m<sup>2</sup> to 2.5 g/m<sup>2</sup>, with respect to the amount of silver.

(Nucleator)

The photothermographic material of the present invention preferably contains a nucleator.

The nucleator according to the present invention is a compound, which can form a compound that can newly induce a development by the reaction with a developing product in consequence of an initial development. It was conventionally known to use a nucleator for the ultra-high gradation photosensitive materials suitable for the use in graphic arts. The ultra-high gradation photosensitive materials had an average gradient of 10 or more and were unsuitable for conventional photographic materials, and especially unsuitable for the medical use where high diagnostic ability was required. And because the ultra-high gradation photosensitive material had rough granularity and did not have enough sharpness, there was no potential for medical diagnostic use.

The nucleator in the present invention completely differs from the nucleator in the conventional ultra-high gradation photosensitive material as regards the effect. The nucleator in the present invention does not make a hard gradation.

The nucleator in the present invention is the compound that can cause development sufficiently, even if the number of photosensitive silver halide grains with respect to non-photosensitive silver salt of an organic acid is extremely low. Although that mechanism is not clear, when thermal development is performed using the nucleator according to the present invention, it becomes clear that a large number of developed silver grains exists than the number of photosensitive silver halide grains in the maximum density part, and it is presumed that the nucleator according to the present invention forms the new development points (development nuclei) in those portions where silver halide grains do not exist.

As the nucleator, hydrazine derivative compounds represented by the following formula (V), vinyl compounds represented by the following formula (VI), and quaternary onium compounds represented by the following formula (P) are preferable. In particular, among the vinyl compounds, cyclic olefine compounds represented by formulae (A), (B), or (C) are preferable.



Formula (V)



Formula (VI)



Formula (P)

-continued



Formula (A)



Formula (B)



Formula (C)

In formula (V),  $A_0$  represents one selected from an aliphatic group, an aromatic group, a heterocyclic group, or a  $-G_0-D_0$  group, each of which may have a substituent.  $B_0$  represents a blocking group.  $A_1$  and  $A_2$  both represent a hydrogen atom, or one represents a hydrogen atom and the other represents one of an acyl group, a sulfonyl group, and an oxalyl group. Wherein,  $G_0$  represents one selected from a  $-CO-$  group, a  $-COCO-$  group, a  $-CS-$  group, a  $-C(=NG_1D_1)-$  group, an  $-SO-$  group, an  $-SO_2-$  group, or a  $-P(O)(G_1D_1)-$  group.  $G_1$  represents one selected from a mere bonding hand, an  $-O-$  group, an  $-S-$  group, or an  $-N(D_1)-$  group, and  $D_1$  represents one selected from an aliphatic group, an aromatic group, a heterocyclic group, or a hydrogen atom. In the case where plural  $D_1$ 's exist in a molecule, they may be the same or different.  $D_0$  represents one selected from a hydrogen atom, an aliphatic group, an aromatic group, a heterocyclic group, an amino group, an alkoxy group, an aryloxy group, an alkylthio group, or an arylthio group. As preferable  $D_0$ , a hydrogen atom, an alkyl group, an alkoxy group, an amino group, and the like can be described.

In formula (V), the aliphatic group represented by  $A_0$  preferably has 1 to 30 carbon atoms, and particularly preferably is a normal, branched or cyclic alkyl group having 1 to 20 carbon atoms. For example, a methyl group, an ethyl group, a t-butyl group, an octyl group, a cyclohexyl group, and a benzyl group are described. These may be further substituted by a suitable substituent (e.g., an aryl group, an alkoxy group, an aryloxy group, an alkylthio group, an arylthio group, a sulfoxyl group, a sulfonamide group, a sulfamoyl group, an acylamino group, a ureido group, or the like).

In formula (V), the aromatic group represented by  $A_0$  is preferably an aryl group of a single or condensed ring. For example, a benzene ring or a naphthalene ring is described. As a heterocycle represented by  $A_0$ , the heterocycle of a single or condensed ring containing at least one heteroatom selected from a nitrogen atom, a sulfur atom, or an oxygen atom is preferable. For example, a pyrrolidine ring, an imidazole ring, a tetrahydrofuran ring, a morpholine ring, a pyridine ring, a pyrimidine ring, a quinoline ring, a thiazole ring, a benzothiazole ring, a thiophene ring and a furan ring are described. The aromatic group, heterocyclic group, or  $-G_0-D_0$  group, as  $A_0$ , may have a substituent. As  $A_0$ , an aryl group and a  $-G_0-D_0$  group are particularly preferable.

And, in formula (V),  $A_0$  preferably contains at least one of a diffusion-resistant group or an adsorptive group to silver halide. As a diffusion-resistance group, a ballast group usually used as non-moving photographic additive is preferable.

5 As a ballast group, a photochemically inactive alkyl group, alkenyl group, alkynyl group, alkoxy group, phenyl group, phenoxy group, alkylphenoxy group and the like are described and it is preferred that the substituent part has 8 or more carbon atoms in total.

10 In formula (V), as an adsorption promoting group to silver halide, a thiourea, a thiourethane group, a mercapto group, a thioether group, a thione group, a heterocyclic group, a thiaamido heterocyclic group, a mercapto heterocyclic group, and an adsorptive group described in JP-A No. 64-90439 are described.

15 In formula (V),  $B_0$  represents a blocking group and preferably a  $-G_0-D_0$  group.  $G_0$  represents one selected from a  $-CO-$  group, a  $-COCO-$  group, a  $-CS-$  group, a  $-C(=NG_1D_1)-$  group, an  $-SO-$  group, an  $-SO_2-$  group,

20 or a  $-P(O)(G_1D_1)-$  group. As preferable  $G_0$ , a  $-CO-$  group and a  $-COCO-$  group are described.  $G_1$  represents one selected from a mere bonding hand, an  $-O-$  group, an  $-S-$  group, or an  $-N(D_1)-$  group, and  $D_1$  represents one selected from an aliphatic group, an aromatic group, a heterocyclic group, or a hydrogen atom. In the case where plural  $D_1$ 's exist in a molecule, they may be the same or different.  $D_0$  represents one selected from a hydrogen atom, an aliphatic group, an aromatic group, a heterocyclic group, an amino group, an alkoxy group, an aryloxy group, an alkylthio group, or an arylthio group. As preferable  $D_0$ , a hydrogen atom, an alkyl group, an alkoxy group, an amino group and the like are described.

25  $A_1$  and  $A_2$  both represent a hydrogen atom, or one of  $A_1$  and  $A_2$  represents a hydrogen atom and the other represents one selected from an acyl group (an acetyl group, a trifluoroacetyl group, a benzoyl group or the like), a sulfonyl group (a methanesulfonyl group, a toluenesulfonyl group or the like), or an oxalyl group (an ethoxalyl group or the like).

30 As specific examples of the compound represented by formula (V), the compound H-1 to H-35 of chemical formula Nos. 12 to 18 and the compound H-1-1 to H-4-5 of chemical formula Nos. 20 to 26 in JP-A No. 2002-131864 are described, however specific examples are not limited in these.

35 The compounds represented by formula (V) can be easily synthesized by known methods. For example, these can be synthesized by referring to U.S. Pat. Nos. 5,464,738 and 5,496,695.

40 In addition, hydrazine derivatives preferably used are the compound H-1 to H-29 described in U.S. Pat. No. 5,545,505, columns 11 to 20 and the compounds 1 to 12 described in U.S. Pat. No. 5,464,738, columns 9 to 11. These hydrazine derivatives can be synthesized by known methods.

45 Next, formula (VI) is explained. In formula (VI), although X and R are displayed in a cis form, a trans form for X and R is also included in formula (VI). This is also similar to the structure display of specific compounds.

50 In formula (VI), X represents an electron-attracting group, and W represents one selected from a hydrogen atom, an alkyl group, an alkenyl group, an alkynyl group, an aryl group, a heterocyclic group, a halogen atom, an acyl group, a thioacyl group, an oxalyl group, an oxymoyl group, a thioxoxalyl group,

55 group, an oxamoyl group, an oxycarbonyl group, a thiocarbonyl group, a carbamoyl group, a thiocarbamoyl group, a sulfonyl group, a sulfanyl group, an oxysulfanyl group, a thiosulfanyl group, a sulfamoyl group, an oxysulfamoyl group, a thiosulfamoyl group, a sulfonamoyl group, a phosphoryl group, a nitro group, an imino group, a N-carbonylimino group, a N-sulfonylimino group, a dicyanoethylene group, an ammonium group, and the like.

60

65

nium group, a sulfonium group, a phosphonium group, a pyrylium group, or an immonium group.

R represents one selected from a halogen atom, a hydroxy group, an alkoxy group, an aryloxy group, a heterocyclic oxy group, an alkenyloxy group, an acyloxy group, an alkoxy carbonyloxy group, an aminocarbonyloxy group, a mercapto group, an alkylthio group, an arylthio group, a heterocyclic thio group, an alkenylthio group, an acylthio group, an alkoxy carbonylthio group, an aminocarbonylthio group, an organic or inorganic salt of hydroxy group or mercapto group (e.g., a sodium salt, a potassium salt, a silver salt, or the like), an amino group, an alkylamino group, a cyclic amino group (e.g., a pyrrolidino group), an acylamino group, an oxycarbonylamino group, a heterocyclic group (a 5 or 6-membered nitrogen-containing heterocycle, e.g., a benzotriazolyl group, an imidazolyl group, a triazolyl group, a tetrazolyl group, or the like), a ureido group, or a sulfonamide group. X and W, and X and R may bind to each other to form a cyclic structure. As the ring formed by X and W, for example, pyrazolone, pyrazolidinone, cyclopentanedione,  $\beta$ -ketolactone,  $\beta$ -ketolactam, and the like are described.

Explaining formula (VI) further, the electron-attracting group represented by X is a substituent which can have a positive value of substituent constant  $\sigma$  p. Specifically, a substituted alkyl group (halogen substituted alkyl and the like), a substituted alkenyl group (cyanovinyl and the like), a substituted or unsubstituted alkynyl group (trifluoromethylacetylenyl, cyanoacetylenyl and the like), a substituted aryl group (cyanophenyl and the like), a substituted or unsubstituted heterocyclic group (pyridyl, triazinyl, benzoxazolyl and the like), a halogen atom, a cyano group, an acyl group (acetyl, trifluoroacetyl, formyl and the like), a thioacetyl group (thioacetyl, thioformyl and the like), an oxalyl group (methyloxalyl and the like), an oxyoxalyl group (ethoxalyl and the like), a thioxoalyl group (ethylthioxoalyl and the like), an oxamoyl group (methyloxamoyl and the like), an oxycarbonyl group (ethoxycarbonyl and the like), a carboxyl group, a thiocarbonyl group (ethylthiocarbonyl and the like), a carbamoyl group, a thiocarbamoyl group, a sulfonyl group, a sulfinyl group, an oxysulfonyl group (ethoxysulfonyl and the like), a thiosulfonyl group (ethylthiosulfonyl and the like), a sulfamoyl group, an oxysulfinyl group (methoxysulfinyl and the like), a thiosulfinyl group (methylthiosulfinyl and the like), a sulfonamoyl group, a phosphoryl group, a nitro group, an imino group, a N-carbonylimino group (N-acetyllimino and the like), a N-sulfonylimino group (N-methanesulfonylimino and the like), a dicyanoethylene group, an ammonium group, a sulfonium group, a phosphonium group, a pyrylium group, an immonium group and the like are described, and a heterocyclic one formed by an ammonium group, a sulfonium group, a phosphonium group, an immonium group or the like is also included. The substituent having  $\sigma$  p value of 0.30 or more is particularly preferable.

As an alkyl group represented by W, methyl, ethyl, trifluoromethyl and the like are described. As an alkenyl group as W, vinyl, halogen-substituted vinyl, cyanovinyl and the like are described. As an alkynyl group as W, acetylenyl, cyanoacetylenyl and the like are described. As an aryl group as W, nitrophenyl, cyanophenyl, pentafluorophenyl and the like are described, and as a heterocyclic group as W, pyridyl, pyrimidyl, triazinyl, succinimide, tetrazolyl, triazolyl, imidazolyl, benzoxazolyl and the like are described. As W, the electron-attracting group having a positive  $\sigma$  p value is preferable, and that value is more preferably 0.30 or more.

Among the substituents of R described above, a hydroxy group, a mercapto group, an alkoxy group, an alkylthio group, a halogen atom, an organic or inorganic salt of hydroxy group

or mercapto group, and a heterocyclic group are preferably described. More preferably, a hydroxy group, an alkoxy group, an organic or inorganic salt of hydroxy group or mercapto group and a heterocyclic group are described, and particularly preferably, a hydroxy group and an organic or inorganic salt of hydroxy group or mercapto group are described.

And among the substituents of X and W described above, the group having a thioether bond in the substituent is preferable.

As specific examples of the compound represented by formula (VI), compound 1-1 to 92-7 of chemical formula Nos. 27 to 50 described in JP-A No. 2002-131864 are described, however specific examples are not limited in these.

In formula (P), Q represents a nitrogen atom or a phosphorus atom. R<sub>1</sub>, R<sub>2</sub>, R<sub>3</sub>, and R<sub>4</sub> each independently represent a hydrogen atom or a substituent, and X<sup>-</sup> represents an anion. In addition, R<sub>1</sub> to R<sub>4</sub> may bind to each other to form a cyclic structure.

As the substituent represented by R<sub>1</sub> to R<sub>4</sub>, an alkyl group (a methyl group, an ethyl group, a propyl group, a butyl group, a hexyl group, a cyclohexyl group and the like), an alkenyl group (an allyl group, a butenyl group and the like), an alkynyl group (a propargyl group, a butynyl group and the like), an aryl group (a phenyl group, a naphthyl group and the like), a heterocyclic group (a piperidinyl group, a piperazinyl group, a morpholinyl group, a pyridyl group, a furyl group, a thienyl group, a tetrahydrofuryl group, a tetrahydrothienyl group, a sulforanyl group and the like), an amino group, and the like are described.

As the ring formed by linking R<sub>1</sub> to R<sub>4</sub> each other, a piperidine ring, a morpholine ring, a piperazine ring, a quinuclidine ring, a pyridine ring, a pyrrole ring, an imidazole ring, a triazole ring, a tetrazole ring, and the like are described.

The group represented by R<sub>1</sub> to R<sub>4</sub> may have a substituent such as a hydroxy group, an alkoxy group, an aryloxy group, a carboxyl group, a sulfo group, an alkyl group, an aryl group, and the like. As R<sub>1</sub>, R<sub>2</sub>, R<sub>3</sub>, and R<sub>4</sub>, a hydrogen atom and an alkyl group are preferable.

As the anion represented by X<sup>-</sup>, an organic or inorganic anion such as a halogen ion, a sulfate ion, a nitrate ion, an acetate ion, a p-toluenesulfonate ion, and the like are described.

As a structure of formula (P), the structure described in paragraph Nos. 0153 to 0163 in JP-A No. 2002-131864 is still more preferable.

As the specific compounds of formula (P), P-1 to P-52 and T-1 to T-18 of chemical formula Nos. 53 to 62 in JP-A No. 2002-131864 can be described, however the specific compound is not limited in these.

The quaternary onium compound described above can be synthesized by referring to known methods. For example, the tetrazolium compound described above can be synthesized by referring to the method described in Chemical Reviews, vol. 55, pages 335 to 483.

Next, the compounds represented by formulae (A) or (B) are explained in detail. In formula (A), Z<sub>1</sub> represents a non-metallic atomic group capable to form a 5 to 7-membered cyclic structure with  $—Y_1—C(=CH—X_1)—C(=O)—$ . Z<sub>1</sub> is preferably an atomic group selected from a carbon atom, an oxygen atom, a sulfur atom, a nitrogen atom, or a hydrogen atom, and several atoms selected from these are bound each other by single bond or double bond to form a 5 to 7-membered cyclic structure with  $—Y_1—C(=CH—X_1)—C(=O)—$ . Z<sub>1</sub> may have a substituent, and Z<sub>1</sub> itself may be an aromatic or a non-aromatic carbon ring, or Z<sub>1</sub> may be a part of an aromatic or a non-aromatic heterocycle, and in this case, a

5 to 7-membered cyclic structure formed by  $Z_1$  with  $—Y_1—C(=CH—X_1)—C(=O) —$  forms a condensed cyclic structure.

In formula (B),  $Z_2$  represents a nonmetallic atomic group capable to form a 5 to 7-membered cyclic structure with  $—Y_2—C(=CH—X_2)—C(Y_3)=N—$ .  $Z_2$  is preferably an atomic group selected from a carbon atom, an oxygen atom, a sulfur atom, a nitrogen atom, or a hydrogen atom, and several atoms selected from these are linked each other by single bond or double bond to form a 5 to 7-membered cyclic structure with  $—Y_2—C(=CH—X_2)—C(Y_3)=N—$ .  $Z_2$  may have a substituent, and  $Z_2$  itself may be an aromatic or a non-aromatic carbon ring, or  $Z_2$  may be a part of an aromatic or a non-aromatic heterocycle and in this case, a 5 to 7-membered cyclic structure formed by  $Z_2$  with  $—Y_2—C(=CH—X_2)—C(Y_3)=N—$  forms a condensed cyclic structure.

In the case where  $Z_1$  and  $Z_2$  have a substituent, examples of substituent are selected from the compounds listed below. Namely, as typical substituent, for example, a halogen-atom (fluorine atom, chlorine atom, bromine atom or iodine atom), an alkyl group (includes an aralkyl group, a cycloalkyl group and an active methine group), an alkenyl group, an alkynyl group, an aryl group, a heterocyclic group, a heterocyclic group containing a quaternary nitrogen (e.g., a pyridinio group), an acyl group, an alkoxy carbonyl group, an aryloxy carbonyl group, a carbamoyl group, a carboxyl group or a salt thereof, a sulfonyl carbamoyl group, an acyl carbamoyl group, a sulfamoyl carbamoyl group, a carbazoyl group, an oxazyl group, an oxamoyl group, a cyano group, a thiocarbamoyl group, a hydroxy group, an alkoxy group (including the group in which ethylene oxy group units or propylene oxy group units are repeated), an aryloxy group, a heterocyclic oxy group, an acyloxy group, an alkoxy carbonyloxy group, an aryloxy carbonyloxy group, a carbamoyloxy group, a sulfonyloxy group, an amino group, an alkylamino group, an arylamino group, a heterocyclic amino group, a  $N$ -substituted nitrogen-containing heterocyclic group, an acylamino group, a sulfonamide group, a ureido group, a thioureido group, an imide group, an alkoxy carbonylamino group, an aryloxycarbonylamino group, a sulfamoylamino group, a semicarbazide group, a thiosemicarbazide group, a hydrazino group, a quaternary ammonio group, an oxamoylamino group, an alkylsulfonylureido group, an arylsulfonylureido group, an acylureido group, an acylsulfamoylamino group, a nitro group, a mercapto group, an alkylthio group, an arylthio group, a heterocyclic thio group, an alkylsulfonyl group, an arylsulfonyl group, a sulfo group or a salt thereof, a sulfamoyl group, an acylsulfamoyl group, a sulfonylsulfamoyl group or a salt thereof, a group containing phosphoric amide or phosphoric ester structure, a silyl group, a stannyl group, and the like are described. These substituents may be further substituted by these substituents.

Next,  $Y_3$  is explained. In formula (B),  $Y_3$  represents a hydrogen atom or a substituent, and when  $Y_3$  represents a substituent, following group is specifically described as that substituent. Namely, an alkyl group, an aryl group, a heterocyclic group, a cyano group, an acyl group, an alkoxy carbonyl group, an aryloxycarbonyl group, a carbamoyl group, an amino group, an alkylamino group, an arylamino group, a heterocyclic amino group, an acylamino group, a sulfonamide group, a ureido group, a thioureido group, an imide group, an alkoxy group, an aryloxy group, an alkylthio group, an arylthio group, a heterocyclic thio group, and the like are described. These substituents may be substituted by any substituents, and specifically, examples of the substituents which  $Z_1$  or  $Z_2$  may have, are described.

In formulae (A) and (B),  $X_1$  and  $X_2$  each independently represent one selected from a hydroxy group (or a salt thereof), an alkoxy group (e.g., a methoxy group, an ethoxy group, a propoxy group, an isopropoxy group, an octyloxy group, a dodecyloxy group, a cetylloxy group, a t-butoxy group, or the like), an aryloxy group (e.g., a phenoxy group, a p-t-pentylphenoxy group, a p-t-octylphenoxy group, or the like), a heterocyclic oxy group (e.g., a benzotriazolyl-5-oxy group, a pyridinyl-3-oxy group, or the like), a mercapto group (or a salt thereof), an alkylthio group (e.g., methylthio group, an ethylthio group, a butylthio group, a dodecylthio group, or the like), an arylthio group (e.g., a phenylthio group, a p-dodecylphenylthio group, or the like), a heterocyclic thio group (e.g., a 1-phenyltetrazoyl-5-thio group, a 2-methyl-1-phenyltriazoyl-5-thio group, a mercaptothiadiazolylthio group, or the like), an amino group, an alkylamino group (e.g., a methylamino group, a propylamino group, an octylamino group, a dimethylamino group, or the like), an arylamino group (e.g., an anilino group, a naphthylamino group, an o-methoxyanilino group, or the like), a heterocyclic amino group (e.g., a pyridylamino group, a benzotriazole-5-ylamino group, or the like), an acylamino group (e.g., an acetamide group, an octanoylamino group, a benzoylamino group, or the like), a sulfonamide group (e.g., a methanesulfonamide group, a benzenesulfonamide group, a dodecylsulfonamide group, or the like), or a heterocyclic group.

Herein, a heterocyclic group is an aromatic or non-aromatic, a saturated or unsaturated, a single ring or condensed ring, or a substituted or unsubstituted heterocyclic group. For example, a  $N$ -methylhydantoyl group, a  $N$ -phenylhydantoyl group, a succinimide group, a phthalimide group, a  $N,N'$ -dimethylurazolyl group, an imidazolyl group, a benzotriazolyl group, an indazolyl group, a morpholino group, a 4,4-dimethyl-2,5-dioxo-oxazolyl group, and the like are described.

And herein, a salt represents a salt of an alkali metal (sodium, potassium, or lithium), a salt of an alkali earth metal (magnesium or calcium), a silver salt, a quaternary ammonium salt (a tetraethylammonium salt, a dimethylcetylbenzylammonium salt, or the like), a quaternary phosphonium salt, or the like. In formulae (A) and (B),  $Y_1$  and  $Y_2$  represent  $—C(=O) —$  or  $—SO_2 —$ .

The preferable range of the compounds represented by formulae (A) or (B) is described in JP-A No. 11-231459, paragraph Nos. 0027 to 0043. As specific examples of the compound represented by formulae (A) or (B), compound 1 to 110 of Table 1 to Table 8 in JP-A No. 11-231459 are described, however the invention is not limited in these.

Next, the compound represented by formula (C) is explained in detail. In formula (C),  $X_3$  represents one selected from an oxygen atom, a sulfur atom, or a nitrogen atom. In the case where  $X_3$  is a nitrogen atom, the bond of  $X_3$  and  $Z_3$  may be either a single bond or a double bond, and in the case of a single bond, a nitrogen atom may have a hydrogen atom or any substituent. As this substituent, for example, an alkyl group (includes an aralkyl group, a cycloalkyl group, an active methine group, and the like), an alkenyl group, an alkynyl group, an aryl group, a heterocyclic group, an acyl group, an alkoxy carbonyl group, an aryloxycarbonyl group, a carbamoyl group, an alkylsulfonyl group, an arylsulfonyl group, a heterocyclic sulfonyl group, and the like are described.

$Y_4$  represents the group represented by one selected from  $—C(=O) —$ ,  $—C(=S) —$ ,  $—SO —$ ,  $—SO_2 —$ ,  $—C(=NR_3) —$ , or  $—(R_4)C=N —$ .  $Z_3$  represents a nonmetallic atomic group capable to form a 5 to 7-membered ring containing  $X_3$  and  $Y_4$ . The atomic group to form that ring is an

atomic group which consists of 2 to 4 atoms that are other than metal atoms, and these atoms may be combined by single bond or double bond, and these may have a hydrogen atom or any substituent (e.g., an alkyl group, an aryl group, a heterocyclic group, an alkoxy group, an alkylthio group, an acyl group, an amino group, or an alkenyl group). When  $Z_3$  forms a 5 to 7-membered ring containing  $X_3$  and  $Y_4$ , the ring is a saturated or unsaturated heterocycle, and may be a single ring or may have a condensed ring. When  $Y_4$  is the group represented by  $C(=NR_3)$ ,  $(R_4)C=N$ , the condensed ring of this case may be formed by binding  $R_3$  or  $R_4$  with the substituent of  $Z_3$ .

In formula (C),  $R_1$ ,  $R_2$ ,  $R_3$ , and  $R_4$  each independently represent a hydrogen atom or a substituent. However,  $R_1$  and  $R_2$  never bind to each other to form a cyclic structure.

When  $R_1$  and  $R_2$  represent a monovalent substituent, the following groups are described as a monovalent substituent.

For example, a halogen atom (fluorine atom, chlorine atom, bromine atom, or iodine atom), an alkyl group (including an aralkyl group, a cycloalkyl group, an active methine group, and the like), an alkenyl group, an alkynyl group, an aryl group, a heterocyclic group, a heterocyclic group containing a quaternary nitrogen atom (e.g., a pyridinio group), an acyl group, an alkoxy carbonyl group, an aryloxycarbonyl group, a carbamoyl group, a carbonyl group and a salt thereof, a sulfonyl carbamoyl group, an acyl carbamoyl group, a sulfamoyl carbamoyl group, a carbazoyl group, an oxazoyl group, an oxamoyl group, a cyano group, a thiocarbamoyl group, a hydroxy group and a salt thereof, an alkoxy group (including the group in which ethylene oxy group units or propylene oxy group units are repeated), an aryloxy group, a heterocyclic oxy group, an acyloxy group, an alkoxy carbonyloxy group, an aryloxycarbonyloxy group, a carbamoyloxy group, a sulfonyloxy group, an amino group, an alkylamino group, an arylamino group, an heterocyclic amino group, a N-substituted nitrogen-containing heterocyclic group, an acylamino group, a sulfonamide group, a ureido group, a thioureido group, an imide group, an alkoxy carbonylamino group, an aryloxycarbonylamino group, a sulfamoylamino group, a semicarbazide group, a thiosemicarbazide group, a hydrazino group, a quaternary ammonium group, an oxamoylamino group, an alkylsulfonylureido group, an arylsulfonylureido group, an acylureido group, an acylsulfamoylamino group, a nitro group, a mercapto group and a salt thereof, an alkylthio group, an arylthio group, an heterocyclic thio group, an alkylsulfonyl group, an arylsulfonyl group, an alkylsulfinyl group, an arylsulfinyl group, a sulfo group and a salt thereof, a sulfamoyl group, an acylsulfamoyl group, a sulfonylsulfamoyl group and a salt thereof, a phosphoryl group, a group containing phosphoric amide or phosphoric ester structure, a silyl group, a stannyl group, and the like are described. These substituents may be further substituted by these monovalent substituents.

When  $R_3$  and  $R_4$  represent a substituent, the same substituent as what  $R_1$  and  $R_2$  may have except the halogen atom can be described as the substituent. Furthermore,  $R_3$  and  $R_4$  may further link to  $Z_3$  to form a condensed ring.

Next, among the compounds represented by formula (C), preferable compounds are described. In formula (C),  $Z_3$  preferably is an atomic group which forms a 5 to 7-membered ring with  $X_3$  and  $Y_4$ , and consists of the atoms selected from 2 to 4 carbon atoms, a nitrogen atom, a sulfur atom, or an oxygen atom. A heterocycle, which is formed by  $Z_3$  with  $X_3$  and  $Y_4$ , preferably contains 3 to 40 carbon atoms in total, more preferably 3 to 25 carbon atoms in total, and most preferably 3 to 20 carbon atoms in total.  $Z_3$  preferably comprises at least one carbon atom.

In formula (C),  $Y_4$  is preferably  $-C(=O)-$ ,  $-C(=S)-$ ,  $-SO_2-$ , or  $-(R_4)C=N-$ , particularly preferably,  $-C(=O)-$ ,  $-C(=S)-$ , or  $-SO_2-$ , and most preferably,  $-C(=O)-$ .

In formula (C), in the case where  $R_1$  and  $R_2$  represent a monovalent substituent, the monovalent substituent represented by  $R_1$  and  $R_2$  is preferably one of the following groups having 0 to 25 carbon atoms in total, namely, those are an alkyl group, an aryl group, a heterocyclic group, an alkoxy group, an aryloxy group, a heterocyclic oxy group, an alkylthio group, an arylthio group, a heterocyclic thio group, an amino group, an alkylamino group, an arylamino group, a heterocyclic amino group, a ureido group, an imide group, an acylamino group, a hydroxy group and a salt thereof, a mercapto group and a salt thereof, and an electron-attracting group. Herein, an electron-attracting group means the substituent capable to have a positive value of Hammett substituent constant  $\sigma_p$ , and specifically a cyano group, a sulfamoyl group, an alkylsulfonyl group, an arylsulfonyl group, a sulfonyamide group, an imino group, a nitro group, a halogen atom, an acyl group, a formyl group, a phosphoryl group, a carboxyl group (or a salt thereof), a sulfo group (or a salt thereof), a saturated or unsaturated heterocyclic group, an alkenyl group, an alkynyl group, an acyloxy group, an acylthio group, a sulfonyloxy group, and an aryl group substituted by these electron-attracting group are described. These substituents may have any substituents.

In formula (C), when  $R_1$  and  $R_2$  represent a monovalent substituent, more preferable are an alkoxy group, an aryloxy group, a heterocyclic oxy group, an alkylthio group, an arylthio group, a heterocyclic thio group, an amino group, an alkylamino group, an arylamino group, a heterocyclic amino group, a ureido group, an imide group, an acylamino group, a sulfonamide group, a heterocyclic group, a hydroxy group or a salt thereof, a mercapto group or a salt thereof, and the like. In formula (C),  $R_1$  and  $R_2$  particularly preferably are a hydrogen atom, an alkoxy group, an aryloxy group, an alkylthio group, an arylthio group, a heterocyclic group, a hydroxy group or a salt thereof, a mercapto group or a salt thereof, or the like. In formula (C), most preferably, one of  $R_1$  and  $R_2$  is a hydrogen atom and another is an alkoxy group, an aryloxy group, an alkylthio group, an arylthio group, a heterocyclic group, a hydroxy group or a salt thereof, or a mercapto group or a salt thereof.

In formula (C), when  $R_3$  represents a substituent,  $R_3$  is preferably an alkyl group having 1 to 25 carbon atoms in total (including an aralkyl group, a cycloalkyl group, an active methine group and the like), an alkenyl group, aryl group, a heterocyclic group, a heterocyclic group containing a quaternary nitrogen (e.g., a pyridinio group), an acyl group, an alkoxy carbonyl group, an aryloxycarbonyl group, a carbamoyl group, an alkylsulfonyl group, an arylsulfonyl group, an alkylsulfinyl group, an arylsulfinyl group, a sulfosulfamoyl group, an alkoxy group, an aryloxy group, a heterocyclic oxy group, an alkylthio group, an arylthio group, a heterocyclic thio group, an amino group, or the like. An alkyl group and an aryl group are particularly preferable.

In formula (C), when  $R_4$  represents a substituent,  $R_4$  is preferably an alkyl group (including an aralkyl group, a cycloalkyl group, an active methine group, and the like) having 1 to 25 carbon atoms in total, an aryl group, a heterocyclic group, a heterocyclic group containing a quaternary nitrogen atom (e.g., a pyridinio group), an acyl group, an alkoxy carbonyl group, an aryloxycarbonyl group, a carbamoyl group, an alkylsulfonyl group, an arylsulfonyl group, an alkylsulfinyl group, an arylsulfinyl group, a sulfosulfamoyl group, an alkoxy group, an aryloxy group, a heterocyclic oxy group, an alkylthio group, an arylthio group, a heterocyclic thio group, an amino group, or the like. An alkyl group and an aryl group are particularly preferable.

55

alkylthio group, an arylthio group, a heterocyclic thio group, or the like. Particularly preferably, an alkyl group, an aryl group, an alkoxy group, an aryloxy group, a heterocyclic oxy group, an alkylthio group, an arylthio group, a heterocyclic thio group, and the like are described.

Specific compounds represented by formula (C) are represented by A-1 to A-230 of chemical formula Nos. 6 to 18 described in JP-A No. 11-133546, however the invention is not limited in these.

The addition amount of the above nucleator is in a range of from  $10^{-5}$  mol to 1 mol per 1 mol of organic silver salt, and preferably, in a range of from  $10^{-4}$  mol to  $5 \times 10^{-1}$  mol.

The nucleator described above may be incorporated into a photothermographic material by being added into the coating solution, such as in the form of a solution, an emulsion dispersion, a solid fine particle dispersion, or the like.

As well known emulsion dispersing method, there can be mentioned a method comprising dissolving the nucleator in an oil such as dibutylphthalate, tricresylphosphate, dioctylsebacate, tri(2-ethylhexyl)phosphate, or the like, using an auxiliary solvent such as ethyl acetate, cyclohexanone, or the like, and then adding a surfactant such as sodium dodecylbenzenesulfonate, sodium oleoil-N-methyltaurinate, sodium di(2-ethylhexyl)sulfosuccinate or the like; from which an emulsion dispersion is mechanically produced. During the process, for the purpose of controlling viscosity of oil droplet and refractive index, the addition of polymer such as  $\alpha$ -methylstyrene oligomer, poly(t-butylacrylamide), or the like is preferable.

As solid particle dispersing method, there can be mentioned a method comprising dispersing the powder of the nucleator in a proper solvent such as water or the like, by means of ball mill, colloid mill, vibrating ball mill, sand mill, jet mill, roller mill, or ultrasonics, thereby obtaining solid dispersion. In this case, there can also be used a protective colloid (such as poly(vinyl alcohol)), or a surfactant (for instance, an anionic surfactant such as sodium triisopropyl-naphthalenesulfonate (a mixture of compounds having the three isopropyl groups in different substitution sites)). In the mills enumerated above, generally used as the dispersion media are beads made of zirconia and the like, and Zr and the like eluting from the beads may be incorporated in the dispersion. Although depending on the dispersing conditions, the amount of Zr and the like generally incorporated in the dispersion is in a range of from 1 ppm to 1000 ppm. It is practically acceptable so long as Zr is incorporated in an amount of 0.5 mg or less per 1 g of silver.

Preferably, an antiseptic (for instance, benzothiazolinone sodium salt) is added in the water dispersion.

The nucleator is particularly preferably used as solid particle dispersion, and is added in the form of fine particles having average particle size of from 0.01  $\mu$ m to 10  $\mu$ m, preferably from 0.05  $\mu$ m to 5  $\mu$ m and, more preferably from 0.1  $\mu$ m to 2  $\mu$ m. In the invention, other solid dispersions are preferably used with this particle size range.

In the photothermographic material which is subjected to a rapid development where time period for development is 20 seconds or less, the compound represented by formulae (V) or (P) is used preferably, and the compound represented by formula (V) is used particularly preferably, among the nucleators described above.

In the photothermographic material where low fog is required, the compound represented by formula (VI) is used preferably, the compound represented by formulae (A), (B), or (C) is used more preferably, and particularly preferably the compound represented by formulae (A) or (B) is particularly preferably used. Moreover, in the photothermographic mate-

56

rials having a few change of photographic property against environmental conditions when used on various environmental conditions (temperature and humidity), the compound represented by formula (C) is preferably used.

Although preferred specific compounds among the above-mentioned nucleators are shown below, the invention is not limited in these.



SH-1



SH-2



SH-3



SH-4



SH-5



SH-6



SH-7

-continued



The nucleator of the present invention can be added to the image forming layer or the layer adjacent to the image forming layer, however, it is preferably added to the image forming layer. The addition amount of nucleator is in a range of from  $10^{-5}$  mol to 1 mol per 1 mol of organic silver salt, and preferably, from  $10^{-4}$  mol to  $5 \times 10^{-1}$  mol. The nucleator may be added either only one kind or, two or more kinds in combination.

The photothermographic material of the present invention may have two or more image forming layers including photosensitive silver halide. In the case of two or more layers, any one of the image forming layers may contain the nucleator. Preferably, the photothermographic material of the present invention has at least two image forming layers, and one of the image forming layers contains the nucleator and the other image forming layer does not contain the nucleator.

(Reducing Agent)

1) Infectious Development Reducing Agent

The photothermographic material according to the invention preferably contains an infectious development reducing agent. As the infectious development reducing agent used in the present invention, any reducing agent may be used as far as it has the ability of infectious development.

Preferable infectious development reducing agent which can be used in the present invention is the compound represented by the following formula (R1).



SH-10

25

In formula (R1) described above, R<sup>11</sup> and R<sup>11'</sup> each independently represent a secondary or tertiary alkyl group having 3 to 20 carbon atoms. R<sup>12</sup> and R<sup>12'</sup> each independently represent a hydrogen atom or a group which links through a nitrogen, an oxygen, a phosphor, or a sulfur atom. R<sup>13</sup> represents a hydrogen atom or an alkyl group having 1 to 20 carbon atoms.

30 Formula (R1) described above is explained in detail. As R<sup>11</sup> and R<sup>11'</sup> described above, a secondary or tertiary alkyl group having 3 to 12 carbon atoms is preferable. Specifically, an isopropyl group, a tert-butyl group, a tert-amyl group, a 1,1-dimethylpropyl group, a 1,1-dimethylbutyl group, a 1,1-dimethylhexyl group, a 1,1-3,3-tetramethylbutyl group, a 35 1,1-dimethyldecyl group, a 1-methylcyclohexyl group, a tert-octyl group, a 1-methylcyclopropyl group and the like are preferable, and a tert-butyl group, a tert-amyl group, a tert-octyl group and a 1-methylcyclohexyl group are more preferable, and a tert-butyl group is most preferable.

SH-11

40

45

In the case where R<sup>12</sup> and R<sup>12'</sup> are an aryloxy group, an arylthio group, an anilino group, a heterocyclic group, or a heterocyclic thio group, each of which may have a substituent. As the said substituent, although any group may be possible as far as it is capable of substituting for a hydrogen atom on a benzene ring and a heterocycle, and, an alkyl group, an aryl group, a heterocyclic group, a halogen atom, an alkoxy group, a hydroxy group, an aryloxy group, an alkylthio group, an arylthio group, an amino group, an acyl group, an acyloxy group, an acylamino group, an alkoxy carbonyl group, a carbamoyl group, a sulfonyl group, a sulfonamide group, a sulfonyloxy group, a sulfamoyl group, a sulfoxido group, an ureido group or an urethane group or the like are described.

50

55

55

In the case where R<sup>12</sup> and R<sup>12'</sup> are an alkoxy group, a carbonyloxy group, an acyloxy group, an alkylthio group, an amino group, an acylamino group, an ureido group or an urethane group, these groups may further have a substituent and as examples of the said substituent, an alkoxy group, an alkoxy carbonyl group, an acyloxy group, an sulfonyl group, a carbonyl group, an alkylthio group, an aryloxy group, an arylthio group, a sulfonamide group, an acylamino group, and the like are described.

60

65

As R<sup>12</sup> and R<sup>12'</sup> described above, a hydrogen atom, a hydroxy group, an amino group, and an anilino group are more preferable, and further, a hydrogen atom, a methoxy group, and a benzyloxy group are most preferable.

As R<sup>13</sup> described above, a hydrogen atom and an alkyl group having 1 to 15 carbon atoms are preferable, and an alkyl

59

group having 1 to 8 carbon atoms is more preferable. As the said alkyl group, a methyl group, an ethyl group, a propyl group, an isopropyl group, and a 2,4,4-trimethylpentyl group are preferable. As R<sup>13</sup> described above, a hydrogen atom, a methyl group, an ethyl group, a propyl group, and an isopropyl group are particularly preferable.

Typical examples of the reducing agent represented by formula (R1) of the present invention are shown below, however the present invention is not limited in these.



US 7,455,960 B2

60

-continued



**61**

-continued

**62**

-continued

R1-14

5



R1-15 15

20



R1-16 30

35



R1-17

45



R1-18

55



R1-19

R1-20

R1-21

R1-22

R1-23

**63**

-continued



R1-24

5

10

15

**64**

-continued

R1-28



R1-25

20

25

30

R1-29



R1-26

35

40

45

R1-30



R1-27

50

55

60

R1-31



65



66



20 The addition amount of the reducing agent represented by the above-described formula (R1) is preferably from 0.01 g/m<sup>2</sup> to 5.0 g/m<sup>2</sup>, and more preferably from 0.1 g/m<sup>2</sup> to 3.0 g/m<sup>2</sup>. It is preferably contained in a range from 5 mol % to 50 mol % and, more preferably, 10 mol % to 40 mol %, per 1 mol of silver in the image forming layer.

25 The reducing agent represented by the above-described formula (R1) is preferably contained in the image forming layer. In particular, the reducing agent represented by the above-described formula (R1) is preferably contained in the 30 image forming layer comprising a silver halide emulsion with low sensitivity.

## 2) Other Reducing Agents

35 In the invention, a reducing agent which has not infectious development properties can be used. The reducing agent which has not infectious development properties may be used alone or in combination with the above-described infectious development reducing agent. More preferably, the reducing agent which has not infectious development properties is used 40 with a nucleator.

45 The reducing agent can be any substance (preferably, organic substance) capable of reducing silver ions into metallic silver. Examples of the reducing agent are described in JP-A No. 11-65021 (column Nos. 0043 to 0045) and EP No. 0803764 (p. 7, line 34 to p. 18, line 12).

50 The reducing agent preferably used in the invention is a so-called hindered phenolic reducing agent or a bisphenol agent having a substituent at the ortho-position to the phenolic hydroxy group. It is more preferably a reducing agent represented by the following formula (R).



In formula (R), R<sup>11</sup> and R<sup>11'</sup> each independently represent an alkyl group having 1 to 20 carbon atoms. R<sup>12</sup> and R<sup>12'</sup> each

independently represent a hydrogen atom or a group capable of substituting for a hydrogen atom on a benzene ring. L represents an —S— group or a —CHR<sup>13</sup>— group. R<sup>13</sup> represents a hydrogen atom or an alkyl group having 1 to 20 carbon atoms. X<sup>1</sup> and X<sup>1'</sup> each independently represent a hydrogen atom or a group capable of substituting for a hydrogen atom on a benzene ring.

Formula (R) is to be described in detail.

In the following description, when referred to as an alkyl group, it means that the alkyl group contains a cycloalkyl group, as far as it is not mentioned specifically.

(1) R<sup>11</sup> and R<sup>11'</sup>

R<sup>11</sup> and R<sup>11'</sup> each independently represent a substituted or unsubstituted alkyl group having 1 to 20 carbon atoms. The substituent for the alkyl group has no particular restriction and can include, preferably, an aryl group, a hydroxy group, an alkoxy group, an aryloxy group, an alkylthio group, an arylthio group, an acylamino group, a sulfonamide group, a sulfonyl group, a phosphoryl group, an acyl group, a carbamoyl group, an ester group, a ureido group, a urethane group, a halogen atom, and the like.

(2) R<sup>12</sup> and R<sup>12'</sup>, X<sup>1</sup> and X<sup>1'</sup>

R<sup>12</sup> and R<sup>12'</sup> each independently represent a hydrogen atom or a group capable of substituting for a hydrogen atom on a benzene ring. X<sup>1</sup> and X<sup>1'</sup> each independently represent a hydrogen atom or a group capable of substituting for a hydrogen atom on a benzene ring. As each of the groups capable of substituting for a hydrogen atom on the benzene ring, an alkyl group, an aryl group, a halogen atom, an alkoxy group, and an acylamino group are described preferably.

(3) L

L represents an —S— group or a —CHR<sup>13</sup>— group. R<sup>13</sup> represents a hydrogen atom or an alkyl group having 1 to 20 carbon atoms in which the alkyl group may have a substituent.

Specific examples of the unsubstituted alkyl group for R<sup>13</sup> can include, for example, a methyl group, an ethyl group, a propyl group, a butyl group, a heptyl group, an undecyl group, an isopropyl group, a 1-ethylpentyl group, a 2,4,4-trimethylpentyl group, cyclohexyl group, 2,4-dimethyl-3-cyclohexenyl group, 3,5-dimethyl-3-cyclohexenyl group, and the like. Examples of the substituent for the alkyl group can include, similar to the substituent of R<sup>11</sup>, a halogen atom, an alkoxy group, an alkylthio group, an aryloxy group, an arylthio group, an acylamino group, a sulfonamide group, a sulfonyl group, a phosphoryl group, an oxycarbonyl group, a carbamoyl group, a sulfamoyl group, and the like.

(4) Preferred Substituents

R<sup>11</sup> and R<sup>11'</sup> are preferably a primary, secondary or tertiary alkyl group having 1 to 15 carbon atoms and can include, specifically, a methyl group, an isopropyl group, a t-butyl group, a t-amyl group, a t-octyl group, a cyclohexyl group, a cyclopentyl group, a 1-methylcyclohexyl group, a 1-methylcyclopropyl group, and the like. R<sup>11</sup> and R<sup>11'</sup> each represent, more preferably, an alkyl group having 1 to 8 carbon atoms and, among them, a methyl group, a t-butyl group, a t-amyl group, and a 1-methylcyclohexyl group are further preferred and, a methyl group and a t-butyl group being most preferred.

R<sup>12</sup> and R<sup>12'</sup> are preferably an alkyl group having 1 to 20 carbon atoms and can include, specifically, a methyl group, an ethyl group, a propyl group, a butyl group, an isopropyl group, a t-butyl group, a t-amyl group, a cyclohexyl group, a 1-methylcyclohexyl group, a benzyl group, a methoxymethyl group, a methoxyethyl group, and the like. More preferred are a methyl group, an ethyl group, a propyl group, an isopropyl group, and a t-butyl group, and particularly preferred are a methyl group and an ethyl group.

X<sup>1</sup> and X<sup>1'</sup> are preferably a hydrogen atom, a halogen atom, or an alkyl group, and more preferably a hydrogen atom.

L is preferably a —CHR<sup>13</sup>— group.

R<sup>13</sup> is preferably a hydrogen atom or an alkyl group having 1 to 15 carbon atoms. The alkyl group is preferably a chain or a cyclic alkyl group. And, a group which has a C=C bond in these alkyl group is also preferably used. Preferable examples of the alkyl group can include a methyl group, an ethyl group, a propyl group, an isopropyl group, a 2,4,4-trimethylpentyl group, a cyclohexyl group, a 2,4-dimethyl-3-cyclohexenyl group, a 3,5-dimethyl-3-cyclohexenyl group and the like. Particularly preferable R<sup>13</sup> is a hydrogen atom, a methyl group, an ethyl group, a propyl group, an isopropyl group, or a 2,4-dimethyl-3-cyclohexenyl group.

In the case where R<sup>11</sup> and R<sup>11'</sup> are a tertiary alkyl group and R<sup>12</sup> and R<sup>12'</sup> are a methyl group, R<sup>13</sup> preferably is a primary or secondary alkyl group having 1 to 8 carbon atoms (a methyl group, an ethyl group, a propyl group, an isopropyl group, a 2,4-dimethyl-3-cyclohexenyl group, or the like).

In the case where R<sup>11</sup> and R<sup>11'</sup> are tertiary alkyl group and R<sup>12</sup> and R<sup>12'</sup> are an alkyl group other than a methyl group, R<sup>13</sup> preferably is a hydrogen atom.

In the case where R<sup>11</sup> and R<sup>11'</sup> are not a tertiary alkyl group, R<sup>13</sup> preferably is a hydrogen atom or a secondary alkyl group, and particularly preferably a secondary alkyl group. As the secondary alkyl group for R<sup>13</sup>, an isopropyl group and a 2,4-dimethyl-3-cyclohexenyl group are preferred.

The reducing agent described above shows different thermal development performances, color tones of developed silver images, or the like depending on the combination of R<sup>11</sup>, R<sup>11'</sup>, R<sup>12</sup>, R<sup>12'</sup>, and R<sup>13</sup>. Since these performances can be controlled by using two or more kinds of reducing agents at various mixing ratios, it is preferred to use two or more kinds of reducing agents in combination depending on the purpose.

Specific examples of the reducing agents of the invention including the compounds represented by formula (R) according to the invention are shown below, but the invention is not restricted to these.

R-1



R-2



**69**

-continued

**70**

-continued



-continued



As preferred reducing agents of the invention other than those above, there can be mentioned compounds disclosed in JP-A Nos. 2001-188314, 2001-209145, 2001-350235, and 2002-156727, and EP No. 1278101A2.

The reducing agent is preferably contained in the image forming layer comprising a silver halide emulsion with high sensitivity.

The addition amount of the reducing agent is preferably from 0.1 g/m<sup>2</sup> to 3.0 g/m<sup>2</sup>, more preferably from 0.2 g/m<sup>2</sup> to 2.0 g/m<sup>2</sup> and, even more preferably from 0.3 g/m<sup>2</sup> to 1.0 g/m<sup>2</sup>. It is preferably contained in a range of from 5 mol % to 50 mol %, more preferably from 8 mol % to 30 mol % and, even more preferably from 10 mol % to 20 mol %, per 1 mol of silver in the image forming layer.

In the case where plural reducing agents are used in combination, the ratio of combination by mole is from 1/99 to 99/1, and preferably from 5/95 to 95/5.

### 3) Adding Method of Reducing Agent

In the invention, the reducing agent may be incorporated into a photothermographic material by being added into the coating solution, such as in the form of a solution, an emulsion dispersion, a solid fine particle dispersion, or the like.

As well known emulsion dispersing method, there can be mentioned a method comprising dissolving the reducing agent in an oil such as dibutylphthalate, tricresylphosphate, dioctylsebacate, tri(2-ethylhexyl)phosphate, or the like, using an auxiliary solvent such as ethyl acetate, cyclohexanone, or the like, and then adding a surfactant such as sodium

R-16

R-17

R-18

dodecylbenzenesulfonate, sodium oleoil-N-methyltaurinate, sodium di(2-ethylhexyl)sulfosuccinate or the like; from which an emulsion dispersion is mechanically produced. During the process, for the purpose of controlling viscosity of oil droplet and refractive index, the addition of polymer such as  $\alpha$ -methylstyrene oligomer, poly(t-butylacrylamide), or the like is preferable.

As solid particle dispersing method, there can be mentioned a method comprising dispersing the powder of the reducing agent in a proper solvent such as water or the like, by means of ball mill, colloid mill, vibrating ball mill, sand mill, jet mill, roller mill, or ultrasonics, thereby obtaining solid dispersion. In this case, there can also be used a protective colloid (such as poly(vinyl alcohol)), or a surfactant (for instance, an anionic surfactant such as sodium triisopropyl-naphthalenesulfonate (a mixture of compounds having the three isopropyl groups in different substitution sites)). In the mills enumerated above, generally used as the dispersion media are beads made of zirconia and the like, and Zr and the like eluting from the beads may be incorporated in the dispersion. Although depending on the dispersing conditions, the amount of Zr and the like generally incorporated in the dispersion is in a range of from 1 ppm to 1000 ppm. It is practically acceptable so long as Zr is incorporated in an amount of 0.5 mg or less per 1 g of silver.

Preferably, an antiseptic (for instance, benzisothiazolinone sodium salt) is added in the water dispersion.

The reducing agent is particularly preferably used as solid particle dispersion, and is added in the form of fine particles having average particle size of from 0.01  $\mu$ m to 10  $\mu$ m, preferably from 0.05  $\mu$ m to 5  $\mu$ m and, more preferably from 0.1  $\mu$ m to 2  $\mu$ m. In the invention, other solid dispersions are preferably used with this particle size range.

### (Phthalic Acid and Derivatives Thereof)

In the present invention, the photothermographic material preferably comprises the compound selected from phthalic acid or derivatives thereof, in combination with the silver iodide complex-forming agent. As phthalic acid and derivatives thereof used in the present invention, the compound represented by the following formula (PH) is preferable.

45



Formula (PH)

50

wherein T represents one selected from a halogen atom (fluorine, bromine, or iodine atom), an alkyl group, an aryl group, an alkoxy group, or a nitro group; k represents an integer of 0 to 4, and when k is 2 or more, plural ks may be the same or different from each other. k is preferably 0 to 2, and more preferably, 0 or 1.

The compound represented by formula (PH) may be used just as an acid or may be used as suitable salt from the viewpoint of easy addition to a coating solution and from the viewpoint of pH adjustment. As a salt, an alkaline metal salt, an ammonium salt, an alkaline earth metals salt, an amine salt, or the like can be used. An alkaline metal salt (Li, Na, K, or the like) and an ammonium salt are preferred.

Phthalic acid and the derivatives thereof used in the present invention are described below, however the present invention is not limited in these compounds.



-continued



In the invention, the addition amount of phthalic acid or a derivative thereof is from  $1.0 \times 10^{-4}$  mol to 1 mol, preferably from  $1.0 \times 10^{-3}$  mol to 0.5 mol and, even more preferably from  $2.0 \times 10^{-3}$  mol to 0.2 mol, per 1 mol of coated silver.

(4) (Development Accelerator)

In the photothermographic material of the invention, sulfonamidophenolic compounds described in the specification of JP-A No. 2000-267222, and represented by formula (A) described in the specification of JP-A No. 2000-330234; hindered phenolic compounds represented by formula (II) described in JP-A No. 2001-92075; hydrazine compounds described in the specification of JP-A No. 10-62895, represented by formula (I) described in the specification of JP-A No. 11-15116, represented by formula (D) described in the specification of JP-A No. 2002-156727, and represented by

(5) 25 formula (1) described in the specification of JP-A No. 2002-278017; and phenolic or naphtholic compounds represented by formula (2) described in the specification of JP-A No. 2001-264929 are used preferably as a development acceler-

(6) 30 ator.  
 (7) 35 The development accelerator described above is used in a range from 0.1 mol % to 20 mol %, preferably, in a range from 0.5 mol % to 10 mol % and, more preferably, in a range from 1 mol % to 5 mol % with respect to the reducing agent. The introducing methods to the photothermographic material can include similar methods as those for the reducing agent and, it is particularly preferred to add as a solid dispersion or an emulsion dispersion.

(8) 40 In the case of adding as an emulsion dispersion, it is preferred to add as an emulsion dispersion dispersed by using a high boiling solvent which is solid at a normal temperature and an auxiliary solvent at a low boiling point, or to add as a so-called oilless emulsion dispersion not using the high boiling solvent.

(9) 45 In the present invention, among the development accelerators described above, it is particularly preferred to use hydrazine compounds represented by formula (1) described in JP-A No. 2002-278017, and phenolic or naphtholic compounds represented by formula (2) described in JP-A No. 2001-264929.

(10) 50 Preferred specific examples for the development accelerator of the invention are to be described below. The invention is not restricted to them.



-continued



A-2

5

10



(9)

NC1=CC=C(C=C1N2NHC(=O)Nc3ccc(Cl)cc3)S(=O)(=O)C2

8 3 15

20



(10)

Oc1ccccc1S(=O)(=O)c2ccccc2NHCOC4H9(t)Cl

A-4

25



CC(Cc1ccc(cc1)OCCNCCNc2ncsc2)C1=CC=CC=C1

A-5



A-6

40



A-7



60

60



### Formula (D)

In formula (D),  $R^{21}$  to  $R^{23}$  each independently represent one selected from an alkyl group, an aryl group, an alkoxy group, an aryloxy group, an amino group, or a heterocyclic group, which may be substituted or unsubstituted.

65 In the case where  $R^{21}$  to  $R^{23}$  have a substituent, examples of the substituent include a halogen atom, an alkyl group, an aryl

group, an alkoxy group, an amino group, an acyl group, an acylamino group, an alkylthio group, an arylthio group, a sulfonamide group, an acyloxy group, an oxycarbonyl group, a carbamoyl group, a sulfamoyl group, a sulfonyl group, a phosphoryl group, and the like, in which preferred as the substituents are an alkyl group or an aryl group, e.g., a methyl group, an ethyl group, an isopropyl group, a t-butyl group, a t-octyl group, a phenyl group, a 4-alkoxyphenyl group, a 4-acyloxyphenyl group, and the like.

Specific examples of an alkyl group expressed by R<sup>21</sup> to R<sup>23</sup> include a methyl group, an ethyl group, a butyl group, an octyl group, a dodecyl group, an isopropyl group, a t-butyl group, a t-amyl group, a t-octyl group, a cyclohexyl group, a 1-methylecyclohexyl group, a benzyl group, a phenetyl group, a 2-phenoxypropyl group, and the like.

As an aryl group, there can be mentioned a phenyl group, a cresyl group, a xylyl group, a naphthyl group, a 4-t-butylphenyl group, a 4-t-octylphenyl group, a 4-anisidyl group, a 3,5-dichlorophenyl group, and the like.

As an alkoxy group, there can be mentioned a methoxy group, an ethoxy group, a butoxy group, an octyloxy group, a 2-ethylhexyloxy group, a 3,5,5-trimethylhexyloxy group, a dodecyloxy group, a cyclohexyloxy group, a 4-methylcyclohexyloxy group, a benzylxy group, and the like.

As an aryloxy group, there can be mentioned a phenoxy group, a cresyloxy group, an isopropylphenoxy group, a 4-t-butylphenoxy group, a naphthoxy group, a biphenyloxy group, and the like.

As an amino group, there can be mentioned a dimethylamino group, a diethylamino group, a dibutylamino group, a diocetylamino group, an N-methyl-N-hexylamino group, a dicyclohexylamino group, a diphenylamino group, an N-methyl-N-phenylamino, and the like.

Preferred as R<sup>21</sup> to R<sup>23</sup> are an alkyl group, an aryl group, an alkoxy group, and an aryloxy group. Concerning the effect of the invention, it is preferred that at least one or more of R<sup>21</sup> to R<sup>23</sup> are an alkyl group or an aryl group, and more preferably, two or more of them are an alkyl group or an aryl group. From the viewpoint of low cost availability, it is preferred that R<sup>21</sup> to R<sup>23</sup> are of the same group.

Specific examples of hydrogen bonding compounds represented by formula (D) of the invention and others are shown below, but it should be understood that the invention is not limited thereto.



79

-continued



80

-continued



D-13      Specific examples of hydrogen bonding compounds other than those enumerated above can be found in those described in JP-A Nos. 2001-281793 and 2002-14438.

D-14      The hydrogen bonding compound of the invention can be used in the photothermographic material by being incorporated into a coating solution in the form of solution, emulsion dispersion, or solid fine particle dispersion, similar to the case of the reducing agent. In the solution, the hydrogen bonding compound of the invention forms a hydrogen-bonded complex with a compound having a phenolic hydroxy group, and can be isolated as a complex in crystalline state depending on the combination of the reducing agent and the compound expressed by formula (D).

D-15      It is particularly preferred to use the crystal powder thus isolated in the form of a solid fine particle dispersion, because it provides stable performance. Further, it is also preferred to use a method of leading to form complex during dispersion by mixing the reducing agent and the hydrogen bonding compound of the invention in the form of powders and dispersing them with a proper dispersing agent using a sand grinder mill or the like.

The hydrogen bonding compound of the invention is preferably used in a range of from 1 mol % to 200 mol %, more

## 81

preferably from 10 mol % to 150 mol %, and further preferably, from 30 mol % to 100 mol %, with respect to the reducing agent.

## (Binder)

Any kind of polymer may be used as the binder for the image forming layer of the invention. Suitable as the binder are those that are transparent or translucent, and that are generally colorless, such as natural resin or polymer and their copolymers; synthetic resin or polymer and their copolymer; or media forming a film; for example, included are gelatin, rubber, poly(vinyl alcohol), hydroxyethyl cellulose, cellulose acetate, cellulose acetate butyrate, poly(vinyl pyrrolidone), casein, starch, poly(acrylic acid), poly(methylmethacrylic acid), poly(vinyl chloride), poly(methacrylic acid), styrene-maleic anhydride copolymers, styrene-acrylonitrile copolymers, styrene-butadiene copolymers, poly(vinyl acetal) (e.g., poly(vinyl formal) or poly(vinyl butyral)), polyester, polyurethane, phenoxy resin, poly(vinylidene chloride), polyepoxide, polycarbonate, poly(vinyl acetate), polyolefin, cellulose esters, and polyamide. A binder may be used with water, an organic solvent or emulsion to form a coating solution.

In the present invention, the glass transition temperature (Tg) of the binder of the image forming layer is preferably in a range of from 10° C. to 80° C., more preferably from 20° C. to 70° C. and, even more preferably from 23° C. to 65° C.

In the specification, Tg is calculated according to the following equation.

$$1/Tg = \sum (Xi/Tgi)$$

where the polymer is obtained by copolymerization of n monomer compounds (from i=1 to i=n); Xi represents the mass fraction of the ith monomer ( $\sum Xi = 1$ ), and Tgi is the glass transition temperature (absolute temperature) of the homopolymer obtained with the ith monomer. The symbol  $\Sigma$  stands for the summation from i=1 to i=n.

Values for the glass transition temperature (Tgi) of the homopolymers derived from each of the monomers were obtained from J. Brandrup and E. H. Immergut, Polymer Handbook (3rd Edition) (Wiley-Interscience, 1989).

The binder may be of one kind or two or more kinds of polymers, when necessary. And, the polymer having Tg of 20° C. or more and the polymer having Tg of less than 20° C. can be used in combination. In the case where two or more kinds of polymers differing in Tg may be blended for use, it is preferred that the weight-average Tg is in the range mentioned above.

In the invention, in the case where the image forming layer is formed by first applying a coating solution containing 30% by weight or more of water in the solvent and by then drying, furthermore, in the case where the binder of the image forming layer is soluble or dispersible in an aqueous solvent (water solvent), and particularly in the case where a polymer latex having an equilibrium water content of 2% by weight or lower under 25° C. and 60% RH is used, the performance can be enhanced.

Most preferred embodiment is such prepared to yield an ion conductivity of 2.5 mS/cm or lower, and as such a preparing method, there can be mentioned a refining treatment using a separation function membrane after synthesizing the polymer.

The aqueous solvent in which the polymer is soluble or dispersible, as referred herein, signifies water or water containing mixed therein 70% by weight or less of a water-admixing organic solvent.

As water-admixing organic solvents, there can be used, for example, alcohols such as methyl alcohol, ethyl alcohol, propyl alcohol, and the like; cellosolves such as methyl cel-

## 82

solve, ethyl cellosolve, butyl cellosolve, and the like; ethyl acetate, dimethylformamide, and the like.

The term "equilibrium water content under 25° C. and 60% RH" as referred herein can be expressed as follows:

$$Equilibrium\ water\ content\ under\ 25^{\circ}\ C.\ and\ 60\% \ RH = [(W1 - W0)/W0] \times 100 \ (\% \ by \ weight)$$

wherein, W1 is the weight of the polymer in moisture-controlled equilibrium under the atmosphere of 25° C. and 60% RH, and W0 is the absolutely dried weight at 25° C. of the polymer.

For the definition and the method of measurement for water content, reference can be made to Polymer Engineering Series 14, "Testing methods for polymeric materials" (The Society of Polymer Science, Japan, published by Chijin Shokan).

The equilibrium water content under 25° C. and 60% RH is preferably 2% by weight or lower, more preferably, from 0.01% by weight to 1.5% by weight, and most preferably, from 0.02% by weight to 1% by weight.

The binders used in the invention are, particularly preferably, polymers capable of being dispersed in an aqueous solvent. Examples of dispersed states may include a latex, in which water-insoluble fine particles of hydrophobic polymer are dispersed, or such in which polymer molecules are dispersed in molecular states or by forming micelles, but preferred are latex-dispersed particles. The average particle size of the dispersed particles is in the range of from 1 nm to 50,000 nm, and preferably from 5 nm to 1,000 nm. There is no particular limitation concerning particle size distribution of the dispersed particles, and they may be widely distributed or may exhibit a monodisperse particle size distribution.

In the invention, preferred embodiment of the polymers capable of being dispersed in aqueous solvent includes hydrophobic polymers such as acrylic polymers, poly(ester), rubber (e.g., SBR resin), polyurethane, poly(vinyl chloride), poly(vinyl acetate), poly(vinylidene chloride), polyolefin, and the like. As the polymers above, usable are straight chain polymers, branched polymers, or crosslinked polymers; also usable are the so-called homopolymers in which one kind of monomer is polymerized, or copolymers in which two or more kinds of monomers are polymerized. In the case of a copolymer, it may be a random copolymer or a block copolymer.

The molecular weight of these polymers is, in number average molecular weight, in the range of from 5,000 to 1,000,000, preferably from 10,000 to 200,000. Those having too small a molecular weight exhibit insufficient mechanical strength on forming the image forming layer, and those having too large a molecular weight are also not preferred because the resulting film-forming properties are poor.

Specific examples of preferred polymer latexes are given below, which are expressed by the starting monomers with % by weight given in parenthesis. The molecular weight is given in number average molecular weight.

In the case polyfunctional monomer is used, the concept of molecular weight is not applicable because they build a crosslinked structure. Hence, they are denoted as "crosslinking", and the molecular weight is omitted. Tg represents glass transition temperature.

P-1; Latex of -MMA(70)-EA(27)-MAA(3)-(molecular weight 37000, Tg 61° C.)

P-2; Latex of -MMA(70)-2EHA(20)-St(5)-AA(5)-(molecular weight 40000, Tg 59° C.)

P-3; Latex of -St(50)-Bu(47)-MAA(3)-(crosslinking, Tg -17° C.)

## 83

- P-4; Latex of -St(68)-Bu(29)-AA(3)-(crosslinking, Tg 17° C.)
- P-5; Latex of -St(71)-Bu(26)-AA(3)-(crosslinking, Tg 24° C.)
- P-6; Latex of -St(70)-Bu(27)-IA(3)-(crosslinking)
- P-7; Latex of -St(75)-Bu(24)-AA(1)-(crosslinking, Tg 29° C.)
- P-8; Latex of -St(60)-Bu(35)-DVB(3)-MAA(2)-(crosslinking)
- P-9; Latex of -St(70)-Bu(25)-DVB(2)-AA(3)-(crosslinking)
- P-10; Latex of -VC(50)-MMA(20)-EA(20)-AN(5)-AA(5)-(molecular weight 80000)
- P-11; Latex of -VDC(85)-MMA(5)-EA(5)-MAA(5)-(molecular weight 67000)
- P-12; Latex of -Et(90)-MAA(10)-(molecular weight 12000)
- P-13; Latex of -St(70)-2EHA(27)-AA(3)-(molecular weight 130000, Tg 43° C.)
- P-14; Latex of -MMA(63)-EA(35)-AA(2)-(molecular weight 33000, Tg 47° C.)
- P-15; Latex of -St(70.5)-Bu(26.5)-AA(3)-(crosslinking, Tg 23° C.)
- P-16; Latex of -St(69.5)-Bu(27.5)-AA(3)-(crosslinking, Tg 20.5° C.)

In the structures above, abbreviations represent monomers as follows. MMA: methyl metacrylate, EA: ethyl acrylate, MAA: methacrylic acid, 2EHA: 2-ethylhexyl acrylate, St: styrene, Bu: butadiene, AA: acrylic acid, DVB: divinylbenzene, VC: vinyl chloride, AN: acrylonitrile, VDC: vinylidene chloride, Et: ethylene, IA: itaconic acid.

The polymer latexes above are commercially available, and polymers below are usable. As examples of acrylic polymers, there can be mentioned Cevian A-4635, 4718, and 4601 (all manufactured by Daicel Chemical Industries, Ltd.), Nipol Lx811, 814, 821, 820, and 857 (all manufactured by Nippon Zeon Co., Ltd.), and the like; as examples of polyester, there can be mentioned FINETEX ES650, 611, 675, and 850 (all manufactured by Dainippon Ink and Chemicals, Inc.), WDS-size and WMS (all manufactured by Eastman Chemical Co.), and the like; as examples of polyurethane, there can be mentioned HYDRAN AP10, 20, 30, and 40 (all manufactured by Dainippon Ink and Chemicals, Inc.), and the like; as examples of rubber, there can be mentioned LACSTAR 7310K, 3307B, 4700H, and 7132C (all manufactured by Dainippon Ink and Chemicals, Inc.), Nipol Lx416, 410, 438C, and 2507 (all manufactured by Nippon Zeon Co., Ltd.), and the like; as examples of poly(vinyl chloride), there can be mentioned G351 and G576 (all manufactured by Nippon Zeon Co., Ltd.), and the like; as examples of poly(vinylidene chloride), there can be mentioned L502 and L513 (all manufactured by Asahi Chemical Industry Co., Ltd.), and the like; as examples of polyolefin, there can be mentioned Chemipearl S120 and SA100 (all manufactured by Mitsui Petrochemical Industries, Ltd.), and the like.

The polymer latex above may be used alone, or may be used by blending two or more kinds depending on needs.

Particularly preferable as the polymer latex for use in the invention are that of styrene-butadiene copolymer. The weight ratio of monomer unit for styrene to that of butadiene constituting the styrene-butadiene copolymer is preferably in a range of from 40:60 to 95:5. Further, the monomer unit of styrene and that of butadiene preferably account for 60% by weight to 99% by weight with respect to the copolymer. Preferable range of molecular weight is similar to that described above.

## 84

- As the latex of styrene-butadiene copolymer preferably used in the invention, there can be mentioned P-3 to P-8, P-14, and P-15, or commercially available LACSTAR 3307B, LACSTAR 7132C, Nipol Lx416, and the like.
- 5 In the image forming layer of the photothermographic material according to the invention, if necessary, there can be added hydrophilic polymers such as gelatin, poly(vinyl alcohol), methyl cellulose, hydroxypropyl cellulose, carboxymethyl cellulose, or the like. These hydrophilic polymers are added at an amount of 30% by weight or less, and preferably 10 20% by weight or less, with respect to the total weight of the binder incorporated in the image forming layer.

According to the invention, the layer containing organic silver salt (image forming layer) is preferably formed by using polymer latex for the binder. According to the amount of the binder for the image forming layer, the weight ratio for total binder to organic silver salt (total binder/organic silver salt) is preferably in a range of from 1/10 to 10/1, and more preferably from 1/5 to 4/1.

- 15 20 The layer containing organic silver salt is, in general, a photosensitive layer (image forming layer) containing a photosensitive silver halide, i.e., the photosensitive silver salt; in such a case, the weight ratio for total binder to silver halide (total binder/silver halide) is in a range of from 400 to 5, and more preferably, from 200 to 10.

The total amount of binder in the image forming layer of the invention is preferably in a range of from 0.2 g/m<sup>2</sup> to 30 g/m<sup>2</sup>, and more preferably from 1 g/m<sup>2</sup> to 15 g/m<sup>2</sup>. As for the image forming layer of the invention, there may be added a 30 crosslinking agent for crosslinking, or a surfactant and the like to improve coating properties.

- In the invention, a solvent of a coating solution for the image forming layer in the photothermographic material of the invention (wherein a solvent and water are collectively described as a solvent for simplicity) is preferably an aqueous solvent containing water at 30% by weight or more. Examples of solvents other than water may include any of water-miscible organic solvents such as methyl alcohol, ethyl alcohol, isopropyl alcohol, methyl cellosolve, ethyl cellosolve, dimethylformamide, ethyl acetate, and the like. A water content in a solvent is more preferably 50% by weight or more, and even more preferably 70% by weight or more.

Concrete examples of a preferable solvent composition, in addition to water=100, are compositions in which methyl alcohol is contained at ratios of water/methyl alcohol=90/10 and 45 70/30, in which dimethylformamide is further contained at a ratio of water/methyl alcohol/dimethylformamide=80/15/5, in which ethyl cellosolve is further contained at a ratio of water/methyl alcohol/ethyl cellosolve=85/10/5, and in which isopropyl alcohol is further contained at a ratio of water/methyl alcohol/isopropyl alcohol=85/10/5 (wherein the numerals presented above are values in % by weight).

- (Antifoggant)
- 1) Organic Polyhalogen Compound
  - 55 It is preferred that the photothermographic material of the invention contains a compound expressed by formula (H) below as an antifoggant.

Q-(Y)<sup>n</sup>-C(Z<sub>1</sub>)(Z<sub>2</sub>)X Formula (H)

60 In formula (H), Q represents one selected from an alkyl group, an aryl group, or a heterocyclic group; Y represents a divalent linking group; n represents 0 or 1; Z<sub>1</sub> and Z<sub>2</sub> each represent a halogen atom; and X represents a hydrogen atom or an electron-attracting group.

65 Q is preferably a phenyl group substituted by an electron-attracting group whose Hammett substituent constant  $\sigma_p$  yields a positive value. For the details of Hammett substituent

85

constant, reference can be made to Journal of Medicinal Chemistry, vol. 16, No. 11 (1973), pages 1207 to 1216, and the like.

As such electron-attracting groups, examples include a halogen atom (fluorine atom (op value: 0.06), chlorine atom (op value: 0.23), bromine atom (op value: 0.23), iodine atom (op value: 0.18)), a trihalomethyl group (tribromomethyl (op value: 0.29), trichloromethyl (op value: 0.33), trifluoromethyl (op value: 0.54)), a cyano group (up value: 0.66), a nitro group (op value: 0.78), an aliphatic aryl sulfonyl group or a heterocyclic sulfonyl group (for example, methanesulfonyl (op value: 0.72)), an aliphatic aryl acyl group or a heterocyclic acyl group (for example, acetyl (op value: 0.50) and benzoyl (op value: 0.43)), an alkynyl group (e.g.,  $C\equiv CH$  (op value: 0.23)), an aliphatic aryl oxycarbonyl group or a heterocyclic oxycarbonyl group (e.g., methoxycarbonyl (op value: 0.45) and phenoxy carbonyl (op value: 0.44)), a carbamoyl group (op value: 0.36), a sulfamoyl group (op value: 0.57), a sulfoxido group, a heterocyclic group, a phosphoryl group, and the like. Preferred range of the op value is from 0.2 to 2.0, and more preferably, from 0.4 to 1.0.

Preferred as the electron-attracting group are a carbamoyl group, an alkoxy carbonyl group, an alkylsulfonyl group, an alkylphosphoryl group, a carboxyl group, an alkylcarbonyl group, an arylcarbonyl group, and an arylsulfonyl group. Particularly preferred among them are a carbamoyl group, an alkoxy carbonyl group, an alkylsulfonyl group, and an alkylphosphoryl group, and most preferred is a carbamoyl group.

X is preferably an electron-attracting group; more preferably, a halogen atom, an aliphatic aryl sulfonyl group, a heterocyclic sulfonyl group, an aliphatic aryl acyl group, a heterocyclic acyl group, an aliphatic aryl oxycarbonyl group, a heterocyclic oxycarbonyl group, a carbamoyl group, or a sulfamoyl group; particularly preferred among them is a halogen atom.

Among halogen atoms, preferred are a chlorine atom, bromine atom, and iodine atom; more preferred are a chlorine atom and bromine atom; and particularly preferred is a bromine atom.

Y preferably represents  $-C(=O)-$ ,  $-SO-$ , or  $-SO_2-$ ; more preferably,  $-C(=O)-$  or  $-SO_2-$ ; and particularly preferred is  $-SO_2-$ . n represents 0 or 1, and preferably represents 1.

Specific examples of the compounds expressed by formula (H) of the invention are shown below, but the present invention is not limited in these.



H-1

H-12



H-2

H-13



H-3



65

86

-continued

H-4



H-5



H-6



H-7



H-8



H-9



H-10



H-11



H-12



H-13



65

-continued



-continued



H-19      The compound expressed by formula (H) of the invention  
40      is preferably used in an amount of from  $10^{-4}$  mol to 0.8 mol,  
more preferably, from  $10^{-3}$  mol to 0.1 mol, and further preferably,  
from  $5 \times 10^{-3}$  mol to 0.05 mol, per 1 mol of non-photosensitive silver salt incorporated in the image forming layer in each case.

H-20      Particularly, in the case where a silver halide having a  
45      composition of a high silver iodide content according to the  
invention is used, an addition amount of the compound  
expressed by formula (H) is important in order to obtain a  
sufficient anti-fogging effect and the compound is most preferably  
used in a range of from  $5 \times 10^{-3}$  mol to 0.03 mol.

H-21      In the invention, methods of incorporating a compound  
50      expressed by formula (H) into a photothermographic material  
are described in the methods of incorporating a reducing  
agent described above.

H-22      A melting point of a compound expressed by formula (H)  
55      is preferably 200°C. or lower, and more preferably 170°C. or lower.

H-23      Examples of other organic polyhalogen compound used in  
the invention are disclosed in paragraph Nos. 0111 to 0112 of  
JP-A No. 11-65021. Preferable examples thereof are an  
organic halogen compound expressed by formula (P)  
described in JP-A No. 11-87297, an organic polyhalogen  
compound expressed by formula (II) described in JP-A No.  
10-339934 and an organic polyhalogen compound described  
in JP-A No. 2001-033911.

## 2) Other Antifoggants

H-24      As other antifoggants, there can be mentioned a mercury  
(II) salt described in paragraph number 0113 of JP-A No.

11-65021, benzoic acids described in paragraph number 0114 of the same literature, a salicylic acid derivative described in JP-A No. 2000-206642, a formaline scavenger compound expressed by formula (S) in JP-A No. 2000-221634, a triazine compound related to Claim 9 of JP-A No. 11-352624, a compound expressed by formula (III), 4-hydroxy-6-methyl-1,3,3a,7-tetrazaindene, and the like, described in JP-A No. 6-11791.

As an antifoggant, stabilizer and stabilizer precursor usable in the invention, there can be mentioned those disclosed in paragraph number 0070 of JP-A No. 10-62899 and in line 57 of page 20 to line 7 of page 21 of EP No. 0803764A1, the compounds described in JP-A Nos. 9-281637 and 9-329864.

The photothermographic material of the invention may further contain an azonium salt in order to prevent fogging. Azonium salts useful in the present invention include a compound expressed by formula (XI) described in JP-A No. 59-193447, a compound described in JP-B No. 55-12581, and a compound expressed by formula (II) in JP-A No. 60-153039. The azonium salt may be added to any part of the photothermographic material, but as an additional layer, it is preferred to select a layer on the side having thereon the image forming layer, and more preferred is to select the image forming layer itself.

The azonium salt may be added at any time of the process of preparing the coating solution; in the case where the azonium salt is added into the image forming layer, any time of the process may be selected, from the preparation of the organic silver salt to the preparation of the coating solution, but preferred is to add the salt after preparing the organic silver salt and just before coating. As the method for adding the azonium salt, any method using a powder, a solution, a fine-particle dispersion, and the like, may be used. Furthermore, it may be added as a solution having mixed therein other additives such as sensitizing agents, reducing agents, toners, and the like.

In the invention, the azonium salt may be added at any amount, but preferably, it is added in a range of from  $1 \times 10^{-6}$  mol to 2 mol, and more preferably, from  $1 \times 10^{-3}$  mol to 0.5 mol per 1 mol of silver.

#### (Other Additives)

##### 1) Mercapto Compounds, Disulfides and Thiones

In the invention, mercapto compounds, disulfide compounds, and thione compounds can be added in order to control the development by suppressing or enhancing development, to improve spectral sensitization efficiency, and to improve storage properties before and after development. Descriptions can be found in paragraph Nos. 0067 to 0069 of JP-A No. 10-62899, a compound expressed by formula (I) of JP-A No. 10-186572 and specific examples thereof shown in paragraph Nos. 0033 to 0052, in lines 36 to 56 in page 20 of EP No. 0803764A1, in JP-A No. 2001-100358 and the like. Among them, mercapto-substituted heterocyclic aromatic compound is preferred.

##### 2) Toner

In the photothermographic material of the present invention, the addition of a toner is preferred. The description of the toner can be found in JP-A No. 10-62899 (paragraph Nos. 0054 to 0055), EP No. 0803764A1 (page 21, lines 23 to 48), JP-A Nos. 2000-356317 and 2000-187298. Preferred are phthalazinones (phthalazinone, phthalazinone derivatives and metal salts thereof, (e.g., 4-(1-naphthyl)phthalazinone, 6-chlorophthalazinone, 5,7-dimethoxyphthalazinone, and 2,3-dihydro-1,4-phthalazinedione); combinations of phthalazinones and phthalic acids (e.g., phthalic acid, 4-methylphthalic acid, 4-nitrophthalic acid, diammonium phthalate, sodium phthalate, potassium phthalate, and tetrachloro-

rophthalic anhydride); phthalazines (phthalazine, phthalazine derivatives and metal salts thereof, (e.g., 4-(1-naphthyl)phthalazine, 6-isopropylphthalazine, 6-tert-butylphthalazine, 6-chlorophthalazine, 5,7-dimethoxyphthalazine, and 2,3-dihydrophthalazine); combinations of phthalazines and phthalic acids. Particularly with regard to a combination with silver halide having a high silver iodide content, preferred is a combination of phthalazines and phthalic acids.

10 The addition amount of phthalazines is preferably from 0.01 mol to 0.3 mol per 1 mol of organic silver salt, more preferably from 0.02 mol to 0.2 mol, and particularly preferably from 0.02 mol to 0.1 mol. The addition amount of the compound is a very important factor for accelerating the development of the silver halide emulsion having high silver iodide content used for the present invention. The adequate selection of the addition amount may be capable of providing sufficient development performance while depressing fog.

##### 3) Plasticizer and Lubricant

20 Plasticizers and lubricants usable in the image forming layer of the invention are described in paragraph No. 0117 of JP-A No. 11-65021. Lubricants are described in paragraph Nos. 0061 to 0064 of JP-A No. 11-84573.

##### 4) Dyes and Pigments

25 From the viewpoint of improving color tone, preventing the generation of interference fringes and preventing irradiation on laser exposure, various kinds of dyes and pigments (for instance, C.I. Pigment Blue 60, C.I. Pigment Blue 64, and C.I. Pigment Blue 15:6) can be used in the image forming layer of the invention. Detailed description can be found in WO No. 98/36322, JP-A Nos. 10-268465 and 11-338098, and the like.

##### 5) Nucleation Accelerator

30 A nucleation accelerator can be used with the nucleator of the invention. Concerning a nucleation accelerator, description can be found in paragraph No. 0102 of JP-A No. 11-65021, and in paragraph Nos. 0194 to 0195 of JP-A No. 11-223898.

40 As the nucleation accelerator, it is preferred to use an acid resulting from hydration of diphosphorus pentaoxide, or a salt thereof. Acids resulting from the hydration of diphosphorus pentaoxide or salts thereof include metaphosphoric acid (salt), pyrophosphoric acid (salt), orthophosphoric acid (salt), triphosphoric acid (salt), tetraphosphoric acid (salt), hexametaphosphoric acid (salt), and the like. Particularly preferred acids obtainable by the hydration of diphosphorus pentaoxide or salts thereof include orthophosphoric acid (salt) and hexametaphosphoric acid (salt). Specifically mentioned as the salts are sodium orthophosphate, sodium dihydrogen orthophosphate, sodium hexametaphosphate, ammonium hexametaphosphate, and the like.

45 The addition amount of the acid obtained by hydration of diphosphorus pentaoxide or the salt thereof (i.e., the coating amount per 1 m<sup>2</sup> of the photothermographic material) may be set as desired depending on sensitivity and fogging, but preferred is an amount of from 0.1 mg/m<sup>2</sup> to 500 mg/m<sup>2</sup>, and more preferably, from 0.5 mg/m<sup>2</sup> to 100 mg/m<sup>2</sup>.

##### (Preparation of Coating Solution and Coating)

50 The temperature for preparing the coating solution for the image forming layer of the invention is preferably from 30°C. to 65°C., more preferably, 35°C. or more and less than 60°C., and further preferably, from 35°C. to 55°C. Furthermore, the temperature of the coating solution for the image forming layer immediately after adding the polymer latex is preferably maintained in the temperature range from 30°C. to 65°C.

## 2. Layer Constitution and Other Constituting Components

The photothermographic material of the present invention is a double-sided type photothermographic material which has image forming layers on both sides of the support.

## (Double-Sided Type Photothermographic Material)

The photothermographic material of the present invention is preferably applied for an image forming method to record X-ray images using a fluorescent intensifying screen.

For the image forming method, the photothermographic material as described below can be preferably employed: where the photothermographic material is exposed with a monochromatic light having the same wavelength as the main emission peak wavelength of the fluorescent intensifying screen and having a half band width of  $15\text{ nm} \pm 5\text{ nm}$ , and after a thermal developing process, an exposure value required for obtaining an image density of  $\text{fog}+0.5$  after removing the image forming layer that is disposed on the opposite side from an exposure face is from  $1 \times 10^{-6}\text{ watt}\cdot\text{sec}\cdot\text{m}^{-2}$  to  $1 \times 10^{-3}\text{ watt}\cdot\text{sec}\cdot\text{m}^{-2}$ , and preferably from  $6 \times 10^{-6}\text{ watt}\cdot\text{sec}\cdot\text{m}^{-2}$  to  $6 \times 10^{-4}\text{ watt}\cdot\text{sec}\cdot\text{m}^{-2}$ .

The image forming method using the photothermographic materials described above comprises:

- (a) providing an assembly for forming an image by placing the photothermographic material between a pair of the X-ray intensifying screens,
- (b) putting an analyte between the assembly and the X-ray source,
- (c) applying X-rays having an energy level in a range of 25 kVp to 125 kVp to the analyte;
- (d) taking the photothermographic material out of the assembly; and
- (e) heating the removed photothermographic material in a temperature range of  $90^\circ\text{ C.}$  to  $180^\circ\text{ C.}$

The photothermographic material used for the assembly in the present invention is subjected to X-ray exposure through a step wedge tablet and thermal development. On the photographic characteristic curve having an optical density (D) and an exposure value (log E) along the rectangular coordinates having the equal axis-of-coordinate unit, it is preferred to adjust so that the thermal developed image may have the photographic characteristic curve where the average gamma ( $\gamma$ ) made at the points of a density of  $\text{fog}+0.1$  and a density of  $\text{fog}+0.5$  is from 0.5 to 0.9, and the average gamma ( $\gamma$ ) made at the points of a density of  $\text{fog}+1.2$  and a density of  $\text{fog}+1.6$  is from 3.2 to 4.0.

For the X-ray radiography employed in the practice of the present invention, the use of photothermographic material having the aforesaid photographic characteristic curve would give the radiation images with excellent photographic properties that exhibit an extended bottom portion and high gamma value at a middle density area. According to this photographic property, the photographic properties mentioned have the advantage of that the depiction in a low density portion on the mediastinal region and the heart shadow region having little X-ray transmittance becomes excellent, and that the density becomes easy to view, and that gradation in the images on the lung field region having much X-ray transmittance becomes excellent.

The photothermographic material having a preferred photographic characteristic curve mentioned above can be easily prepared, for example, by the method where each of the image forming layer of both sides may be constituted of two or more image forming layers containing silver halide and having a sensitivity different from each other. Especially, the aforesaid image forming layer preferably comprises an emulsion of high sensitivity for the upper layer and an emulsion with photographic properties of low sensitivity and high gra-

dation for the lower layer. In the case of preparing the image forming layer comprising two layers, the sensitivity difference between the silver halide emulsion in each layer is preferably from 1.5 times to 20 times, and more preferably from 2 times to 15 times.

The ratio of the amount of emulsion used for forming each layer may depend on the sensitivity difference between emulsions used and the covering power. Generally, as the sensitivity difference is large, the ratio of the using amount of high sensitivity emulsion is reduced. For example, if the sensitivity difference is two times, and the covering power is equal, the ratio of the amount of high sensitivity emulsion to low sensitivity emulsion would be preferably adjusted to be in a range of from 1:20 to 1:50 with respect to the amount of silver.

## 15 (Fluorescent Intensifying Screen)

Next, the fluorescent intensifying screen employed in the practice of the present invention is explained below. The fluorescent intensifying screen essentially comprises a support and a fluorescent substance layer coated on one side of 20 the support as the fundamental structure. The fluorescent substance layer is a layer where the fluorescent substance is dispersed in binders. On the surface of a fluorescent substance layer opposite to the support side (the surface of the side that does not face on the support), a transparent protective layer is 25 generally disposed to protect the fluorescent substance layer from chemical degradation and physical shock.

Preferred fluorescent substances according to the present invention are described below.

Tungstate fluorescent substances ( $\text{CaWO}_4$ ,  $\text{MgWO}_4$ , 30  $\text{CaWO}_4\text{:Pb}$ , and the like), terbium activated rare earth sulfoxide fluorescent substances ( $\text{Y}_2\text{O}_3\text{:Tb}$ ,  $\text{Gd}_2\text{O}_3\text{S:Tb}$ ,  $\text{La}_2\text{O}_3\text{S:Tb}$ ,  $(\text{Y},\text{Gd})_2\text{O}_3\text{S:Tb}$ ,  $(\text{Y},\text{Gd})\text{O}_3\text{S:Tb}$ ,  $\text{Tm}$ , and the like), terbium activated rare earth phosphate fluorescent substances 35 ( $\text{YPO}_4\text{:Tb}$ ,  $\text{GdPO}_4\text{:Tb}$ ,  $\text{LaPO}_4\text{:Tb}$ , and the like), terbium activated rare earth oxyhalogen fluorescent substances ( $\text{LaOBr:Tb}$ ,  $\text{LaOBr:Tb}$ ,  $\text{Tm}$ ,  $\text{LaOCl:Tb}$ ,  $\text{LaOCl:Tb}$ ,  $\text{Tm}$ ,  $\text{LaOBr:Tb}$ ,  $\text{GdOBr:Tb}$ ,  $\text{GdOCl:Tb}$ , and the like), thulium activated rare 40 earth oxyhalogen fluorescent substances ( $\text{LaOBr:Tm}$ ,  $\text{LaOCl:Tm}$ , and the like), barium sulfate fluorescent substances ( $\text{BaSO}_4\text{:Pb}$ ,  $\text{BaSO}_4\text{:Eu}^{2+}$ ,  $(\text{Ba},\text{Sr})\text{SO}_4\text{:Eu}^{2+}$ , and the like), divalent europium activated alkali earth metal phosphate 45 fluorescent substances ( $(\text{Ba}_2\text{PO}_4)_2\text{:Eu}^{2+}$ ,  $(\text{Ba}_2\text{PO}_4)_2\text{:Eu}^{2+}$ , and the like), divalent europium activated alkali earth metal fluorinated halogenide fluorescent substances ( $\text{BaFCl:Eu}^{2+}$ ,  $\text{BaFBr:Eu}^{2+}$ ,  $\text{BaFCl:Eu}^{2+}$ ,  $\text{Tb}$ ,  $\text{BaF}_2\text{-BaCl-KCl:Eu}^{2+}$ ,  $(\text{Ba},\text{Mg})\text{F}_2\text{-BaCl-KCl:Eu}^{2+}$ , and the like), iodide fluorescent substances ( $\text{CsI:Na}$ ,  $\text{CsI:Tl}$ ,  $\text{NaI}$ ,  $\text{KI:Tl}$ , and the like), sulfide fluorescent substances ( $\text{ZnS:Ag}$ ,  $(\text{Zn},\text{Cd})\text{S:Cu}$ ,  $(\text{Zn},\text{Cd})\text{S:Cu}$ ,  $\text{Al}$ , and the like), hafnium phosphate fluorescent substances ( $\text{HfP}_2\text{O}_7\text{:Cu}$  and the like),  $\text{YTaO}_4$  and a substance in which various activator is 50 added as an emission center to  $\text{YTaO}_4$ .

However, the fluorescent substance used in the present invention is not particularly limited to these specific 55 examples, so long as to emit light in visible or near ultraviolet region by exposure to a radioactive ray.

The fluorescent intensifying screen which is more preferred for the present invention is a screen where 50% or more of the emission light has a wavelength region from 350 nm to 60 420 nm. Especially, as the fluorescent substance, a divalent europium activated fluorescent substance is preferred, and a divalent europium activated barium halide fluorescent substance is more preferred. The emission wavelength region is preferably from 360 nm to 420 nm, and more preferably from 65 370 nm to 420 nm. Moreover, the preferred fluorescent screen can emit 70% or more of the above region, and more preferably 85% or more thereof.

The ratio of the emission light can be calculated from the following method; the emission spectrum is measured where an antilogarithm of the emission wavelength is plotted on the abscissa axis at equal interval and a number of the emitted photon is plotted on the ordinate. The ratio of the emission light in the wavelength region from 350 nm to 420 nm is defined as a value dividing the area from 350 nm to 420 nm on the chart by the entire area of the emission spectrum. The photothermographic materials of the present invention used in combination with the fluorescent substance emitting the above wavelength region can attain high sensitivity.

In order that most of the emission light of the fluorescent substance may exist in the above wavelength region, the narrower half band width is preferred. The preferred half band width is from 1 nm to 70 nm, more preferably from 5 nm to 50 nm, and even more preferably from 10 nm to 40 nm.

So long as the fluorescent substance has the above emission, the fluorescent substance used in the present invention is not particularly limited, but the europium activated fluorescent substance where the divalent europium is an emission center is preferred to attain high sensitivity as the purpose of the invention. Specific examples of these fluorescent substances are described below, but the scope of the present invention is not limited to the examples.

BaFCl:Eu, BaFBr:Eu, BaFI:Eu, and the fluorescent substances where their halogen composition is changed; BaSO<sub>4</sub>:Eu, SrFBr:Eu, SrFCl:Eu, SrFI:Eu, (Sr,Ba)Al<sub>2</sub>Si<sub>2</sub>O<sub>8</sub>:Eu, SrB<sub>4</sub>O<sub>7</sub>F:Eu, SrMgP<sub>2</sub>O<sub>7</sub>:Eu, Sr<sub>3</sub>(PO<sub>4</sub>)<sub>2</sub>:Eu, Sr<sub>2</sub>P<sub>2</sub>O<sub>7</sub>:Eu, and the like.

More preferred fluorescent substance is a divalent europium activated barium halide fluorescent substance expressed by the following formula:



wherein, M represents Ba as a main component, but a small amount of Mg, Ca, Sr, or other compounds may be included. X<sub>1</sub> and X<sub>2</sub> each represent a halogen atom, and can be selected from F, Cl, Br and I. Herein, X<sub>1</sub> is more preferably a fluorine atom. X<sub>2</sub> can be selected from Cl, Br, and I, and the mixture with other halogen composition may be used preferably. More preferably X<sub>1</sub>=Br. Eu represents an europium atom. Eu as an emission center is preferably contained at a ratio from 10<sup>-7</sup> to 0.1, based on Ba, more preferably from 10<sup>-4</sup> to 0.05. Preferably the mixture with a small quantity of other compounds can be included. As most preferred fluorescent substance, BaFCl:Eu, BaFBr:Eu and BaFBr<sub>1-X</sub>I<sub>X</sub>:Eu can be described.

The fluorescent intensifying screen preferably consists of a support, an undercoat layer on the support, a fluorescent substance layer, and a surface protective layer.

The fluorescent substance layer is prepared as follows. A dispersion solution is prepared by dispersing the fluorescent substance particles described above in an organic solvent solution containing binder resins. The thus prepared solution is coated directly on the support (or on the undercoat layer such as a light reflective layer provided beforehand on the support) and dried to form the fluorescent substance layer. Besides the above method, the fluorescent substance layer may be formed by the steps of coating the above dispersion solution on the temporary support, drying the coated dispersion to form a fluorescent substance layer sheet, peeling off the sheet from the temporary support, and fixing the sheet onto a permanent support by means of an adhesive agent.

The particle size of the fluorescent substance particles used in the present invention is not particularly restricted, but is usually in a range of from about 1 μm to 15 μm, and preferably

from about 2 μm to 10 μm. The higher volume filling factor of the fluorescent substance particles in the fluorescent substance layer is preferred, usually in the range of from 60% to 85%, preferably from 65% to 80%, and particularly preferably from 68% to 75%. (The ratio of the fluorescent substance particles in the fluorescent substance layer is usually 80% by weight or more, preferably 90% by weight or more, and particularly preferably 95% by weight or more). Various kinds of known documents have described the binder resins, organic solvents, and the various additives used for forming the fluorescent substance layer. The thickness of the fluorescent substance layer may be set arbitrary according to the target sensitivity, but is preferably in a range of from 70 μm to 150 μm for the front side screen, and in a range of from 80 μm to 400 μm for the backside screen. The X-ray absorption efficiency of the fluorescent substance layer depends on the coating amount of the fluorescent substance particles in the fluorescent substance layer.

The fluorescent substance layer may consist of one layer, or 20 may consist of two or more layers. It preferably consists of one to three layers, and more preferably, one or two layers. For example, the layer may be prepared by coating a plurality of layers comprising the fluorescent substance particles with different particle size having a comparatively narrow particle 25 size distribution. In that case, the particle size of the fluorescent substance particles contained in each layer may gradually decrease from the top layer to the bottom layer provided next to the support. Especially, the fluorescent substance particles having a large particle size is preferably coated at the 30 side of the surface protective layer and fluorescent substance particles having a small particle size is preferably coated at the side of the support. Hereto, the small particle size of fluorescent substance is preferably in the range of from 0.5 μm to 2.0 μm and the large size is preferably in the range of 35 from 10 μm to 30 μm. The fluorescent substance layer may be formed by mixing the fluorescent substance particles with different particle sizes, or the fluorescent substances may be packed in a particle size graded structure as described in JP-A No. 55-33560 (page 3, line 3 on the left column to page 4, line 40 39 on the left column). Usually, a variation coefficient of a particle size distribution of the fluorescent substance is in a range of from 30% to 50%, but a monodispersed fluorescent substance particles with a variation coefficient of less than 30% can also be preferably used.

Attempts to attain a desired sharpness by dying the fluorescent substance layer with respect to the emission light wavelength are practiced. However, the layer with least dying is preferably required. The absorption length of the fluorescent substance layer is preferably 100 μm or more, and more 50 preferably 1000 μm or more.

The scattering length of the fluorescent substance layer is 55 preferably designed to be from 0.1 μm to 100 μm, and more preferably from 1 μm to 100 μm. The scattering length and the absorption length can be calculated from the equation based on the theory of Kubelka-Munk mentioned below.

Concerning the support, any support can be selected from various kinds of supports used in the well-known radiographic intensifying screen depending on the purpose. For example, a polymer film containing white pigments such as 60 titanium dioxide or the like, and a polymer film containing black pigments such as carbon black or the like may be preferably used. An undercoat layer such as a light reflective layer containing a light reflective agent may be preferably coated on the surface of the support (the surface of the fluorescent substance layer side). The light reflective layer as described in JP-A No. 2001-124898 may be preferably used. Especially, the light reflective layer containing yttrium oxide 65

described in Example 1 of the above patent or the light reflective layer described in Example 4 thereof is preferred. As for the preferred light reflective layer, the description in JP-A No. 23001-124898 (paragraph 3, 15 line on the right side to paragraph 4, line 23 on the right side) can be referred.

A surface protective layer is preferably coated on the surface of the fluorescent substance layer. The light scattering length measured at the main emission wavelength of the fluorescent substance is preferably in a range of from 5  $\mu\text{m}$  to 80  $\mu\text{m}$ , and more preferably from 10  $\mu\text{m}$  to 70  $\mu\text{m}$ , and particularly preferably from 10  $\mu\text{m}$  to 60  $\mu\text{m}$ . The light scattering length indicates a mean distance in which a light travels straight until it is scattered. Therefore a short scattering length means that the light scattering efficiency is high. On the other hand, the light absorption length, which indicates a mean free distance until a light is absorbed, is optional. From the viewpoint of the screen sensitivity, no absorption by the surface protective layer favors preventing the desensitization. In order to compensate the scattering loss, a very slightly absorption may be allowable. A preferred absorption length is 800  $\mu\text{m}$  or more, and more preferably 1200  $\mu\text{m}$  or more. The light scattering length and the light absorption length can be calculated from the equation based on the theory of Kubelka-Munk using the measured data obtained by the following method.

Three or more film samples comprising the same component composition as the surface protective layer of the aimed sample but a different thickness from each other are prepared, and then the thickness ( $\mu\text{m}$ ) and the diffuse transmittance (%) of each of the samples is measured. The diffuse transmittance can be measured by means of a conventional spectrophotometer equipped with an integrating sphere. For the measurement of the present invention, an automatic recording spectrophotometer (type U-3210, manufactured by Hitachi Ltd.) equipped with an integrating sphere of 150 $\phi$  (150-0901) is used. The measuring wavelength must correspond to the wavelength of the main emission peak of the fluorescent substance in the fluorescent substance layer having the surface protective layer.

Thereafter, the film thickness ( $\mu\text{m}$ ) and the diffuse transmittance (%) obtained in the above measurement is introduced to the following equation (A) derived from the theoretical equation of Kubelka-Munk. For example, the equation (A) can be derived easily, under the boundary condition of the diffuse transmittance (%), from the equations 5·1·12 to 5·1·15 on page 403 described in "Keikotai Hando Bukku" (the Handbook of Fluorescent Substance) (edited by Keikotai Gakkai, published by Ohmsha Ltd. 1987).

$$T/100 = 4\beta/[(1+\beta)^2 \cdot \exp(\alpha d) - (1-\beta)^2 \cdot \exp(-\alpha d)] \quad \text{Equation (A)}$$

wherein, T represents a diffuse transmittance (%), d represents a film thickness ( $\mu\text{m}$ ) and,  $\alpha$  and  $\beta$  are defined by the following equation respectively.

$$\alpha = [K \cdot (K+2S)]^{1/2}$$

$$\beta = [K/(K+2S)]^{1/2}$$

T (diffuse transmittance: %) and d (film thickness:  $\mu\text{m}$ ) measured from three or more film samples are introduced respectively to the equation (A), and thereby the value of K and S are determined to satisfy the equation (A). The scattering length ( $\mu\text{m}$ ) and the absorption length ( $\mu\text{m}$ ) are defined by 1/S and 1/K respectively.

The surface protective layer may preferably comprise light scattering particles dispersed in a resin material. The light refractive index of the light scattering particles is usually 1.6 or more, and more preferably 1.9 or more. The particle size of

the light scattering particles is in a range of from 0.1  $\mu\text{m}$  to 1.0  $\mu\text{m}$ . Examples of the light scattering particles may include the fine particles of aluminum oxide, magnesium oxide, zinc oxide, zinc sulfide, titanium oxide, niobium oxide, barium sulfate, lead carbonate, silicon oxide, polymethyl methacrylate, styrene, and melamine.

The resin materials used to form the surface protective layer are not particularly limited, but poly(ethylene terephthalate), poly(ethylene naphthalate), polyamide, aramid, 10 fluororesin, polyesters, or the like are preferably used. The surface protective layer can be formed by the step of dispersing the light scattering particles set forth above in an organic solvent solution containing the resin material (binder resin) to 15 prepare a dispersion solution, coating the dispersion solution on the fluorescent substance layer directly (or via an optionally provided auxiliary layer), and then drying the coated solution. By other way, the surface protective sheets prepared 20 separately can be overlaid on the fluorescent substance layer by means of an adhesive agent. The thickness of the surface protective layer is usually in a range of from 2  $\mu\text{m}$  to 12  $\mu\text{m}$ , and more preferably from 3.5  $\mu\text{m}$  to 10  $\mu\text{m}$ .

In addition, in respect with the preferred producing methods and the materials used for the process of the radiographic intensifying screen, references can be made to various publications, for example, JP-A No. 9-21899 (page 6, line 47 on left column to page 8, line 5 on left column), JP-A No. 6-347598 (page 2, line 17 on right column to page 3, line 33 on left column) and (page 3, line 42 on left column to page 4, line 22 on left column).

30 In the fluorescent intensifying sheets used for the present invention, the fluorescent substance is preferably packed in a particle size graded structure. Especially, the fluorescent substance particles having a large particle size are preferably coated at the side of the surface protective layer and fluorescent substance particles having a small particle size are preferably coated at the side of the support. The small particle size of fluorescent substance is preferably in the range of from 0.5  $\mu\text{m}$  to 2.0  $\mu\text{m}$ , and the large size is preferably in the range of from 10  $\mu\text{m}$  to 30  $\mu\text{m}$ .

#### 40 (Non-Photosensitive Layers)

The photothermographic material according to the invention can have a non-photosensitive layer in addition to the image forming layer. The non-photosensitive layers can be classified depending on the layer arrangement into (a) a surface protective layer provided on the image forming layer (on the side farther from the support), (b) an intermediate layer provided among plural image forming layers or between the image forming layer and the protective layer, (c) an undercoat layer provided between the image forming layer and the support, and (d) a back layer provided to the side opposite to the image forming layer.

Furthermore, a layer that functions as an optical filter may be provided as (a) or (b) above. An antihalation layer may be provided as (c) or (d) to the photothermographic material.

#### 55 1) Surface Protective Layer

The photothermographic material of the invention can comprise a surface protective layer with an object to prevent adhesion of the image forming layer. The surface protective layer may be a single layer, or plural layers. Description of the surface protective layer may be found in paragraph Nos. 0119 to 0120 of JP-A No. 11-65021 and in JP-A No. 2001-348546.

60 Preferred as the binder of the surface protective layer of the invention is gelatin, but poly(vinyl alcohol) (PVA) may be used preferably instead, or in combination. As gelatin, there can be used an inert gelatin (e.g., Nitta gelatin 750), a phthalated gelatin (e.g., Nitta gelatin 801), and the like.

Usable as PVA are those described in paragraph Nos. 0009 to 0020 of JP-A No. 2000-171936, and preferred are the completely saponified product PVA-105 and the partially saponified PVA-205 and PVA-335, as well as modified poly(vinyl alcohol) MP-203 (trade name of products from Kuraray Ltd.).

The coating amount of poly(vinyl alcohol) (per 1 m<sup>2</sup> of support) in the protective layer (per one layer) is preferably in a range of from 0.3 g/m<sup>2</sup> to 4.0 g/m<sup>2</sup>, and more preferably, from 0.3 g/m<sup>2</sup> to 2.0 g/m<sup>2</sup>.

The coating amount of total binder (including water-soluble polymer and latex polymer) (per 1 m<sup>2</sup> of support) in the surface protective layer (per one layer) is preferably in a range of from 0.3 g/m<sup>2</sup> to 5.0 g/m<sup>2</sup>, and more preferably, from 0.3 g/m<sup>2</sup> to 2.0 g/m<sup>2</sup>.

### 2) Antihalation Layer

The photothermographic material of the present invention can comprise an antihalation layer provided to the side farther from the light source with respect to the image forming layer. Descriptions on the antihalation layer can be found in paragraph Nos. 0123 to 0124 of JP-A No. 11-65021, in JP-A Nos. 11-223898, 9-230531, 10-36695, 10-104779, 11-231457, 11-352625, 11-352626, and the like.

The antihalation layer contains an antihalation dye having its absorption at the wavelength of the exposure light. In the case the exposure wavelength is in the infrared region, an infrared-absorbing dye may be used, and in such a case, preferred are dyes having no absorption in the visible region.

In the case of preventing halation from occurring by using a dye having absorption in the visible region, it is preferred that the color of the dye would not substantially remain after image formation, and is preferred to employ a means for decoloring by the heat of thermal development; in particular, it is preferred to add a thermal bleaching dye and a base precursor to the non-photosensitive layer to impart function as an antihalation layer. Those techniques are described in JP-A No. 11-231457 and the like.

The addition amount of the bleaching dye is determined depending on the usage of the dye. In general, it is used at an amount as such that the optical density (absorbance) exceeds 0.1 when measured at the desired wavelength. The optical density is preferably in a range of from 0.2 to 2. The addition amount of dyes to obtain optical density in the above range is generally from about 0.001 g/m<sup>2</sup> to 1 g/m<sup>2</sup>.

By decoloring the dye in such a manner, the optical density after thermal development can be lowered to 0.1 or lower. Two or more kinds of bleaching dyes may be used in combination in a photothermographic material. Similarly, two or more kinds of base precursors may be used in combination.

In the case of thermal decolorization by the combined use of a bleaching dye and a base precursor, it is advantageous from the viewpoint of thermal decolorization efficiency to further use a substance capable of lowering the melting point by at least 3° C. (deg) when mixed with the base precursor (e.g., diphenylsulfone or 4-chlorophenyl(phenyl)sulfone) as disclosed in JP-A No. 11-352626.

In the invention, coloring matters having maximum absorption in the wavelength range of from 300 nm to 450 nm can be added in order to improve color tone of developed silver images and a deterioration of the images during aging. Such coloring matters are described in, for example, JP-A Nos. 62-210458, 63-104046, 63-103235, 63-208846, 63-306436, 63-314535, 01-61745, 2001-100363, and the like.

### 3) Matting Agent

In the invention, a matting agent is preferably added to the surface protective layer in order to improve transportability.

Description of the matting agent can be found in paragraphs Nos. 0126 to 0127 of JP-A No. 11-65021.

The addition amount of the matting agent is preferably in a range of from 1 mg/m<sup>2</sup> to 400 mg/m<sup>2</sup>, and more preferably, from 5 mg/m<sup>2</sup> to 300 mg/m<sup>2</sup>, with respect to the coating amount per 1 m<sup>2</sup> of the photothermographic material.

The level of matting on the surface is not restricted as far as star-dust trouble occurs, but the level of matting of from 30 seconds to 2000 seconds is preferred, particularly preferred, 10 from 40 seconds to 1500 seconds as Beck's smoothness. Beck's smoothness can be calculated easily, by using Japan Industrial Standard (JIS) P8119 "The method of testing Beck's smoothness for papers and sheets using Beck's test apparatus", or TAPPI standard method T479.

15 In the present invention, a matting agent is preferably contained in an outermost layer, in a layer which can function as an outermost layer, or in a layer nearer to outer surface of the photothermographic material, and is also preferably contained in a layer which can function as a so-called protective layer.

### 4) Polymer Latex

A polymer latex can be incorporated in the surface protective layer of the photothermographic material according to the present invention.

25 Concerning such polymer latex, descriptions can be found in "Gosei Jushi Emulsion (Synthetic resin emulsion)" (Taira Okuda and Hiroshi Inagaki, Eds., published by Kobunshi Kankokai (1978)), "Gosei Latex no Oyo (Application of synthetic latex)" (Takaaki Sugimura, Yasuo Kataoka, Soichi Suzuki, and Keiji Kasahara, Eds., published by Kobunshi Kankokai (1993)), and "Gosei Latex no Kagaku (Chemistry of synthetic latex)" (Soichi Muroi, published by Kobunshi Kankokai (1970)). More specifically, there can be mentioned a latex of methyl methacrylate (33.5% by weight)/ethyl acrylate (50% by weight)/methacrylic acid (16.5% by weight) copolymer, a latex of methyl methacrylate (47.5% by weight)/butadiene (47.5% by weight)/itaconic acid (5% by weight) copolymer, a latex of ethyl acrylate/methacrylic acid copolymer, a latex of methyl methacrylate (58.9% by weight)/2-ethylhexyl acrylate (25.4% by weight)/styrene (8.6% by weight)/2-hydroxyethyl methacrylate (5.1% by weight)/acrylic acid (2.0% by weight) copolymer, a latex of methyl methacrylate (64.0% by weight)/styrene (9.0% by weight)/butyl acrylate (20.0% by weight)/2-hydroxyethyl methacrylate (5.0% by weight)/acrylic acid (2.0% by weight) copolymer, and the like.

40 The polymer latex in the surface protective layer or the back layer is preferably contained in an amount of from 10% by weight to 90% by weight, particularly preferably, from 20% by weight to 80% by weight of the total weight of binder.

### 5) Surface pH

45 The surface pH of the photothermographic material according to the invention preferably yields a pH of 7.0 or lower, and more preferably, 6.6 or lower, before thermal developing process. Although there is no particular restriction concerning the lower limit, the lower limit of pH value is about 3. Most preferred surface pH range is from 4 to 6.2.

50 From the viewpoint of reducing the surface pH, it is preferred to use an organic acid such as phthalic acid derivative or a non-volatile acid such as sulfuric acid, or a volatile base such as ammonia for the adjustment of the surface pH. In particular, ammonia can be used favorably for the achievement of low surface pH, because it can easily vaporize to remove it before the coating step or before applying thermal development.

55 It is also preferred to use a non-volatile base such as sodium hydroxide, potassium hydroxide, lithium hydroxide, and the

like, in combination with ammonia. The method of measuring surface pH value is described in paragraph No. 0123 of the specification of JP-A No. 2000-284399.

6) Hardener

A hardener may be used in each of the image forming layer, protective layer, back layer, and the like.

As examples of the hardener, descriptions of various methods can be found in pages 77 to 87 of T. H. James, "THE THEORY OF THE PHOTOGRAPHIC PROCESS, FOURTH EDITION" (Macmillan Publishing Co., Inc., 1977). Preferably used are, in addition to chromium alum, sodium salt of 2,4-dichloro-6-hydroxy-s-triazine, N,N-ethylene bis(vinylsulfonacetamide), and N,N-propylene bis(vinylsulfonacetamide), polyvalent metal ions described in page 78 of the above literature and the like, polyisocyanates described in U.S. Pat. No. 4,281,060, JP-A No. 6-208193 and the like, epoxy compounds of U.S. Pat. No. 4,791,042 and the like, and vinyl sulfone compounds of JP-A No. 62-89048.

The hardener is added as a solution, and the solution is added to the coating solution for protective layer 180 minutes before coating to just before coating, preferably 60 minutes before to 10 seconds before coating. However, so long as the effect of the invention is sufficiently exhibited, there is no particular restriction concerning the mixing method and the conditions of mixing.

As specific mixing methods, there can be mentioned a method of mixing in the tank, in which the average stay time calculated from the flow rate of addition and the feed rate to the coater is controlled to yield a desired time, or a method using static mixer as described in Chapter 8 of N. Harnby, M. F. Edwards, A. W. Nienow (translated by Koji Takahashi) "EKITAI KONGO GIJUTSU (Liquid Mixing Technology)" (Nikkan Kogyo Shinbunsha, 1989), and the like.

7) Surfactant

Concerning the surfactant applicable in the invention, description can be found in paragraph No. 0132 of JP-A No. 11-65021.

In the invention, preferably used are fluorocarbon surfactants. Specific examples of fluorocarbon surfactants can be found in those described in JP-A Nos. 10-197985, 2000-19680, and 2000-214554. Polymer fluorocarbon surfactants described in JP-A 9-281636 can be also used preferably.

For the photothermographic material of the invention, fluorocarbon surfactants described in JP-A No. 2000-206560 are particularly preferably used.

8) Antistatic Agent

The photothermographic material of the invention preferably contains an electrically conductive layer including metal oxides or electrically conductive polymers. The antistatic layer may serve as an undercoat layer, a back surface protective layer, or the like, but can also be placed specially. Specific examples of the antistatic layer in the invention include described in paragraph Nos. 0135 of JP-A No. 11-65021, in JP-A Nos. 56-143430, 56-143431, 58-62646, and 56-120519, and in paragraph Nos. 0040 to 0051 of JP-A No. 11-84573, in U.S. Pat. No. 5,575,957, and in paragraph Nos. 0078 to 0084 of JP-A No. 11-223898.

9) Support

As the transparent support, preferably used is polyester, particularly, polyethylene terephthalate, which is subjected to heat treatment in the temperature range of from 130° C. to 185° C. in order to relax the internal strain caused by biaxial stretching and remaining inside the film, and to remove strain ascribed to heat shrinkage generated during thermal development.

As the support of the photothermographic material used in combination with the ultraviolet light emission screen, PEN

is preferably used, but the present invention is not limited thereto. As PEN, polyethylene-2,6-naphthalate is preferred. The term "polyethylene-2,6-naphthalate" herein means that the structure repeating units essentially may consist of ethylene-2,6-naphthalene dicarboxylate units and also may include un-copolymerized polyethylene-2,6-naphthalene dicarboxylate, and the copolymer comprising 10% or less, and preferably 5% or less, of the structure repeating units modified with the other components and mixtures or constituents of other polymers.

Polyethylene-2,6-naphthalate can be synthesized by reacting a naphthalene-2,6-dicarboxylic acid or functional derivatives thereof, and an ethylene glycol or functional derivatives thereof in the presence of a suitable catalyst at a proper reaction condition. The polyethylene-2,6-naphthalate of the present invention may be copolymerized or blended polymers, where one or more kinds of suitable third component (denaturing agent) is added before the completion of polymerization of the polyethylene-2,6-naphthalate. As the suitable third component, compounds containing a divalent ester forming functional group, for example, dicarboxylic acids such as oxalic acid, adipic acid, phthalic acid, isophthalic acid, terephthalic acid, naphthalene-2,7-dicarboxylic acid, succinic acid, diphenylether dicarboxylic acid, and the like, or lower alkylesters thereof, oxycarboxylic acids such as p-oxybenzoic acid, p-oxyethoxybenzoic acid, or lower alkylesters thereof, and divalent alcohols such as propylene glycol, trimethylene glycol, and the like are described.

Polyethylene-2,6-naphthalate and the modified polymers thereof may include, for example, the polymer where the terminal hydroxy group and/or the carboxyl group is blocked by mono-functional compounds such as benzoic acid, benzoyl benzoic acid, benzyloxy benzoic acid, methoxy polyalkylene glycol, or the like, or the polymer modified with a very small amount of compounds having tri-functional or tetra-functional ester forming group such as glycerine and penta-erthritol in the extent to form linear chain copolymers substantially.

In the case of a photothermographic material for medical use, the transparent support may be colored with a blue dye (for instance, dye-1 described in the Example of JP-A No. 8-240877), or may be uncolored.

Specific examples of the support can be found in paragraph No. 0134 of JP-A No. 11-65021.

As to the support, it is preferred to apply undercoating technology, such as water-soluble polyester described in JP-A No. 11-84574, a styrene-butadiene copolymer described in JP-A No. 10-186565, a vinylidene chloride copolymer described in JP-A No. 2000-39684, and the like.

10) Other Additives

Furthermore, antioxidant, stabilizing agent, plasticizer, UV absorbent, or a film-forming promoting agent may be added to the photothermographic material. Each of the additives is added to either of the image forming layer or the non-photosensitive layer.

Reference can be made to WO No. 98/36322, EP No. 803764A1, JP-A Nos. 10-186567 and 10-18568, and the like.

11) Coating Method

The photothermographic material of the invention may be coated by any method. More specifically, various types of coating operations inclusive of extrusion coating, slide coating, curtain coating, immersion coating, knife coating, flow coating, or an extrusion coating using the kind of hopper described in U.S. Pat. No. 2,681,294 are used. Preferably used is extrusion coating or slide coating described in pages 399 to 536 of Stephen F. Kistler and Peter M. Schweizer,

## 101

"LIQUID FILM COATING" (Chapman & Hall, 1997), and particularly preferably used is slide coating.

Example of the shape of the slide coater for use in slide coating is shown in FIG. 11b.1, page 427, of the same literature. If desired, two or more layers can be coated simultaneously by the method described in pages 399 to 536 of the same literature, or by the method described in U.S. Pat. No. 2,761,791 and British Patent No. 837095.

The coating solution for the image forming layer in the invention is preferably a so-called thixotropic fluid. Concerning this technology, reference can be made to JP-A No. 11-52509.

Viscosity of the coating solution for the image forming layer of the invention at a shear velocity of  $0.1 \text{ S}^{-1}$  is preferably from 400 mPa·s to 100,000 mPa·s, and more preferably, from 500 mPa·s to 20,000 mPa·s.

At a shear velocity of  $1000 \text{ S}^{-1}$ , the viscosity is preferably from 1 mPa·s to 200 mPa·s, and more preferably, from 5 mPa·s to 80 mPa·s.

## 12) Wrapping Material

In order to suppress fluctuation from occurring on the photographic property during a preservation of the photothermographic material of the invention before use, or in order to improve curling or winding tendencies when the photothermographic material is manufactured in a roll state, it is preferred that a wrapping material having low oxygen transmittance and/or vapor transmittance is used. Preferably, oxygen transmittance is  $50 \text{ mL} \cdot \text{atm}^{-1} \text{m}^{-2} \text{day}^{-1}$  or lower at  $25^\circ \text{C}$ ., more preferably,  $10 \text{ mL} \cdot \text{atm}^{-1} \text{m}^{-2} \text{day}^{-1}$  or lower, and further preferably,  $1.0 \text{ mL} \cdot \text{atm}^{-1} \text{m}^{-2} \text{day}^{-1}$  or lower. Preferably, vapor transmittance is  $10 \text{ g} \cdot \text{atm}^{-1} \text{m}^{-2} \text{day}^{-1}$  or lower, more preferably,  $5 \text{ g} \cdot \text{atm}^{-1} \text{m}^{-2} \text{day}^{-1}$  or lower, and further preferably,  $1 \text{ g} \cdot \text{atm}^{-1} \text{m}^{-2} \text{day}^{-1}$  or lower. As specific examples of a wrapping material having low oxygen transmittance and/or vapor transmittance, reference can be made to, for instance, the wrapping material described in JP-A Nos. 8-254793 and 2000-206653.

## 13) Other Applicable Techniques

Techniques which can be used for the photothermographic material of the invention also include those in EP No. 803764A1, EP No. 883022A1, WO No. 98/36322, JP-A Nos. 56-62648, and 58-62644, JP-A Nos. 09-43766, 09-281637, 09-297367, 09-304869, 09-311405, 09-329865, 10-10669, 10-62899, 10-69023, 10-186568, 10-90823, 10-171063, 10-186565, 10-186567, 10-186569 to 10-186572, 10-197974, 10-197982, 10-197983, 10-197985 to 10-197987, 10-207001, 10-207004, 10-221807, 10-282601, 10-288823, 10-288824, 10-307365, 10-312038, 10-339934, 11-7100, 11-15105, 11-24200, 11-24201, 11-30832, 11-84574, 11-65021, 11-109547, 11-125880, 11-129629, 11-133536 to 11-133539, 11-133542, 11-133543, 11-223898, 11-352627, 11-305377, 11-305378, 11-305384, 11-305380, 11-316435, 11-327076, 11-338096, 11-338098, 11-338099, and 11-343420, JP-A Nos. 2000-187298, 2001-200414, 2001-234635, 2002-20699, 2001-275471, 2001-275461, 2000-313204, 2001-292844, 2000-324888, 2001-293864, and 2001-348546.

## 3. Image Forming Method

An image is formed by subjecting the photothermographic material of the invention to exposure and thermally development with a thermal developing apparatus having a heating means.

## 3-1. Temperature and Time Period for Thermal Development

Although any method may be used for the development of the photothermographic material of the invention, the thermal developing process is usually performed by elevating the

## 102

temperature of the photothermographic material exposed imagewise. The temperature for the development is preferably in a range of from  $80^\circ \text{C}$ . to  $250^\circ \text{C}$ ., more preferably from  $100^\circ \text{C}$ . to  $140^\circ \text{C}$ ., and even more preferably from  $110^\circ \text{C}$ . to  $130^\circ \text{C}$ . Time period for development is preferably in a range of from 1 second to 60 seconds, more preferably from 3 seconds to 30 seconds, even more preferably from 5 seconds to 25 seconds, and particularly preferably from 7 seconds to 15 seconds.

## 3-2. Thermal Developing Apparatus

Preferred embodiments of a thermal developing method and a thermal developing apparatus used for the present invention are explained hereinafter in detail with reference to the attached drawings.

Symbols used in Figures are explained below.

31: Support

33a: First surface

33b: Second surface

35: Image forming layer

44: Preheating means

49a, 81a, 91a, 101a: First heating means

49b, 81b, 91b, 101b: Second heating means

51: Plate

53: Pressing roller

83: Drum

85: Pressing roller

95: Endless belt

97: Pressing roller

100, 200, 300, 400: Thermal developing apparatus

A: Recording material (photosensitive photothermographic material)

C: Conveying route

H: Heater

T: Development reaction temperature

δ: Clearance

FIG. 1 is a structural diagram illustrating a first embodiment of a thermal developing apparatus for practicing the present invention. FIG. 2 is a sectional view showing the photothermographic material of the present invention. FIG. 3 is an explanatory diagram indicating a correlation between temperatures of the back and front surfaces of a recording material respectively heated by first and second heating means and time. FIG. 4 is a block diagram showing a control means.

The thermal developing apparatus 100 according to the embodiment of the present invention heats the photothermographic material A to make visible the latent image recorded in the image forming layer. The photothermographic material A used for the thermal developing apparatus 100 comprises image forming layers 35, 35 coated both on a first surface 33a as one side of the support 31 and the other face, a second surface 33b as shown in FIG. 2.

In the thermal developing apparatus 100, for example, when a fluorescent intensifying screen (not shown) is placed on both sides of the first surface 33a and the second surface 33b of the photothermographic material A, the photothermographic material A can be used for the direct radiography. The fluorescent intensifying screen can emit a fluorescent light by exposure to X-ray beam. The image forming layers 35, 35 coated on the first surface 33a and the second surface 33b respectively have a sensitivity to the fluorescent light emitted by the fluorescent intensifying screen and then can be sensitized by a small amount of X-ray beam thereby.

The photothermographic material A having a latent image in the image forming layer 35 is usually stocked in a cassette 37 one by one, and the cassette 37 including the materials is

## 103

loaded to the thermal developing apparatus 100. An opening and closing cover 39 of the cassette 37 loaded in the thermal developing apparatus 100 is opened and the photothermographic material A included is taken out from the cassette by means of a suction cup 41.

Further, the thermal developing apparatus 100 may have a structure of a magazine (not shown) where a plurality of the photothermographic materials A are accommodated together. In this case, each of the photothermographic material A having a latent image is taken out from the cassette 37 in a darkroom and then stacked in the magazine. The photothermographic material A stacked and accommodated in the magazine is taken out one by one by means of the suction cup 41. In place of the suction cup 41, a pick-up roller can be applied.

The thermal developing apparatus 100 may have a structure where the photothermographic material A having a latent image is taken out from the cassette 37 manually in a darkroom and then directly inserting it into a conveying roller pair 43.

The photothermographic material A taken out thereby is conveyed to a thermal developing section 47 located downstream to a travelling direction via a conveying roller pair 43 and a transporting guide 45. A width aligning portion which aligns the photothermographic material A taken out in the direction normal to that of the travelling direction and the position of the photothermographic material A in the thermal developing section 47 located downstream may be installed between the conveying roller pair 43 and the thermal developing section 47.

In the thermal developing section 47, a first heating means 49a for heating the first surface 33a of the photothermographic material A and a second heating means 49b for heating the second surface 33b of the photothermographic material A are equipped alternatively crossing the conveying route C of the photothermographic material A. According to the embodiment, the first heating means 49a and the second heating means 49b are composed of a plate 51 and rotary pressing rollers 53 to push the photothermographic material A against the plate 51. Either the plate 51 or the pressing rollers 53 may include a heater as a heating source.

According to the embodiment, the heater as a heating source is included in the plate 51. Therefore, in the first heating means 49a, the plate 51 is placed facing the first surface 33a of the photothermographic material A, and in the second heating means 49b, the plate 51 is placed facing the second surface 33b of the photothermographic material A. The first surface 33a and the second surface 33b may be heated alternatively thereby. The term "heated alternatively" used herein includes a heating method where the first surface 33a is heated at first, thereafter the second surface 33b is heated, and finish heating, that is the case where the back and front sides of the material are heated only one time respectively.

The plate 51 has a circular-arc configuration and install a plurality of the pressing rollers 53 along the inner side. The photothermographic material A is inserted to the conveying route C formed in a clearance between the plate 51 and the pressing rollers 53, and conveyed tightly in contact with the plate 51 while pushing against the plate 51 by the pressing rollers 53. And then the material A is developed by the heat of the plate 51.

The heating source for the plate 51 is not particularly restricted, but a heat generating body such as a nichrome wire, a light source such as a halogen lamp, hot air heating or other well-known heating means can be applied.

## 104

The pressing rollers 53 are selected from a metal roller, a heat-resistant resin roller, a heat-resistant rubber roller, and the like. Overall region in the plate 51, it is preferable to install a plurality of the rollers.

According to the thermal developing section 47, in the first heating means 49a, wherein the second surface 33b of the photothermographic material A is pushed by the pressing rollers 53, the first surface 33a is pushed against the plate 51. Thereafter the photothermographic material A is conveyed to the second heating means 49b, wherein the first surface 33a is pushed by the pressing rollers 53, the second surface 33b is pushed against the plate 51. As the result, the first surface 33a and the second surface 33b of the photothermographic material A are heated alternatively. Thereby, the rapid temperature raise of the photothermographic material A can be avoided and also uniform heating of both surfaces can be attained. In addition, the above-mentioned configuration has an advantage of decreasing the movable parts and miniaturizing the apparatus structure, because the pressing roller 53 rotates alone.

In the thermal developing section 47, with respect to the total heating amount which is more than the development reaction temperature for the image forming layer 35 heated by the first surface 33a and the second surface 33b of the photothermographic material A, if the total heating amount for the first surface 33a is taken as 100, the total heating amount for the second surface 33b is set to be in a range of 100±30.

The temperature of both the first heating means 49a and the second heating means 49b is set at the glass transition temperature of the photothermographic material A or higher. The temperature of the heating means (the first heating means 49a) located upstream to the travelling direction of the photothermographic material A is set a lower temperature than that of the heating means (the second heating means 49b) located downstream to the travelling direction.

The above-mentioned total heating amount can be derived from the integral value of the temperature of greater than the development reaction temperature and the time lapse from the time when the temperature is reached to the development reaction temperature. Namely, in the graph shown in FIG. 3, the total heating amount of the first surface 33a can be obtained from the area S<sub>1</sub> which is enclosed between the line segment T<sub>0</sub> representing the development reaction temperature T and the curve K<sub>1</sub> representing the temperature change of the first surface 33a. The total heating amount of the second surface 33b can be obtained from the area S<sub>2</sub> which is enclosed between the line segment T<sub>0</sub> representing the development reaction temperature T and the curve K<sub>2</sub> representing the temperature change of the second surface 33b.

Thereby, the total heating amount can be controlled by the specific parameters of the temperature and the time lapse for the first heating means 49a and the second heating means 49b, because the total heating amount (S<sub>1</sub>, S<sub>2</sub>) on the first surface 33a and the second surface 33b can be determined from the integral value of the temperature and the time lapse respectively. As the result, uniformity of the total heating amount on both surfaces of the photothermographic material A can be easily attained.

Further, concerning the total heating amount, if the heating temperature of the first heating means 49a and the second heating means 49b and a contact length L<sub>1</sub>, L<sub>2</sub> of the photothermographic material A with the first heating means 49a and the second heating means 49b are used as a parameter, and the total heating amount on the first surface 33a is taken as 100, then the total heating amount on the second surface 33b may be set to a range of 100±30. Thereby, the total

## 105

heating amount can be controlled by the specific parameter of the temperature and the contact length L1, L2, and then the uniformity of the total heating amount on both surfaces of the photothermographic material A can be easily attained.

According to the above configuration, the temperature of the photothermographic material A becomes the glass transition temperature or higher when the heating face is the first surface 33a, and also the temperature becomes the glass transition temperature or higher when the heating face is transferred from the first surface 33a to the second surface 33b. Therefore the photothermographic material A is maintained to be in a softening state during the heating process. Thereby, the generation of a wrinkle caused by pushing the photothermographic material A by the pressing rollers 53 can be prevented. Because the heating temperature of the first heating means 49a is set to be lower than the heating temperature of the second heating means 49b, the rapid temperature rise on the first surface 33a is avoided at the beginning stage of the heating. The generation of a wrinkle caused by a rapid thermal swelling of the photothermographic material A can be prevented thereby.

Furthermore, in the thermal developing section 47, the clearance  $\delta$  between the first heating means 49a and the second heating means 49b is set to 100 mm or less. Therefore, when the photothermographic material A whose first surface 33a is heated by the heating means 49a is conveyed to the second heating means 49b to heat the second surface 33b, the temperature drop of the photothermographic material A heated by the first heating means 49a is prevented because of the narrow clearance on the order of 100 mm or less.

Thereby, the photothermographic material A is kept at more than the predetermined temperature shown in FIG. 3, even if the heating face is changed between the back and front sides, and the development reaction can proceed successively without any delay.

The photothermographic material A developed in the thermal developing section 47 is then conveyed to a gradual cooling section 61 located downstream to the travelling direction as shown in FIG. 1. The gradual cooling section 61 installs a plurality of cooling roller pairs 63 and can gradually cool the thermally developed photothermographic material A. The photothermographic material A cooled in the gradual cooling section 61 is then conveyed to the downstream direction by a discharging roller pairs 65, and 67 and then discharged to a tray 69.

The thermal developing apparatus 100 also includes a control section 71 which can control the first heating means 49a, the second heating means 49b and the transporting speed of the photothermographic material A. As shown in FIG. 4, the control section 71 can control the first heating means 49a via the first temperature-setting portion 73, the second heating means 49b via the second temperature-setting portion 75.

And, the control section 71 can also control a driving portion for transportation 79 such as a driving motor via a transporting speed-setting portion 77. The control section 71 can control the total heating amount for heating the first surface 33a and the second surface 33b to be in the above described range using the temperature and the transporting speed as the parameter.

According to the thermal developing apparatus 100, the first surface 33a of the photothermographic material A may be heated first, and then the second surface 33b is heated. Therefore, the both surfaces of the photothermographic material A can be thermally developed, while suppressing a rapid temperature raise. Also, because the total heating amount of the second surface 33b is set to be in the prescribed range of the total heating amount of the first surface 33a, the total

## 106

heating amount of both surfaces of the photothermographic material A result in an approximately equal amount. Thereby, the photothermographic material A can be thermally developed evenly without any wrinkle generation, color tone difference and density fluctuation.

According to the thermal developing method using the thermal developing apparatus 100, the first surface 33a and the second surface 33b of the photothermographic material A are heated alternatively, and with respect to each of the total heating amount which is more than the development reaction temperature to the image forming layer 35 heated by the first surface 33a and the second surface 33b, if the total heating amount of the first surface 33a is taken as 100, the total heating amount of the second surface 33b is set to be in the range of 100±30. Thereby, both sides of the photothermographic material A are heated evenly and then can be thermally developed uniformly. In addition, even if the first surface 33a and the second surface 33b are heated alternatively, both surfaces can be heated evenly while suppressing a rapid temperature raise. Thereby, for the case of the photothermographic material A which has an image forming layer on both sides, uniformly heat development of both surfaces can be attained without the generation of wrinkles, and also without color tone difference and density fluctuation. The loading of the photothermographic material A to the thermal developing apparatus and the development thereof can be carried out without any consideration about the back and front sides.

The other embodiments of the thermal developing apparatus used for the present invention are explained hereinafter.

In the following embodiments, only the main portions of the thermal developing apparatus (thermal developing section) are shown. Every thermal developing section has a construction where the first surface 33a and the second surface 33b of the photothermographic material A are heated alternatively by the first heating means and the second heating means respectively, and the total heating amount of the second surface 33b is set to be in a range of 100±30 when the total heating amount of the first surface 33a is taken as 100.

FIG. 5 show a schematic diagram of a main portion of a thermal developing apparatus installed with a drum and a plurality of pressing rollers according to the second embodiment.

The thermal developing apparatus 200 has a construction in which both of a first heating means 81a and a second heating means 81b use a rotary driven cylindrical drum 83 and a plurality of rotary pressing rollers 85 pushing the photothermographic material A against the circumferential surface of the drum 83. A heater as a heating source may be equipped in either the drum 83 or the pressing rollers 85. In this embodiment, the drum 83 contains the heater as the heating source.

The first heating means 81a and the second heating means 81b are disposed close together, and the drum 83 of the first heating means 81a rotates reversely to the drum 83 of the second heating means 81b. Therefore, the first heating means 81a and the second heating means 81b form an S-shaped conveying route C. Even in the thermal developing apparatus 200 according to the embodiment, the first surface 33a of the photothermographic material A is heated by the first heating means 81a and then the second surface 33b is heated by the second heating means 81b.

The photothermographic material A transported by the first heating means 81a is conveyed with nipping by the drum 83 and the pressing rollers 85 while the first surface 33a is conveyed in close contact with the drum 83. As a result, the material is heated by the heat of the drum 83 to make visible the latent image formed by the exposure. Next to the above, the photothermographic material A in which the first surface

33a is heated is conveyed to the second heating means 81b, and then conveyed with nipping by the drum 83 and the pressing rollers 85 while the second surface 33b is conveyed in close contact with the drum 83 in a similar way as the above. Thereby the material is thermally developed by the heat of the drum 83.

According to the thermal developing apparatus 200, the first surface 33a of the photothermographic material A is pushed against the drum 83 in the heating means 81a, and then the second surface 33b is pushed against the drum 83 in the second heating means 81b. As a result, the first surface 33a and the second surface 33b of the photothermographic material A are heated alternatively. Therefore, the rapid temperature raise of the photothermographic material A can be avoided and then the uniform heating of both faces is attained. Also, a configuration where the drum 83 and the pressing rollers 85 are rotated synchronously with the transporting speed of the photothermographic material A advantageously results in no rubbing between the heating means and the photothermographic material A.

The thermal developing apparatus of the third embodiment of the present invention is explained hereinafter.

FIG. 6 shows a schematic diagram of the main portion of a thermal developing apparatus having a carrier, an endless belt and a pressing roller.

The thermal developing apparatus 300 has a construction in which each of the first heating means 91a and the second heating means 91b consist of a pipe type carrier 93 installed with a heater H as a heat source, the endless belt 95 surrounding the carrier 93, and the pressing roller 97 rotating the endless belt 95 at the same speed while pushing the endless belt 95 against the carrier 93. The endless belt 95 may be made of a material having enough heat conductivity such as aluminum, resin and the like, or a rubber heater. With respect to the heating amount of the first heating means 91a and the second heating means 91b, if each heating means is adjusted to heat the back and front surfaces of the photothermographic material A evenly, the number of the first heating means 91a and the heating means 91b disposed is not necessary the same.

According to the thermal developing apparatus 300, for example, in the heating means 91a shown in the left side of FIG. 6, while pushing the second surface 33b of the photothermographic material A by the pressing roller 97, the first surface 33a is pushed against the carrier 93 by means of the endless belt 95. Then the photothermographic material A is conveyed to the second heating means 91b, in succession, while pushing the first surface 33a by the pressing roller 97, the second surface 33b is pushed against the carrier 93 by means of the endless belt 95. Thereby, the first surface 33a and the second surface 33b of the photothermographic material A are heated alternatively. Both surfaces of the photothermographic material A can be heated uniformly, and the gradual heating with the plural heating means prevents the rapid temperature raise. And also, the configuration in which the endless belt 95 surrounding the carrier 93 is moved synchronized with the transporting speed of the photothermographic material A may result in no rubbing between the heating means and the photothermographic material A. Therefore no damage in the image forming layer is occurred.

The thermal developing apparatus of the fourth embodiment of the present invention will be explained in detail hereinafter.

FIG. 7 shows a schematic diagram of a main portion of the thermal developing apparatus installed with plural sets of a first heating means and a second heating means.

The thermal developing apparatus 400 installs plural sets of a first heating means 101a composed of a heating roller 101 along the conveying route C of the photothermographic material A and a second heating means 101b composed of similar heating roller 101. The heating roller 101 consists of a cylindrical heating body 103 and a heating source 105 such as a halogen heater and the like to heat the inner side of the heating body 103.

Especially, according to the embodiment, the first heating means 101a and the second heating means 101b are disposed in the staggered form along the conveying route C of the photothermographic material A.

Therefore, according to the thermal developing apparatus 400, after the first surface 33a and the second surface 33b of the photothermographic material A are heated alternatively by the first heating means 101a and the second heating means 101b of the first set respectively, the photothermographic material A is conveyed to the first heating means 101a and the second heating means 101b of the second set where the first surface 33a and the second surface 33b is again heated alternatively. This alternative heating is repeated in the plural sets of the heating means. Thereby, a rapid temperature raise in the photothermographic material A can be avoided and also both surfaces of the photothermographic material A can be heated uniformly with gradually heating.

The thermal developing apparatus 400 in which plural sets of the first heating means 101a and the heating means 101b are disposed in the staggered form along the conveying route C has the configuration where a plurality of the first heating means 101a disposed on the one side of the conveying route C and a plurality of the second heating means 101b disposed on the other side of the conveying route C are inserted alternatively in the gap between the neighboring heating means and disposed with some contact angle to each heating means. Therefore, the conveying route C is formed as a wavy shape. Thereby, the contact area between the photothermographic material A and the heating means is increased, the efficiency of the heat conductance to the photothermographic material A is enhanced.

In each embodiment described above, only main part of the thermal developing apparatus (i.e., thermal developing section) is shown. However, similar heating means can be selected for the preheating means 44 in the diagram showing the first embodiment of the thermal developing apparatus shown in FIG. 1 according to the present invention. As for a heating means for the preheating section, the known heating means, for example, such as a hot air method can be selected.

#### 4. Application of the Invention

The photothermographic material of the invention is preferably employed as photothermographic materials for use in medical diagnosis.

The present invention is specifically explained by way of Examples below, which should not be construed as limiting the invention thereto.

#### EXAMPLES

##### Example 1

###### 1. Preparation of PET Support and Undercoating

###### 1-1. Film Manufacturing

PET having IV (intrinsic viscosity) of 0.66 (measured in phenol/tetrachloroethane=6/4 (weight ratio) at 25° C.) was obtained according to a conventional manner using terephthalic acid and ethylene glycol. The product was pelletized,

109

dried at 130° C. for 4 hours, and colored blue with the blue dye (1,4-bis(2,6-diethylanilinoanthraquinone). Thereafter, the mixture was extruded from a T-die and rapidly cooled to form a non-tentered film.

The film was stretched along the longitudinal direction by 3.3 times using rollers of different peripheral speeds, and then stretched along the transverse direction by 4.5 times using a tenter machine. The temperatures used for these operations were 110° C. and 130° C., respectively. Then, the film was subjected to thermal fixation at 240° C. for 20 seconds, and relaxed by 4% along the transverse direction at the same temperature. Thereafter, the chucking part was slit off, and both edges of the film were knurled. Then the film was rolled up at the tension of 4 kg/cm<sup>2</sup> to obtain a roll having the thickness of 175 µm.

#### 1-2. Surface Corona Discharge Treatment

Both surfaces of the support were treated at room temperature at 20 m/minute using Solid State Corona Discharge Treatment Machine Model 6 KVA manufactured by Piller GmbH. It was proven that treatment of 0.375 KV·A·minute<sup>1/2</sup>·m<sup>2</sup> was executed, judging from the readings of current and voltage on that occasion. The frequency upon this treatment was 9.6 kHz, and the gap clearance between the electrode and dielectric roll was 1.6 mm.

#### 1-3. Undercoating

|                                                                                                                               |        |
|-------------------------------------------------------------------------------------------------------------------------------|--------|
| Pesresin A-520 manufactured by Takamatsu Oil & Fat Co., Ltd. (30% by weight solution)                                         | 46.8 g |
| BAIRONAARU WD-1200 manufactured by Toyo Boseki Co., Ltd.                                                                      | 10.4 g |
| Polyethylene glycol monononylphenylether (average ethylene oxide number = 8.5) 1% by weight solution                          | 11.0 g |
| MP-1000 manufactured by Soken Chemical & Engineering Co., Ltd. (PMMA polymer fine particle, mean particle diameter of 0.4 µm) | 0.91 g |
| distilled water                                                                                                               | 931 mL |

Both surfaces of the aforementioned biaxially tentered polyethylene terephthalate support having the thickness of 175 µm were subjected to the corona discharge treatment as described above. Thereafter, the coating solution for the undercoat was coated with a wire bar so that the amount of wet coating became 6.6 mL/m<sup>2</sup> (per one side), and dried at 180° C. for 5 minutes. Thus, an undercoated support was produced.

#### 2. Image Forming Layer, Intermediate Layer, and Surface Protective-Layer

##### 2-1. Preparations of Coating Material

###### 1) Preparation of Silver Halide Emulsion

<Preparation of Silver Halide Emulsion A (Silver Iodobromide Emulsion Having Fine Grains)>

A solution was prepared by adding 3.1 mL of a 1% by weight potassium bromide solution, and then 3.5 mL of 0.5 mol/L sulfuric acid and 35.5 g of phthalated gelatin to 1421 mL of distilled water. The solution was kept at 35° C. while stirring in a stainless steel reaction vessel, and thereto were added total amount of: solution A prepared through diluting 22.22 g of silver nitrate by adding distilled water to give the volume of 95.4 mL; and solution B prepared through diluting 15.3 g of potassium bromide and 0.8 g of potassium iodide with distilled water to give the volume of 97.4 mL, over 45 seconds at a constant flow rate.

110

Thereafter, 10 mL of a 3.5% by weight aqueous solution of hydrogen peroxide was added thereto, and 10.8 mL of a 10% by weight aqueous solution of benzimidazole was further added. Moreover, a solution C prepared through diluting 51.86 g of silver nitrate by adding distilled water to give the volume of 317.5 mL and a solution D prepared through diluting 44.2 g of potassium bromide and 2.2 g of potassium iodide with distilled water to give the volume of 400 mL were added. A controlled double jet method was executed through adding 10 total amount of the solution C at a constant flow rate over 20 minutes, accompanied by adding the solution D while maintaining the pAg at 8.1. Potassium hexachloroiridate (III) was added in its entirety to give 1×10<sup>-4</sup> mol per 1 mol of silver, at 15 10 minutes post initiation of the addition of the solution C and the solution D.

Moreover, at 5 seconds after completing the addition of the solution C, a potassium hexacyanoferate (II) in an aqueous solution was added in its entirety to give 3×10<sup>-4</sup> mol per 1 mol of silver. The mixture was adjusted to the pH of 3.8 with 0.5 mol/L sulfuric acid. After stopping stirring, the mixture was subjected to precipitation/desalting/water washing steps. The mixture was adjusted to the pH of 5.9 with 1 mol/L sodium hydroxide to produce a silver halide dispersion having the pAg of 8.0.

25 The above-described silver halide dispersion was kept at 38° C. with stirring, and thereto was added 5 mL of a 0.34% by weight methanol solution of 1,2-benzisothiazoline-3-one, followed by elevating the temperature to 47° C. at 40 minutes thereafter. At 20 minutes after elevating the temperature, 30 sodium benzene thiosulfonate in a methanol solution was added at 7.6×10<sup>-5</sup> mol per 1 mol of silver. At additional 5 minutes later, a tellurium sensitizer C in a methanol solution was added at 2.9×10<sup>-4</sup> mol per 1 mol of silver and subjected to ripening for 91 minutes. At one minute later, 1.3 mL of a 35 0.8% by weight methanol solution of N,N'-dihydroxy-N",N"-diethylmelamine was added thereto, and at additional 4 minutes thereafter, 5-methyl-2-mercaptopbenzimidazole in a methanol solution at 4.8×10<sup>-3</sup> mol per 1 mol of silver, 1-phenyl-2-heptyl-5-mercaptop-1,3,4-triazole in a methanol solution at 5.4×10<sup>-3</sup> mol per 1 mol of silver, and 1-(3-methylureidophenyl)-5-mercaptopetrazole in an aqueous solution at 40 8.5×10<sup>-3</sup> mol per 1 mol of silver were added to produce a silver halide emulsion A.

45 Grains in thus prepared silver halide emulsion were silver iodobromide grains having a mean equivalent spherical diameter of 0.06 µm, a variation coefficient of an equivalent spherical diameter distribution of 20%, which uniformly include iodine at 3.5 mol %. Grain size and the like were determined from the average of 1000 grains using an electron microscope. The {100} face ratio of these grains was found to be 80% using a Kubelka-Munk method.

###### <Preparations of Emulsion for Coating Solution>

The silver halide emulsion A was dissolved and thereto was added benzothiazolium iodide in a 1% by weight aqueous solution at 7×10<sup>-3</sup> mol per 1 mol of silver. Further, as "a compound that can be one-electron-oxidized to provide a one-electron oxidation product, which releases one or more electrons", the compounds Nos. 1, 2, and 3 were added respectively in an amount of 2×10<sup>-3</sup> mol per 1 mol of silver in silver halide. Thereafter, as "a compound having an adsorptive group and a reducing group", the compound Nos. 1 and 2 were added respectively in an amount of 8×10<sup>-3</sup> mol per 1 mol of silver halide.

60 65 Further, water was added thereto to give the content of silver halide of 15.6 g in terms of silver, per 1 liter of the emulsion for a coating solution.

2) Preparation of Dispersion of Silver Salt of Fatty Acid  
<Preparation of Recrystallized Behenic Acid>

Behenic acid manufactured by Henkel Co. (trade name: Edenor C22-85R) in an amount of 100 kg was admixed with 1200 kg of isopropyl alcohol, and dissolved at 50° C. The mixture was filtrated through a 10  $\mu\text{m}$  filter, and cooled to 30° C. to allow recrystallization. Cooling speed for the recrystallization was controlled to be 3° C./hour. The resulting crystal was subjected to centrifugal filtration, and washing was performed with 100 kg of isopropyl alcohol. Thereafter, the crystal was dried. The resulting crystal was esterified, and subjected to GC-FID analysis to give the results of the content of behenic acid being 96 mol %, lignoceric acid 2 mol %, and arachidic acid 2 mol %. In addition, erucic acid was included at 0.001 mol %.

## &lt;Preparation of Dispersion of Silver Salt of Fatty Acid&gt;

88 kg of the recrystallized behenic acid, 422 L of distilled water, 49.2 L of 5 mol/L sodium hydroxide aqueous solution, 120 L of t-butyl alcohol were admixed, and subjected to a reaction with stirring at 75° C. for one hour to give a solution of sodium behenate. Separately, 206.2 L of an aqueous solution of 40.4 kg of silver nitrate (pH 4.0) was provided, and kept at a temperature of 10° C. A reaction vessel charged with 635 L of distilled water and 30 L of t-butyl alcohol was kept at 30° C., and thereto were added the total amount of the solution of sodium behenate and the total amount of the aqueous silver nitrate solution with sufficient stirring at a constant flow rate over 93 minutes and 15 seconds, and 90 minutes, respectively.

Upon this operation, during first 11 minutes following the initiation of adding the aqueous silver nitrate solution, the added material was restricted to the aqueous silver nitrate solution alone. The addition of the solution of sodium behenate was thereafter started, and during 14 minutes and 15 seconds following the completion of adding the aqueous silver nitrate solution, the added material was restricted to the solution of sodium behenate alone.

The temperature inside of the reaction vessel was then set to be 30° C., and the temperature outside was controlled so that the liquid temperature could be kept constant. In addition, the temperature of a pipeline for the addition system of the solution of sodium behenate was kept constant by circulation of warm water outside of a double wall pipe, so that the temperature of the liquid at an outlet in the leading edge of the nozzle for addition was adjusted to be 75° C. Further, the temperature of a pipeline for the addition system of the aqueous silver nitrate solution was kept constant by circulation of cool water outside of a double wall pipe. Position at which the solution of sodium behenate was added and the position, at which the aqueous silver nitrate solution was added, was arranged symmetrically with a shaft for stirring located at a center. Moreover, both of the positions were adjusted to avoid contact with the reaction liquid.

After completing the addition of the solution of sodium behenate, the mixture was left to stand at the temperature as it was for 20 minutes. The temperature of the mixture was then elevated to 35° C. over 30 minutes followed by ripening for 210 minutes. Immediately after completing the ripening, solid matters were filtered out with centrifugal filtration. The solid matters were washed with water until the electric conductivity of the filtrated water became 30  $\mu\text{S}/\text{cm}$ . A silver salt of fatty acid was thus obtained. The resulting solid matters were stored as a wet cake without drying.

When the shape of the resulting particles of the silver behenate was evaluated by an electron micrography, a crystal was revealed having  $a=0.21 \mu\text{m}$ ,  $b=0.4 \mu\text{m}$  and  $c=0.4 \mu\text{m}$  on the average value, with a mean aspect ratio of 2.1, and a

variation coefficient of an equivalent spherical diameter distribution of 11% (a, b and c are as defined aforementioned.).

To the wet cake corresponding to 260 kg of a dry solid matter content, were added 19.3 kg of poly(vinyl alcohol) (trade name: PVA-217) and water to give the total amount of 1000 kg. Then, a slurry was obtained from the mixture using a dissolver blade. Additionally, the slurry was subjected to preliminary dispersion with a pipeline mixer (manufactured by MIZUHO Industrial Co., Ltd.: PM-10 type).

Next, a stock liquid after the preliminary dispersion was treated three times using a dispersing machine (trade name: Microfluidizer M-610, manufactured by Microfluidex International Corporation, using Z type Interaction Chamber) with the pressure controlled to be 1150 kg/cm<sup>2</sup> to give a dispersion of the silver behenate. For the cooling manipulation, coiled heat exchangers were equipped in front of and behind the interaction chamber respectively, and accordingly, the temperature for the dispersion was set to be 18° C. by regulating the temperature of the cooling medium.

## 3) Preparation of Reducing Agent Dispersion

## &lt;Preparation of Reducing Agent-1 Dispersion&gt;

To 10 kg of reducing agent-1 (1,1-bis(2-hydroxy-3,5-dimethylphenyl)-3,5,5-trimethylhexane) and 16 kg of a 10% by weight aqueous solution of modified poly(vinyl alcohol) (manufactured by Kuraray Co., Ltd., Poval MP203) is added 10 kg of water, and thoroughly mixed to give a slurry. This slurry is fed with a diaphragm pump, and is subjected to dispersion with a horizontal sand mill (UVM-2: manufactured by AIMEX Co., Ltd.) packed with zirconia beads having a mean particle diameter of 0.5 mm for 3 hours. Thereafter, 0.2 g of a benzisothiazolinone sodium salt and water are added thereto, thereby adjusting the concentration of the reducing agent to be 25% by weight. This dispersion is subjected to heat treatment at 60° C. for 5 hours to obtain reducing agent-1 dispersion. Particles of the reducing agent included in the resulting reducing agent dispersion have a median diameter of 0.40  $\mu\text{m}$ , and a maximum particle diameter of 1.4  $\mu\text{m}$  or less. The resultant reducing agent dispersion is subjected to filtration with a polypropylene filter having a pore size of 3.0  $\mu\text{m}$  to remove foreign substances such as dust, and stored.

## 4) Preparation of Hydrogen Bonding Compound Dispersion

To 10 kg of hydrogen bonding compound-1 (tri(4-t-butylphenyl)phosphineoxide) and 16 kg of a 10% by weight aqueous solution of modified poly(vinyl alcohol) (manufactured by Kuraray Co., Ltd., Poval MP203) was added 10 kg of water, and thoroughly mixed to give a slurry. This slurry was fed with a diaphragm pump, and was subjected to dispersion with a horizontal sand mill (UVM-2: manufactured by AIMEX Co., Ltd.) packed with zirconia beads having a mean particle diameter of 0.5 mm for 4 hours. Thereafter, 0.2 g of a benzisothiazolinone sodium salt and water were added thereto, thereby adjusting the concentration of the hydrogen bonding compound to be 25% by weight.

This dispersion was warmed at 40° C. for one hour, followed by a subsequent heat treatment at 80° C. for one hour to obtain hydrogen bonding compound-1 dispersion. Particles of the hydrogen bonding compound included in the resulting hydrogen bonding compound dispersion had a median diameter of 0.45  $\mu\text{m}$ , and a maximum particle diameter of 1.3  $\mu\text{m}$  or less. The resultant hydrogen bonding compound dispersion was subjected to filtration with a polypropylene filter having a pore size of 3.0  $\mu\text{m}$  to remove foreign substances such as dust, and stored.

## 5) Preparations of Dispersions of Development Accelerator and Color-Tone-Adjusting Agent

## &lt;Preparation of Development Accelerator-1 Dispersion&gt;

To 10 kg of development accelerator-1 and 20 kg of a 10% by weight aqueous solution of modified poly(vinyl alcohol) (manufactured by Kuraray Co., Ltd., Poval MP203) was added 10 kg of water, and thoroughly mixed to give a slurry. This slurry was fed with a diaphragm pump, and was subjected to dispersion with a horizontal sand mill (UVM-2: manufactured by AIMEX Co., Ltd.) packed with zirconia beads having a mean particle diameter of 0.5 mm for 3 hours and 30 minutes. Thereafter, 0.2 g of a benzisothiazolinone sodium salt and water were added thereto, thereby adjusting the concentration of the development accelerator to be 20% by weight. Accordingly, development accelerator-1 dispersion was obtained. Particles of the development accelerator included in the resulting development accelerator dispersion had a median diameter of 0.48  $\mu\text{m}$ , and a maximum particle diameter of 1.4  $\mu\text{m}$  or less. The resultant development accelerator dispersion was subjected to filtration with a polypropylene filter having a pore size of 3.0  $\mu\text{m}$  to remove foreign substances such as dust, and stored.

## &lt;Preparations of Solid Dispersions of Development Accelerator-2 and Color-Tone-Adjusting Agent&gt;

Also concerning solid dispersions of development accelerator-2 and color-tone-adjusting agent-1, dispersion was executed similar to the development accelerator-1, and thus dispersions of 20% by weight and 15% by weight were respectively obtained.

## 6) Preparations of Organic Polyhalogen Compound Dispersion

## &lt;Preparation of Organic Polyhalogen Compound-1 Dispersion&gt;

10 kg of organic polyhalogen compound-1 (tribromomethane sulfonylbenzene), 10 kg of a 20% by weight aqueous solution of modified poly(vinyl alcohol) (manufactured by Kuraray Co., Ltd., Poval MP203), 0.4 kg of a 20% by weight aqueous solution of sodium triisopropylnaphthalenesulfonate and 14 kg of water were thoroughly admixed to give a slurry. This slurry was fed with a diaphragm pump, and was subjected to dispersion with a horizontal sand mill (UVM-2: manufactured by AIMEX Co., Ltd.) packed with zirconia beads having a mean particle diameter of 0.5 mm for 5 hours. Thereafter, 0.2 g of a benzisothiazolinone sodium salt and water were added thereto, thereby adjusting the concentration of the organic polyhalogen compound to be 30% by weight. Accordingly, organic polyhalogen compound-1 dispersion was obtained.

Particles of the organic polyhalogen compound included in the resulting organic polyhalogen compound dispersion had a median diameter of 0.41  $\mu\text{m}$ , and a maximum particle diameter of 2.0  $\mu\text{m}$  or less. The resultant organic polyhalogen compound dispersion was subjected to filtration with a polypropylene filter having a pore size of 10.0  $\mu\text{m}$  to remove foreign substances such as dust, and stored.

## &lt;Preparation of Organic Polyhalogen Compound-2 Dispersion&gt;

10 kg of organic polyhalogen compound-2 (N-butyl-3-tribromomethane sulfonylbenzamide), 20 kg of a 10% by weight aqueous solution of modified poly(vinyl alcohol) (manufactured by Kuraray Co., Ltd., Poval MP203) and 0.4 kg of a 20% by weight aqueous solution of sodium triisopropylnaphthalenesulfonate were thoroughly admixed to give a slurry. This slurry was fed with a diaphragm pump, and was subjected to dispersion with a horizontal sand mill (UVM-2: manufactured by AIMEX Co., Ltd.) packed with zirconia beads having a mean particle diameter of 0.5 mm for 5 hours. Thereafter, 0.2 g of a benzisothiazolinone sodium salt and water were added thereto, thereby adjusting the concentration

of the organic polyhalogen compound to be 30% by weight. This fluid dispersion was heated at 40° C. for 5 hours to obtain organic polyhalogen compound-2 dispersion. Particles of the organic polyhalogen compound included in the resulting organic polyhalogen compound dispersion had a median diameter of 0.40  $\mu\text{m}$ , and a maximum particle diameter of 1.3  $\mu\text{m}$  or less. The resultant organic polyhalogen compound dispersion was subjected to filtration with a polypropylene filter having a pore size of 3.0  $\mu\text{m}$  to remove foreign substances such as dust, and stored.

## 7) Preparation of Phthalazone Solution

A 5% by weight solution of phthalazone was prepared.

## 8) Preparations of Aqueous Solution of Mercapto Compound

## &lt;Preparation of Aqueous Solution of Mercapto Compound-1&gt;

Mercapto compound-1 (1-(3-sulfophenyl)-5-mercaptopetrazole sodium salt) in an amount of 7 g was dissolved in 993 g of water to give a 0.7% by weight aqueous solution.

## &lt;Preparation of Aqueous Solution of Mercapto Compound-2&gt;

Mercapto compound-2 (1-(3-methylureidophenyl)-5-mercaptopetrazole) in an amount of 20 g was dissolved in 980 g of water to give a 2.0% by weight aqueous solution.

## 9) Preparation of SBR Latex Solution

To a polymerization tank of a gas monomer reaction apparatus (manufactured by Taiatsu Techno Corporation, TAS-2J type), were charged 287 g of distilled water, 7.73 g of a surfactant (Pionin A-43-S (manufactured by TAKEMOTO OIL & FAT CO., LTD.): solid matter content of 48.5% by weight), 14.06 mL of 1 mol/L sodium hydroxide, 0.15 g of ethylenediamine tetraacetate tetrasodium salt, 255 g of styrene, 11.25 g of acrylic acid, and 3.0 g of tert-dodecyl mercaptan, followed by sealing of the reaction vessel and stirring at a stirring rate of 200 rpm. Degassing was conducted with a vacuum pump, followed by repeating nitrogen gas replacement several times. Thereto was injected 108.75 g of 1,3-butadiene, and the inner temperature is elevated to 60° C. Thereto was added a solution of 1.875 g of ammonium persulfate dissolved in 50 mL of water, and the mixture was stirred for 5 hours as it stands.

The temperature was further elevated to 90° C., followed by stirring for 3 hours. After completing the reaction, the inner temperature was lowered to reach to the room temperature, and thereafter the mixture was treated by adding 1 mol/L sodium hydroxide and ammonium hydroxide to give the molar ratio of  $\text{Na}^+$  ion:  $\text{NH}_4^+$  ion=1:5.3, and thus, the pH of the mixture was adjusted to 8.4. Thereafter, filtration with a polypropylene filter having the pore size of 1.0  $\mu\text{m}$  was conducted to remove foreign substances such as dust followed by storage. Accordingly, SBR latex was obtained in an amount of 774.7 g. Upon the measurement of halogen ion by ion chromatography, concentration of chloride ion was revealed to be 3 ppm. As a result of the measurement of the concentration of the chelating agent by high performance liquid chromatography, it was revealed to be 145 ppm.

The aforementioned latex had a mean particle diameter of 90 nm,  $T_g$  of 17° C., solid matter concentration of 44% by weight, the equilibrium moisture content at 25° C. and 60% RH of 0.6% by weight, ionic conductance of 4.80 mS/cm (measurement of the ionic conductance performed using a conductivity meter CM-30S manufactured by To a Electronics Ltd. for the latex stock solution (44% by weight) at 25° C.) and pH of 8.4.

## 6) 2-2. Preparations of Coating Solution

## 1) Preparations of Coating Solution for Image Forming Layer

To the dispersion of silver salt of fatty acid in an amount of 1000 g and 276 mL of water were serially added the organic polyhalogen compound-1 dispersion, the organic polyhalogen compound-2 dispersion, the SBR latex (Tg: 17°C.) solution, the reducing agent-1 dispersion, the phthalazone dispersion, the hydrogen bonding compound-1 dispersion, the development accelerator-1 dispersion, the development accelerator-2 dispersion, the color-tone-adjusting agent-1 dispersion, the mercapto compound-1 aqueous solution, and the mercapto compound-2 aqueous solution. After adding thereto the silver iodide complex-forming agent, the emulsion for coating solution was added thereto in an amount shown in Table 1, followed by thorough mixing just prior to the coating, which is fed directly to a coating die.

2) Preparation of Coating Solution for Intermediate Layer

To 1000 g of poly(vinyl alcohol) PVA-205 (manufactured by Kuraray Co., Ltd.) and 4200 mL of a 19% by weight solution of methyl methacrylate/styrene/butyl acrylate/hydroxyethyl methacrylate/acrylic acid copolymer (weight ratio of the copolymerization of 64/9/20/5/2) latex were added 27 mL of a 5% by weight aqueous solution of aerosol OT (manufactured by American Cyanamid Co.), 135 mL of a 20% by weight aqueous solution of diammonium phthalate, and water to give total amount of 10000 g. The mixture was adjusted with sodium hydroxide to give the pH of 7.5. Accordingly, the coating solution for the intermediate layer was prepared, and was fed to a coating die to provide 9.1 mL/m<sup>2</sup>.

Viscosity of the coating solution was 58 [mPa·s] which was measured with a B type viscometer at 40°C. (No. 1 rotor, 60 rpm).

3) Preparation of Coating Solution for First Layer of Surface Protective Layers

In water was dissolved 64 g of inert gelatin, and thereto were added 112 g of a 19.0% by weight solution of methyl methacrylate/styrene/butyl acrylate/hydroxyethyl methacrylate/acrylic acid copolymer (weight ratio of the copolymerization of 64/9/20/5/2) latex, 30 mL of a 15% by weight methanol solution of phthalic acid, 23 mL of a 10% by weight aqueous solution of 4-methyl phthalic acid, 28 mL of 0.5 mol/L sulfuric acid, 5 mL of a 5% by weight aqueous solution of aerosol OT, 0.5 g of phenoxyethyl alcohol, and 0.1 g of benzisothiazolinone. Water was added to give total amount of 750 g. Immediately before coating, 26 mL of a 4% by weight chrome alum which had been mixed with a static mixer was fed to a coating die so that the amount of the coating solution became 18.6 mL/m<sup>2</sup>.

Viscosity of the coating solution was 20 [mPa·s] which was measured with a B type viscometer at 40°C. (No. 1 rotor, 60 rpm).

4) Preparation of Coating Solution for Second Layer of Surface Protective Layers

In water was dissolved 80 g of inert gelatin and thereto were added 102 g of a 27.5% by weight solution of methyl methacrylate/styrene/butyl acrylate/hydroxyethyl methacrylate/acrylic acid copolymer (weight ratio of the copolymerization of 64/9/20/5/2) latex, 5.4 mL of a 2% by weight solution of a fluorocarbon surfactant (F-1), 5.4 mL of a 2% by weight aqueous solution of another fluorocarbon surfactant (F-2), 23 mL of a 5% by weight aqueous solution of aerosol OT, 4 g of polymethyl methacrylate fine particles (mean particle diameter of 0.7 µm, distribution of volume weighted average being 30%), 21 g of polymethyl methacrylate fine particles (mean particle diameter of 3.6 µm, distribution of volume weighted average being 60%), 1.6 g of 4-methyl phthalic acid, 4.8 g of phthalic acid, 44 mL of 0.5 mol/L sulfuric acid, and 10 mg of benzisothiazolinone. Water was

added to give total amount of 650 g. Immediately before coating, 445 mL of an aqueous solution containing 4% by weight chrome alum and 0.67% by weight phthalic acid were added and admixed with a static mixer to give a coating solution for the second layer of the surface protective layers, which was fed to a coating die so that 8.3 mL/m<sup>2</sup> could be provided.

Viscosity of the coating solution was 19 [mPa·s] which was measured with a B type viscometer at 40°C. (No. 1 rotor, 60 rpm).

2-3. Preparations of Sample Nos. 1-1 to 1-8 of Photothermographic Materials

To compare the double-sided photothermographic material and the single-sided photothermographic material, simultaneous overlaying coating by a slide bead coating method was subjected, on one side and both sides of the support, in order of the image forming layer, intermediate layer, first layer of the surface protective layers, and second layer of the surface protective layers, starting from the undercoated face. Thus sample Nos. 1-1 to 1-8 of photothermographic materials were produced. In this method, the temperature of the coating solution was adjusted to 31°C. for the image forming layer and intermediate layer, to 36°C. for the first layer of the surface protective layers, and to 37°C. for the second layer of the surface protective layers.

Concerning the double-sided photothermographic material, the amount of coated silver contained in the silver salt of fatty acid was 0.646 g/m<sup>2</sup> per one side, and 1.292 g/m<sup>2</sup> with respect to the sum of both sides. Concerning the single-sided photothermographic material, the amount of coated silver contained in the silver salt of fatty acid was 1.292 g/m<sup>2</sup>, which was similar to the sum of the coating amounts of both sides in the double-sided photothermographic material.

The coating amount of each compound (g/m<sup>2</sup>) for the image forming layer per one side in the double-sided photothermographic material is as follows.

|                                            |               |
|--------------------------------------------|---------------|
| Silver salt of fatty acid                  | 2.85          |
| Organic polyhalogen compound-1             | 0.028         |
| Organic polyhalogen compound-2             | 0.094         |
| SBR latex                                  | 5.20          |
| Reducing agent-1                           | 0.46          |
| Phthalazone                                | 0.18          |
| Hydrogen bonding compound-1                | 0.15          |
| Development accelerator-1                  | 0.005         |
| Development accelerator-2                  | 0.035         |
| Color-tone-adjusting agent-1               | 0.002         |
| Mercapto compound-1                        | 0.001         |
| Mercapto compound-2                        | 0.003         |
| Silver halide (on the basis of Ag content) | (see Table 1) |

Conditions for coating and drying were as follows.

The support was discharged by ionic wind. Coating was performed at the speed of 160 m/min. Conditions for coating and drying were adjusted within the range described below, and conditions were set to obtain the most stable surface state. The clearance between the leading end of the coating die and the support was 0.10 mm to 0.30 mm. The pressure in the vacuum chamber was set to be lower than atmospheric pressure by 196 Pa to 882 Pa. In the subsequent cooling zone, the coating solution was cooled by wind having the dry-bulb temperature of 10°C. to 20°C. Transportation with no contact was carried out, and the coated support was dried with an air of the dry-bulb of 23°C. to 45°C. and the wet-bulb of 15°C. to 21°C. in a helical type contactless drying apparatus. After drying, moisture conditioning was performed at 25°C.

**117**

in the humidity of 40% RH to 60% RH. Then, the film surface was heated to be 70° C. to 90° C., and after heating, the film surface was cooled to 25° C.

Thus prepared photothermographic material had a level of matting of 250 seconds as Beck's smoothness.

Chemical structures of the compounds used in Examples of the invention are shown below.



Compound 1 that can be one-electron-oxidized to provide a one-electron oxidation product which releases one or more electrons



5



Compound 2 that can be one-electron-oxidized to provide a one-electron oxidation product which releases one or more electrons

10

20

Compound 3 that can be one-electron-oxidized to provide a one-electron oxidation product which releases one or more electrons

25

30

35



TABLE 1

| Sample No.       | Emulsion No. | Silver Halide | Amount of Coated Silver Halide |                                |           |               | Note        |
|------------------|--------------|---------------|--------------------------------|--------------------------------|-----------|---------------|-------------|
|                  |              |               | One Side (g/m <sup>2</sup> )   | Both Sides (g/m <sup>2</sup> ) | Light (%) | Crossover (%) |             |
| 1-1 Single-sided | A            |               | 1.00                           | —                              | 1.0       | X             | Comparative |
| 1-2 Coating      | A            |               | 0.50                           | —                              | 3.0       | X             | Comparative |
| 1-3              | A            |               | 0.25                           | —                              | 5.5       | X             | Comparative |
| 1-4              | A            |               | 0.125                          | —                              | 6.7       | X             | Comparative |
| 1-5 Double-sided | A            |               | 0.50                           | 1.00                           | 3.0       | 25.5          | Comparative |
| 1-6 Coating      | A            |               | 0.25                           | 0.50                           | 4.3       | 27.3          | Comparative |
| 1-7              | A            |               | 0.125                          | 0.25                           | 6.8       | 38.1          | Invention   |
| 1-8              | A            |               | 0.0625                         | 0.125                          | 8.2       | 43.1          | Invention   |

TABLE 2

| Sample No.       | Fog  | Sensitivity | Dmax | Gradation | Sharpness | Note        |
|------------------|------|-------------|------|-----------|-----------|-------------|
| 1-1 Single-sided | 0.25 | 100         | 3.83 | 4.52      | 0.61      | Comparative |
| 1-2 Coating      | 0.21 | 90          | 3.05 | 3.82      | 0.58      | Comparative |
| 1-3              | 0.18 | 71          | 2.00 | 3.02      | 0.55      | Comparative |
| 1-4              | 0.17 | 45          | 1.55 | 2.63      | 0.52      | Comparative |
| 1-5 Double-sided | 0.35 | 117         | 3.95 | 4.83      | 0.51      | Comparative |
| 1-6 Coating      | 0.30 | 97          | 3.09 | 4.31      | 0.53      | Comparative |
| 1-7              | 0.17 | 92          | 2.05 | 3.88      | 0.63      | Invention   |
| 1-8              | 0.16 | 78          | 1.65 | 3.05      | 0.65      | Invention   |

**119**

-continued  
Compound 1 having adsorptive group and reducing group



Compound 2 having adsorptive group and reducing group



Reducing agent-1



Hydrogen bonding compound-1



Organic polyhalogen compound-1

**120**

-continued  
Organic polyhalogen compound-2



Mercapto compound-1



Mercapto compound-2



Development accelerator-1



Development accelerator-2



Color-tone-adjusting agent-1





### 3. Evaluation of Photographic Properties

#### 3-1. Preparation

The obtained sample was cut into a half-cut size, and was wrapped with the following packaging material under an environment of 25°C. and 50% RH, and stored for 2 weeks at an ambient temperature.

##### <Packaging Material>

A film laminated with PET 10 µm/PE 12 µm/aluminum foil 9 µm/Ny 15 µm/polyethylene 50 µm containing carbon at 3% by weight:

oxygen permeability at 25°C.: 0.02 mL·atm<sup>-1</sup>m<sup>-2</sup>day<sup>-1</sup>;  
vapor permeability at 25°C.: 0.10 g·atm<sup>-1</sup>m<sup>-2</sup>day<sup>-1</sup>.

#### 3-2. Exposure

In the case of the double-sided photothermographic material, two sheets of the fluorescent intensifying screen A described below were used. The assembly for image formation was provided by inserting the sample between them. This assembly was subjected to X-ray exposure for 0.05 seconds, and then X-ray sensitometry was performed. The X-ray apparatus used was DRX-3724HD (trade name) produced by Toshiba Corp., and a tungsten target tube was used. X-ray emitted by a pulse generator operated at three phase voltage of 80 kVp and penetrated through a filter comprising 7 cm thickness of water having the absorption ability almost the same as human body was used as the light source. While changing the exposure value of X-ray by a distance method, the sample was subjected to exposure with a step wedge tablet having a width of 0.15 in terms of log E.

In the case of the single-sided photothermographic material, one sheet of the following fluorescent intensifying screen A was used. The X-ray source, screen, image forming layer, support, and black paper were set in a cassette in this order, wherein the image forming layer side was set to be the side of the screen, and the assembly was subjected to exposure similar to the double-sided photothermographic material.

##### <Preparation of Fluorescent Intensifying Screen A>

###### (1) Undercoating

A light reflecting layer comprising alumina powder was coated on a poly(ethylene terephthalate) film (support) having a thickness of 250 µm in a similar manner to the Example 4 in JP-A, No. 2001-124898. The light reflecting layer which had a film thickness of 50 µm after drying, was prepared.

###### (2) Preparation of Fluorescent Substance Sheet

250 g of BaFBr:Eu fluorescent substance (mean particle size of 3.5 µm), 8 g of polyurethane type binder resin (manufactured by Dai Nippon Ink & Chemicals, Inc., trade name: PANDEX T5265M), 2 g of epoxy type binder resin (manufactured by Yuka Shell Epoxy Co., Ltd., trade name: EPIKOTE 101) and 0.5 g of isocyanate compounds (manufactured by Nippon Polyurethane Industry Co., Ltd., trade name: CORONATE HX) were added into methyl ethyl ketone, and the mixture was then dispersed by a propeller mixer to prepare the coating solution for the fluorescent substance

layer having a viscosity of 25 PS (25°C.). This coating solution was coated on the surface of a temporary support (pretreated by coating a silicone agent on the surface of polyethylene terephthalate film), and dried to make the fluorescent substance layer. Thereafter, the fluorescent substance sheet was prepared by peeling the fluorescent substance layer from the temporary support.

###### (3) Overlaying the Fluorescent Substance Sheet on Light Reflective Layer.

10 The fluorescent substance sheet prepared above was overlaid on the surface of the light reflective layer of the support having a light reflective layer made in the above process (1), and then pressed by a calendar roller at the pressure of 400 kgw/cm<sup>2</sup> and the temperature of 80°C. to form the fluorescent substance layer on the light reflective layer. The thickness of the obtained fluorescent substance layer was 125 µm and the volume filling factor of fluorescent substance particles in the fluorescent substance layer was 68%.

###### (4) Preparation of Surface Protective Layer

20 Polyester type adhesive agents were coated on one side of a polyethylene terephthalate (PET) film having a thickness of 6 µm, and thereafter the surface protective layer was formed on the fluorescent substance layer by a laminating method. As described above, the fluorescent intensifying screen A comprising a support, a light reflective layer, a fluorescent substance layer and a surface protective layer was prepared.

###### (5) Emission Characteristics

30 The emission spectrum of the intensifying screen A was measured by X-ray at 40 kVp and is shown in FIG. 8. The fluorescent intensifying screen A showed an emission having a peak at 390 nm and a narrow half width.

#### 3-3. Thermal Development

35 As shown in FIG. 9, Fuji Medical dry laser Imager FM-DP L was modified so that 6 sheets of panel heater were set to be arranged in a staggered form. The photothermographic material was conveyed so that the front side and the backside of the material became in direct contact with the panel heater surface alternatively. The temperature of 6 panel heaters and time period for passing through the 6 panel heaters were set to the values shown in Table 3. The total time period for passing through the 6 panel heaters was set to be 33 seconds. The above was used for the evaluation of general photographic properties at thermally developing both sides simultaneously.

TABLE 3

|                             | Temperature (°C.) | Time Period (sec) |
|-----------------------------|-------------------|-------------------|
| First Heating Means (L1-1)  | 100               | 5.5               |
| Second Heating Means (L2-1) | 100               | 5.5               |
| Third Heating Means (L1-2)  | 112               | 5.5               |
| Fourth Heating Means (L2-2) | 119               | 5.5               |
| Fifth Heating Means (L1-3)  | 119               | 5.5               |
| Sixth Heating Means (L2-3)  | 121               | 5.5               |

#### 3-4. Condition for Evaluation

##### 1) Measurement of Haze of Film

60 The haze indicates the degree of diffusion of the light incident to a photosensitive material, and the ratio of the amount of diffused transmitted light to total amount of transmitted light is expressed in percentage. The haze measuring apparatus Model 1001DP produced by NIPPON DEN-SHOKU Co., Ltd. was used for the measurement of haze.

65 The haze of the film was measured before and after thermal development of each unexposed sample, and the ratio of haze after thermal development to haze before thermal development is calculated.

## 123

2) Measurement of Parallel Light Component of Transmitted Light

<Measurement of Parallel Light Component>

One side of the double-sided photothermographic material was removed and the resultant was placed in a spectrophotometer U-3350 produced by Hitachi, Ltd., and the transmitted light density at 390 nm was measured.

3) Measurement of Sensitivity

Density of obtained thermally developed sample was measured and therefrom a photographic characteristic curve was formed. Sensitivity is expressed in terms of relative value based on the sensitivity obtained for sample No. 1-1, which is taken as 100.

4) Measurement of Sharpness

In respect with sample Nos. 1-1 to 1-4, the samples was inserted between a black paper and the above-described fluorescent intensifying screen A, and subjected to exposure with a rectangular chart for MTF measurement (made from Molybdenum, thickness: 80  $\mu\text{m}$ , the spatial frequency: from 0 line/mm to 10 lines/mm) placed in a distance of 2 mm from the X-ray source. The X-ray source and the development condition were similar to the above. Time period for X-ray exposure was adjusted to give an optical density of 1.2 in the area where the molybdenum was not covered. In respect with sample Nos. 1-5 to 1-8, the sample was placed between a pair of the above-described fluorescent intensifying screen A and subjected to exposure by adjusting the exposure value to give an optical density of 1.2, followed by thermal development to form a rectangular chart. Thereafter, the sample was measured by scanning with a microdensitometer.

A slit having an aperture of 30  $\mu\text{m}$  on the scanning direction and 500  $\mu\text{m}$  on the perpendicular direction was used, and the density profile was measured in a sampling interval of 30  $\mu\text{m}$ . This measurement was repeated by 20 times and then the average value was determined. The results were then utilized as a density profile for calculating CTF value. Thereafter by detecting the peak of the rectangular wave in the density profile at each frequency, the gradation in density at each frequency were calculated. The values of the spatial frequency of one line/mm are shown in Table 2.

5) Measurement of Crossover

The sample was inserted between a black paper and the fluorescent intensifying screen mentioned above, and subjected to X-ray exposure from the black paper side. Similar X-ray source to the above was used for the exposure. The sample was subjected to X-ray exposure while changing the X-ray radiation value by a distance method.

After the exposure, the sample was subjected to thermal development in a similar condition to the above. Thereafter, the developed sample was divided into two parts and then each image forming layer was peeled off. The optical density of the image forming layer of the side which was contacted with the fluorescent intensifying screen was higher than that of the opposite side. The photographic characteristic curves of each image forming layer were formed and an average sensitivity difference ( $\Delta \log E$ ) was determined from the straight portion of the curve (from a density of 0.5 to a density of 1.0). Crossover is calculated from the average value according to the following formula.

$$\text{Crossover}(\%) = 100 / (\text{Antilog}(\Delta \log E) + 1)$$

6) Other Photographic Properties

Fog: The density of the unexposed portion is expressed as fog.

Dmax: Dmax is a maximum density saturated by increasing the exposure value.

## 124

Gradation: Gradation is expressed as a gradient of a line joining the points at fog+(optical density of 0.50) and fog+(optical density of 1.5) on a photographic characteristic curve (i.e., the value equals tan when the angle between the line and the abscissa axis is).

4. Results of Evaluation

The obtained results are shown in Table 1 and Table 2.

It is revealed that the photothermographic materials of the present invention can produce excellent image quality with high sensitivity and high gradation with less amount of silver, compared with the material where the same amount of silver are coated on a single side of the support. Moreover, in spite of the high sensitivity and high gradation, sharpness of the photothermographic material of the present invention is increased rather than reduced with the reduction of the silver amount. The above result is opposed to the conventional understanding that sharpness is reduced by a double-sided photosensitive material where sensitivity is high, but crossover is big, and can not be expected from the traditional knowledge. It is supposed that the increase of the parallel light can increase the sensitivity without deteriorating the sharpness.

Example 2

1. Preparation of Silver Halide Emulsion

<Preparation of Silver Halide Emulsion B (Silver Iodobromide Emulsion)>

3.1 mL of a 1% by weight potassium bromide solution, and then 3.5 mL of 0.5 mol/L sulfuric acid and 31.7 g of phthalated gelatin were added to 1421 mL of distilled water. The liquid was kept at 70°C. while stirring in a stainless steel reaction vessel, and thereto were added total amount of: solution A prepared through diluting 11.11 g of silver nitrate by adding distilled water to give the volume of 95.4 mL; and solution B prepared through diluting 7.15 g of potassium bromide and 0.4 g of potassium iodide with distilled water to give the volume of 97.4 mL, over 130 seconds at a constant flow rate.

Thereafter, 10 mL of a 3.5% by weight aqueous solution of hydrogen peroxide was added thereto, and 10.8 mL of a 10% by weight aqueous solution of benzimidazole was further added.

Moreover, a solution C prepared through diluting 51.86 g of silver nitrate by adding distilled water to give the volume of 317.5 mL and a solution D prepared through diluting 44.2 g of potassium bromide and 2.2 g of potassium iodide with distilled water to give the volume of 400 mL were added. A controlled double jet method was executed through adding total amount of the solution C at a constant flow rate over 30 minutes, accompanied by adding the solution D while maintaining the pAg at 8.1. Potassium hexachloroiridate (III) was added in its entirety to give  $1.5 \times 10^{-4}$  mol per 1 mol of silver, at 10 minutes post initiation of the addition of the solution C and the solution D. Moreover, at 5 seconds after completing the addition of the solution C, a potassium hexacyanoferrate (II) in an aqueous solution was added in its entirety to give  $3.5 \times 10^{-4}$  mol per 1 mol of silver. The mixture was adjusted to the pH of 3.8 with 0.5 mol/L sulfuric acid. After stopping stirring, the mixture was subjected to precipitation/desalting/water washing steps. The mixture was adjusted to the pH of 5.9 with 1 mol/L sodium hydroxide to produce a silver halide dispersion having the pAg of 8.0.

The above-described silver halide dispersion was kept at 38°C. with stirring, and thereto was added 5 mL of a 0.44% by weight methanol solution of 1,2-benzisothiazoline-3-one,

125

followed by elevating the temperature to 47° C. at 40 minutes thereafter. At 20 minutes after elevating the temperature, sodium benzene thiosulfonate in a methanol solution was added at  $9.0 \times 10^{-5}$  mol per 1 mol of silver. At additional 5 minutes later, tellurium sensitizer C in a methanol solution was added at  $1.5 \times 10^{-4}$  mol per 1 mol of silver and subjected to ripening for 91 minutes. Thereafter, 0.5 mL of a 0.8% by weight methanol solution of N,N'-dihydroxy-N'',N''-diethylmelamine was added thereto, and at additional 4 minutes thereafter, 5-methyl-2-mercaptopbenzimidazole in a methanol solution at  $2.2 \times 10^{-3}$  mol per 1 mol of silver, 1-phenyl-2-heptyl-5-mercaptop-1,3,4-triazole in a methanol solution at  $2.5 \times 10^{-3}$  mol per 1 mol of silver, and 1-(3-methylureidophenyl)-5-mercaptoptetrazole in an aqueous solution at  $3.5 \times 10^{-3}$  mol per 1 mol of silver were added to produce a silver halide emulsion B.

Grains in thus prepared silver halide emulsion were silver iodobromide grains having a mean equivalent spherical diameter of 0.13  $\mu\text{m}$ , a variation coefficient of an equivalent spherical diameter distribution of 18%, which uniformly include iodine at 3.5 mol %. Grain size and the like were determined from the average of 1000 grains using an electron microscope. The {100} face ratio of these grains was found to be 80% using a Kubelka-Munk method.

<Preparations of Silver Halide Emulsion C and D (High-Silver Iodide Emulsion)>

Silver halide emulsion C was prepared in a similar manner to the preparation of silver halide emulsion B except that the amounts of potassium bromide and potassium iodide in solution B and solution D were adjusted and the temperature, addition time, and the pAg were adjusted. Grains in the silver halide emulsion C were silver iodobromide grains having a mean equivalent spherical diameter of 0.13  $\mu\text{m}$ , a variation coefficient of an equivalent spherical diameter distribution of 19%, which uniformly include iodine at 65 mol %.

Silver halide emulsion D was prepared in a similar manner to the preparation of silver halide emulsion B except that potassium bromide and potassium iodide in solutions B and D were all changed to silver iodide and the temperature, addition time, and the pAg were adjusted. Grains in the silver halide emulsion D were pure silver iodide grains having a mean equivalent spherical diameter of 0.13  $\mu\text{m}$ , a variation coefficient of an equivalent spherical diameter distribution of 18%.

## 2. Preparations of Photothermographic Material

<Preparation of Silver Iodide Complex-forming Agent Solution>

8 kg of modified poly(vinyl alcohol) MP203 was dissolved in 174.57 kg of water, and thereto were added 3.15 kg of a 20% by weight aqueous solution of sodium triisopropylnaphthalenesulfonate and 14.28 kg of a 70% by weight aqueous solution of 6-isopropylphthalazine. Accordingly, a 5% by weight solution of silver iodide complex-forming agent compound was prepared.

## <Preparations of Coated Sample>

Similar to Example 1, simultaneous overlaying coating by a slide bead coating method was subjected, on both sides of the support, in order of the image forming layer, intermediate layer, first layer of the surface protective layers, and second layer of the surface protective layers, starting from the under-coated face. Thus sample Nos. 2-1 to 2-10 of photothermographic materials were produced. In this method, the temperature of the coating solution was adjusted to 31° C. for the image forming layer and intermediate layer, to 36° C. for the first layer of the surface protective layers, and to 37° C. for the second layer of the surface protective layers.

126

The amount of coated silver contained in the silver salt of fatty acid was 0.646 g/m<sup>2</sup> per one side, and 1.292 g/m<sup>2</sup> with respect to the sum of both sides.

The coating amount of each compound (g/m<sup>2</sup>) for the image forming layer per one side is as follows.

|    |                                            |               |
|----|--------------------------------------------|---------------|
| 10 | Silver salt of fatty acid                  | 2.85          |
|    | Organic polyhalogen compound-1             | 0.028         |
|    | Organic polyhalogen compound-2             | 0.094         |
|    | Silver iodide complex-forming agent        | 0.46          |
|    | SBR latex                                  | 5.20          |
|    | Reducing agent-1                           | 0.46          |
|    | Hydrogen bonding compound-1                | 0.15          |
|    | Development accelerator-1                  | 0.005         |
|    | Development accelerator-2                  | 0.035         |
|    | Color-tone-adjusting agent-1               | 0.002         |
|    | Mercapto compound-1                        | 0.001         |
|    | Mercapto compound-2                        | 0.003         |
|    | Silver halide (on the basis of Ag content) | (see Table 4) |

## 3. Evaluation of Photographic Properties

Evaluation similar to Example 1 was performed and the results are shown in Table 4 and Table 5. From the results, it is revealed that the effect of the invention is higher in the case where the silver iodide content is 65 mol %, and the effect is more higher in the case of 100 mol %.

## Example 3

### 1. Preparations of Silver Halide Emulsion

<Preparation of Silver Halide Emulsion E (Tabular AgI Emulsion of Ultra High Aspect Ratio)>

#### -Preparation of Host Emulsion-

A solution was prepared by adding 4.3 mL of a 1% by weight potassium iodide solution, and then 3.5 mL of 0.5 mol/L sulfuric acid and 5.8 g of phthalated gelatin to 1421 mL of distilled water. The solution was kept at 79° C. while stirring in a stainless steel reaction vessel, and thereto were added total amount of: solution A prepared through diluting 22.22 g of silver nitrate by adding distilled water to give the volume of 195.6 mL; and solution B prepared through diluting 21.8 g of potassium iodide with distilled water to give the volume of 218 mL, over 9 minutes at a constant flow rate.

Thereafter, 10 mL of a 3.5% by weight aqueous solution of hydrogen peroxide was added thereto, and 10.8 mL of a 10% by weight aqueous solution of benzimidazole was further added. The mixture was subjected to ripening for 10 minutes and thereto, 30.9 g of phthalated gelatin was added thereto.

Moreover, a solution C prepared through diluting 51.86 g of silver nitrate by adding distilled water to give the volume of 317.5 mL and a solution D prepared through diluting 60 g of potassium iodide with distilled water to give the volume of 600 mL were added. A method of controlled double jet was

executed through adding total amount of the solution C at a constant flow rate over 120 minutes, accompanied by adding the solution D while maintaining the pAg at 8.1. Potassium hexachloroiridate (III) was added in its entirety to give  $1.2 \times 10^{-4}$  mol per 1 mol of silver, at 10 minutes post initiation of the addition of the solution C and the solution D. The mixture was adjusted to the pH of 3.8 with 0.5 mol/L sulfuric acid. After stopping stirring, the mixture was subjected to precipitation/desalting/water washing steps. The mixture was adjusted to the pH of 5.9 with 1 mol/L sodium hydroxide to produce a silver halide dispersion having the pAg of 8.0.

The obtained silver halide emulsion was a pure silver iodide emulsion, and the obtained silver halide grains were

tabular grains having a mean projected area equivalent diameter of 1.707  $\mu\text{m}$ , a variation coefficient of a projected area equivalent diameter distribution of 18.7%, a mean thickness of 0.085  $\mu\text{m}$ , and a mean aspect ratio of 19.8. Tabular grains having an aspect ratio of 10 or more occupied 80% or more of the total projected area. A mean equivalent spherical diameter of the grains was 0.72  $\mu\text{m}$ . 30% or more of the silver iodide existed in  $\gamma$  phase from the result of powder X-ray diffraction analysis.

mol per 1 mol of silver. At additional 5 minutes later, tellurium sensitizer C in a methanol solution was added at  $2.0 \times 10^{-5}$  mol per 1 mol of silver and subjected to ripening for 91 minutes. And then, 1.2 mL of a 0.8% by weight N,N'-dihydroxy-N",N"-diethylmelamine in methanol was added thereto, and at additional 4 minutes thereafter, 5-methyl-2-mercaptopbenzimidazole in a methanol solution at  $3.5 \times 10^{-3}$  mol per 1 mol of silver, 1-phenyl-2-heptyl-5-mercapto-1,3,4-triazole in a methanol solution at  $2.4 \times 10^{-3}$  mol per 1 mol of

TABLE 4

| Sample No. | Emulsion No. | Silver Halide | Silver Halide | Amount of Coated Silver Halide |                              | Haze before                    | Haze after         | Crossover (%)       | Note                |
|------------|--------------|---------------|---------------|--------------------------------|------------------------------|--------------------------------|--------------------|---------------------|---------------------|
|            |              |               |               | Composition AgI (mol %)        | One Side (g/m <sup>2</sup> ) | Both Sides (g/m <sup>2</sup> ) | Parallel Light (%) | Thermal Development | Thermal Development |
| 2-1        | B            | 3.5           | 0.50          | 1.00                           | 2.0                          | 73                             | 75                 | 18.0                | Comparative         |
| 2-2        | B            | 3.5           | 0.33          | 0.66                           | 3.0                          | 68                             | 69                 | 27.7                | Comparative         |
| 2-3        | B            | 3.5           | 0.27          | 0.54                           | 4.5                          | 65                             | 64                 | 32.3                | Invention           |
| 2-4        | B            | 3.5           | 0.15          | 0.30                           | 5.3                          | 60                             | 61                 | 36.8                | Invention           |
| 2-5        | C            | 65.0          | 0.27          | 0.54                           | 5.2                          | 64                             | 55                 | 32.9                | Invention           |
| 2-6        | C            | 65.0          | 0.15          | 0.30                           | 6.5                          | 59                             | 50                 | 35.3                | Invention           |
| 2-7        | D            | 85.0          | 0.50          | 1.00                           | 4.5                          | 73                             | 63                 | 28.9                | Comparative         |
| 2-8        | D            | 85.0          | 0.33          | 0.66                           | 5.3                          | 69                             | 53                 | 28.9                | Invention           |
| 2-9        | D            | 85.0          | 0.27          | 0.54                           | 6.3                          | 64                             | 42                 | 33.1                | Invention           |
| 2-10       | D            | 85.0          | 0.15          | 0.30                           | 8.3                          | 59                             | 38                 | 35.5                | Invention           |

TABLE 5

| Sam- ple No. | Emulsion No. | Silver Halide |      |           |           |             | Note |
|--------------|--------------|---------------|------|-----------|-----------|-------------|------|
|              |              | Fog           | Dmax | Gradation | Sharpness |             |      |
| 2-1          | B            | 0.40          | 2.53 | 4.33      | 0.63      | Comparative | 35   |
| 2-2          | B            | 0.38          | 2.22 | 3.81      | 0.61      | Comparative | 36   |
| 2-3          | B            | 0.33          | 2.03 | 3.55      | 0.65      | Invention   | 37   |
| 2-4          | B            | 0.31          | 1.64 | 3.03      | 0.70      | Invention   | 38   |
| 2-5          | C            | 0.25          | 2.15 | 3.65      | 0.72      | Invention   | 39   |
| 2-6          | C            | 0.21          | 1.66 | 3.33      | 0.75      | Invention   | 40   |
| 2-7          | D            | 0.28          | 2.51 | 4.41      | 0.63      | Comparative | 41   |
| 2-8          | D            | 0.22          | 2.29 | 3.96      | 0.70      | Invention   | 42   |
| 2-9          | D            | 0.18          | 2.21 | 3.67      | 0.74      | Invention   | 43   |
| 2-10         | D            | 0.16          | 1.76 | 3.35      | 0.78      | Invention   | 44   |

#### -Epitaxial Growth of Grains-

1 mol equivalent of the silver iodide tabular host emulsion described above was added to the reaction vessel. The pAg measured at 38°C. was 10.2. After adding potassium hexacyanoferrate (II) in an aqueous solution in its entirety to give  $1.0 \times 10^{-3}$  mol per 1 mol of silver, 0.5 mol/L potassium bromide solution and 0.5 mol/L silver nitrate solution were added at an addition speed of 10 mL/min over 20 minutes by double jet addition to precipitate substantially a 8 mol % of silver bromide on the silver iodide host grains as epitaxial form while keeping the pAg at 10.2 during the operation.

Furthermore, the mixture was adjusted to the pH of 3.8 with 0.5 mol/L sulfuric acid. After stopping stirring, the mixture was subjected to precipitation/desalting/water washing steps. The mixture was adjusted to the pH of 5.9 with 1 mol/L sodium hydroxide to produce a silver halide dispersion having the pAg of 11.0.

The above-mentioned silver halide dispersion was kept at 38°C. with stirring, and thereto was added 5 mL of a 0.34% by weight methanol solution of 1,2-benzisothiazoline-3-one, and after 40 minutes the temperature was elevated to 47°C. At 20 minutes after elevating the temperature, sodium benzene thiosulfonate in a methanol solution was added at  $6.5 \times 10^{-5}$

silver, and 1-(3-methylureido phenyl)-5-mercaptopetrazole in an aqueous solution at  $8.5 \times 10^{-3}$  mol per 1 mol of silver were added to produce silver halide emulsion E.

#### <Preparation of Silver Halide Emulsion F (Non-Tabular Silver Iodide Emulsion)>

Preparation of silver halide emulsion F was conducted in a similar manner to the process in the preparation of silver halide emulsion E except that a non-tabular silver halide emulsion having an mean projected area equivalent diameter of 0.71  $\mu\text{m}$  prepared according to silver halide emulsion D of Example 2 was used instead of the tabular silver iodide host emulsion; and the addition amount of the tellurium sensitizer was optimized.

#### <Preparation of Silver Halide Emulsion G (Tabular Silver Iodide Emulsion Having Different Aspect Ratio)>

Preparation of silver halide emulsion G was conducted in a similar manner to the process in the preparation of silver halide emulsion E except that the host emulsion, which was prepared by adjusting the addition speed of solution C and solution D and the pAg, was used and the addition amount of the tellurium sensitizer was optimized. Grains in the host emulsion had a mean projected area equivalent diameter of 0.907  $\mu\text{m}$ , a variation coefficient of a projected area equivalent diameter distribution of 15.7%, a mean thickness of 0.302  $\mu\text{m}$ , and a mean aspect ratio of 3.1, and tabular grains having an aspect ratio of 2 or more occupied 80% or more of the total projected area. A mean equivalent spherical diameter of the grains was 0.72  $\mu\text{m}$ .

#### <Preparation of Silver Halide Emulsion H (Tabular Silver Iodide Emulsion Having Different Aspect Ratio)>

Preparation of silver halide emulsion H was conducted in a similar manner to the process in the preparation of silver halide emulsion E except that the host emulsion, which was prepared by adjusting the addition speed of solution C and solution D and the pAg, was used and the addition amount of the tellurium sensitizer was optimized. Grains in the host emulsion had a mean projected area equivalent diameter of 1.551  $\mu\text{m}$ , a variation coefficient of a projected area equivalent diameter distribution of 17.3%, a mean thickness of

0.103  $\mu\text{m}$ , and a mean aspect ratio of 15.1, and tabular grains having an aspect ratio of 5 or more occupied 80% or more of the total projected area. A mean equivalent spherical diameter of the grains was 0.72  $\mu\text{m}$ .

<Preparation of Silver Halide Emulsion I>

Preparation of silver halide emulsion I was conducted in a similar manner to the process in the preparation of silver halide emulsion E except that the host emulsion prepared by adjusting the temperature at the addition of solution A and solution B, the addition speed of solution C and solution D, and the pAg was used, and the addition amount of the tellurium sensitizer was optimized. Grains in the host emulsion had a mean projected area equivalent diameter of 0.205  $\mu\text{m}$ , a variation coefficient of a projected area equivalent diameter distribution of 15.3%, a mean thickness of 0.127  $\mu\text{m}$ , a mean aspect ratio of 1.6, and a mean equivalent spherical diameter of 0.15  $\mu\text{m}$ .

2. Preparations of Photothermographic Material

<Preparation of Nucleator Dispersion>

2.5 g of poly(vinyl alcohol) (manufactured by Kuraray Co., Ltd., PVA-217) and 87.5 g of water are added to 10 g of nucleator SH-7, and thoroughly admixed to give a slurry. This slurry is allowed to stand for 3 hours. Zirconia beads having a mean particle diameter of 0.5 mm are provided in an amount of 240 g, and charged in a vessel with the slurry. Dispersion is performed with a dispersing machine (1/4G sand grinder mill: manufactured by AIMEX Co., Ltd.) for 10 hours to obtain a solid fine particle dispersion of nucleator. Particles of the nucleator included in the resulting nucleator dispersion have a mean particle diameter of 0.5  $\mu\text{m}$ , and 80% by weight of the particles has a particle diameter of 0.1  $\mu\text{m}$  to 1.0  $\mu\text{m}$ .

<Preparation of Coated Sample>

Similar to Example 1, simultaneous overlaying coating by a slide bead coating method was subjected, on both sides of the support, in order of the image forming layer, intermediate layer, first layer of the surface protective layers, and second layer of the surface protective layers, starting from the under-coated face. Thus sample Nos. 3-1 to 3-9 of photothermographic materials were produced. In this method, the temperature of the coating solution was adjusted to 31°C. for the image forming layer and intermediate layer, to 36°C. for the first layer of the surface protective layers, and to 37°C. for the second layer of the surface protective layers.

The amount of coated silver contained in the silver salt of fatty acid was 0.646  $\text{g}/\text{m}^2$  per one side, and 1.292  $\text{g}/\text{m}^2$  with respect to the sum of both sides.

The coating amount of each compound ( $\text{g}/\text{m}^2$ ) for the image forming layer per one side is as follows.

|    |                                            |               |
|----|--------------------------------------------|---------------|
| 5  | Silver salt of fatty acid                  | 2.85          |
|    | Organic polyhalogen compound-1             | 0.028         |
|    | Organic polyhalogen compound-2             | 0.094         |
|    | Silver iodide complex-forming agent        | 0.46          |
| 10 | SBR latex                                  | 5.20          |
|    | Reducing agent-1                           | 0.46          |
|    | Nucleator                                  | 0.035         |
|    | Hydrogen bonding compound-1                | 0.15          |
| 15 | Development accelerator-1                  | 0.005         |
|    | Development accelerator-2                  | 0.035         |
|    | Color-tone-adjusting agent-1               | 0.002         |
|    | Mercapto compound-1                        | 0.001         |
|    | Mercapto compound-2                        | 0.003         |
|    | Silver halide (on the basis of Ag content) | (see Table 6) |

<Measurement of Sensitivity>

20 Sensitivity at 390 nm that is the main emission peak of the aforesaid fluorescent intensifying screen A was measured as follows.

25 Each sample was subjected to exposure for  $1/10$  seconds by a 2856K° color temperature tungsten light source filtered through a interference filter produced by Corning Inc., which has a half band width of 10 nm and a central transparency wavelength at 390 nm, an infrared light cut filter, and a neutral step wedge. After exposure, the photothermographic material 30 was subjected to thermal development in a similar manner to the manner described above. After peeling off the image forming layer which was disposed on the opposite side to the exposed side, densities were measured to draw a photographic characteristic curve. From the photographic characteristic curve, the exposure value required to give a density of fog+0.5 was determined. On determination of the exposure value, the light emitted by the tungsten light source and 35 passed through the filter was measured using the radiophotometer DR-2550 (a corrected one) produced by EG&G Inc.

40 Evaluation similar to Example 1 and Example 2 was performed and the results are shown in Table 6 and Table 7. From the results, it is revealed that the higher is the aspect ratio and the thinner is the thickness of the emulsion, higher sharpness can be observed.

TABLE 6

| Sample No. | Silver Emulsion No. | Amount of Coated Silver Halide |                              |                                | Equivalent   |                        | Equivalent     |                         |                    |                                 |                                | Crossover Note |
|------------|---------------------|--------------------------------|------------------------------|--------------------------------|--------------|------------------------|----------------|-------------------------|--------------------|---------------------------------|--------------------------------|----------------|
|            |                     | Halide Emulsion                | One Side (g/m <sup>2</sup> ) | Both Sides (g/m <sup>2</sup> ) | Aspect Ratio | Circular Diameter (μm) | Thickness (μm) | Spherical Diameter (μm) | Parallel Light (%) | Haze before Thermal Development | Haze after Thermal Development | (%)            |
| 3-1        | E                   | 0.53                           | 1.06                         | 19.8                           | 1.707        | 0.085                  | 0.72           | 3.9                     | 72                 | 60                              | 25.3                           | Comparative    |
| 3-2        | E                   | 0.33                           | 0.66                         | 19.8                           | 1.707        | 0.085                  | 0.72           | 5.6                     | 66                 | 55                              | 27.8                           | Comparative    |
| 3-3        | E                   | 0.28                           | 0.56                         | 19.8                           | 1.707        | 0.085                  | 0.72           | 8.5                     | 60                 | 45                              | 34.3                           | Invention      |
| 3-4        | E                   | 0.19                           | 0.38                         | 19.8                           | 1.707        | 0.085                  | 0.72           | 10.3                    | 55                 | 40                              | 38.8                           | Invention      |
| 3-5        | E                   | 0.11                           | 0.22                         | 19.8                           | 1.707        | 0.085                  | 0.72           | 14.5                    | 43                 | 28                              | 45.5                           | Invention      |
| 3-6        | F                   | 0.19                           | 0.38                         | —                              | —            | —                      | 0.72           | 10.5                    | 67                 | 46                              | 36.5                           | Invention      |
| 3-7        | G                   | 0.19                           | 0.38                         | 3.1                            | 0.907        | 0.302                  | 0.72           | 9.8                     | 64                 | 45                              | 37.1                           | Invention      |
| 3-8        | H                   | 0.19                           | 0.38                         | 15.1                           | 1.551        | 0.103                  | 0.72           | 9.5                     | 60                 | 45                              | 37.8                           | Invention      |
| 3-9        | I                   | 0.19                           | 0.38                         | 1.6                            | 0.205        | 0.127                  | 0.15           | 7.3                     | 68                 | 48                              | 31.1                           | Invention      |

TABLE 7

| Sample No. | Silver Halide Emulsion No. | Fog  | Sensitivity (w · sec · m <sup>-2</sup> ) | Dmax | Gradation | Sharpness | Note        |
|------------|----------------------------|------|------------------------------------------|------|-----------|-----------|-------------|
| 3-1        | E                          | 0.35 | $3.20 \times 10^{-5}$                    | 2.65 | 3.83      | 0.64      | Comparative |
| 3-2        | E                          | 0.33 | $3.17 \times 10^{-5}$                    | 2.63 | 3.81      | 0.63      | Comparative |
| 3-3        | E                          | 0.31 | $3.18 \times 10^{-5}$                    | 2.63 | 3.82      | 0.75      | Invention   |
| 3-4        | E                          | 0.29 | $3.19 \times 10^{-5}$                    | 2.64 | 3.81      | 0.79      | Invention   |
| 3-5        | E                          | 0.28 | $3.20 \times 10^{-5}$                    | 2.59 | 3.75      | 0.83      | Invention   |
| 3-6        | F                          | 0.33 | $2.95 \times 10^{-5}$                    | 2.64 | 3.75      | 0.75      | Invention   |
| 3-7        | G                          | 0.32 | $3.05 \times 10^{-5}$                    | 2.63 | 3.77      | 0.72      | Invention   |
| 3-8        | H                          | 0.30 | $3.11 \times 10^{-5}$                    | 2.62 | 3.65      | 0.72      | Invention   |
| 3-9        | I                          | 0.29 | $2.25 \times 10^{-3}$                    | 2.61 | 3.55      | 0.69      | Invention   |

What is claimed is:

1. A photothermographic material comprising, on both sides of a support, an image forming layer comprising at least a photosensitive silver halide, a non-photosensitive organic silver salt, a reducing agent, and a binder, which is to be exposed with X-rays using a fluorescent intensifying screen, wherein

(1) a coating amount of the photosensitive silver halide per one side is from 0.01 g/m<sup>2</sup> to 0.45 g/m<sup>2</sup> in terms of silver amount, and

(2) when parallel light having the same wavelength as a main emission peak wavelength of the fluorescent intensifying screen is incident perpendicular to the surface of the photothermographic material, the parallel light component of transmitted light comprises 5% or more of the incident light.

2. The photothermographic material according to claim 1, wherein the parallel light component of the transmitted light comprises 6.5% or more of the incident light.

3. The photothermographic material according to claim 2, wherein the parallel light component of the transmitted light comprises 8% or more of the incident light.

4. The photothermographic material according to claim 1, further comprising a nucleator.

5. The photothermographic material according to claim 4, wherein the nucleator is selected from the group consisting of hydrazine derivative compounds represented by the following formula (V), vinyl compounds represented by the following formula (VI), and quaternary onium compounds represented by the following formula (P):



### Formula (V)

### Formula (VI)

### Formula (P)

wherein, in formula (V),  $A_0$  represents one selected from an aliphatic group, an aromatic group, a heterocyclic group, or a  $-G_0-D_0$  group, each of which may have a substituent;  $B_0$  represents a blocking group;  $A_1$  and  $A_2$  both represent a hydrogen atom, or one represents a hydrogen atom and the

5 other represents one of an acyl group, a sulfonyl group, and an oxalyl group;  $G_0$  represents one selected from a  $-\text{CO}-$  group, a  $-\text{COCO}-$  group, a  $-\text{CS}-$  group, a  $-\text{C}(\text{=NG}_1\text{D}_1)$  group, an  $-\text{SO}-$  group, an  $-\text{SO}_2-$  group, or a  $-\text{P}(\text{O})(\text{G}_1\text{D}_1)-$  group;  $G_1$  represents one selected from a mere bonding hand, an  $-\text{O}-$  group, an  $-\text{S}-$  group, or an  $-\text{N}(\text{D}_1)-$  group;  $D_1$  represents one selected from an aliphatic group, an aromatic group, a heterocyclic group, or a hydrogen atom; in the case where plural  $\text{D}_1$ 's exist in a molecule, they 10 may be the same or different; and  $D_0$  represents one selected from a hydrogen atom, an aliphatic group, an aromatic group, a heterocyclic group, an amino group, an alkoxy group, an aryloxy group, an alkylthio group, or an arylthio group;

in formula (VI), X represents an electron-attracting group, and W represents one selected from a hydrogen atom, an alkyl group, an alkenyl group, an alkynyl group, an aryl group, a heterocyclic group, a halogen atom, an acyl group, a thioacyl group, an oxalyl group, an oxyoxalyl group, a thioxalyl group, an oxamoyl group, an oxy-carbonyl group, a thiocarbonyl group, a carbamoyl group, a thiocarbamoyl group, a sulfonyl group, a sulfinyl group, an oxysulfinyl group, a thiosulfinyl group, a sulfamoyl group, an oxysulfamoyl group, a sulfuryl group, a nitro group, an imino group, a N-carboxylimino group, a N-sulfonylimino group, a dicyanoethylene group, an ammonium group, a sulfonium group, a phosphonium group, a pyrylium group, or an immonium group; R represents one selected from a halogen atom, a hydroxyl group, an alkoxy group, an aryloxy group, a heterocyclic oxy group, an alkenyloxy group, an acyloxy group, an alkoxycarbonyloxy group, an ammocarbonyloxy group, a mercapto group, an alkylthio group, an arylthio group, a heterocyclic thio group, an alkenylthio group, an acylthio group, an alkoxy carbonylthio group, an amine carbonylthio group, an organic or inorganic salt of hydroxy group or mercapto group, an amino group, an alkylamino group, a cyclic amino group, an acylamino group, an oxy carbonyl amino group, a heterocyclic group, a ureido group, or a sulfonamide group; and X and W, and X and R may bind to each other to form a cyclic structure;

in formula (P), Q represents a nitrogen atom or a phosphorus atom;  $R_1$ ,  $R_2$ ,  $R_3$ , and  $R_4$  each independently represent a hydrogen atom or a substituent, and  $X^-$  represents an anion; and  $R_1$  to  $R_4$  may bind to each other to form a cyclic structure.

6. The photothermographic material according to claim 5, wherein the vinyl compound is a cyclic olefine compound represented by the following formula (A), (B), or (C):



wherein, in formula (A),  $Z_1$  represents a nonmetallic atomic group capable to form a 5 to 7-membered cyclic structure with  $—Y_1—C(=CH—X_1)—C(=O)—$ ;  $Z_1$  may have a substituent, and  $Z_1$  itself may be an aromatic or a non-aromatic carbon ring, or  $Z_1$  may be a part of an aromatic or a non-aromatic heterocycle, and in this case, a 5 to 7-membered cyclic structure formed by  $Z_1$  with  $—Y_1—C(=CH—X_1)—C(=O)—$  forms a condensed cyclic structure; and  $X_1$  represents one selected from a hydroxy group (or a salt thereof), an alkoxy group, an aryloxy group, a heterocyclic oxy group, a mercapto group, an alkylthio group, an arylthio group, a hetero-

30 Formula (A)

5 in formula (B),  $Z_2$  represents a nonmetallic atomic group capable of forming a 5 to 7-membered cyclic structure with  $—Y_2—C(=CH—X_2)—C(Y_3)=N—$ ;  $Z_2$  may have a substituent, and  $Z_2$  itself may be an aromatic or a non-aromatic carbon ring, or  $Z_2$  may be a part of an aromatic or a non-aromatic heterocycle and in this case, a 5 to 7-membered cyclic structure formed by  $Z_2$  with  $—Y_2—C(=CH—X_2)—C(Y_3)=N—$  forms a condensed cyclic structure;  $X_2$  represents one selected from a hydroxy group (or a salt thereof), an alkoxy group, an aryloxy group, a heterocyclic oxy group, a mercapto group, an alkylthio group, an arylthio group, a heterocyclic thio group, an amino group, an alkylamino group, an arylamino group, a heterocyclic amino group, an acylamino group, a sulfonamide group, or a heterocyclic group; and  $Y_3$  represents a hydrogen atom or a substituent;

10 15 20 25 30 35 in formula (C),  $X_3$  represents one selected from an oxygen atom, a sulfur atom, or a nitrogen atom;  $Y_4$  represents the group represented by one selected from  $—C(=O)—$ ,  $—C(=S)—$ ,  $—SO—$ ,  $—SO_2—$ ,  $—C(=NR_3)—$ , or  $—(R_4)C=N—$ ;  $Z_3$  represents a nonmetallic atomic group capable to form a 5 to 7-membered ring containing  $X_3$  and  $Y_4$ ;  $R_1$ ,  $R_2$ ,  $R_3$ , and  $R_4$  each independently represent a hydrogen atom or a substituent; and  $R_1$  and  $R_2$  never bind to each other to form a cyclic structure.

7. The photothermographic material according to claim 4, wherein the nucleator is contained in an image forming layer or a layer adjacent to the image forming layer.

8. The photothermographic material according to claim 1, wherein the photosensitive silver halide is silver bromide or silver chloride.

\* \* \* \* \*